



US012233510B1

(12) **United States Patent**  
**Heaton et al.**

(10) **Patent No.:** **US 12,233,510 B1**  
(45) **Date of Patent:** **Feb. 25, 2025**

(54) **LEACHED POLYCRYSTALLINE DIAMOND ELEMENTS**

(71) Applicant: **US SYNTHETIC CORPORATION**, Orem, UT (US)

(72) Inventors: **Daren Nathaniel Heaton**, Spanish Fork, UT (US); **Jeremy Brett Lynn**, Nephi, UT (US); **Mark Pehrson Chapman**, Provo, UT (US); **Oakley D. Bond**, Nephi, UT (US)

(73) Assignee: **US Synthetic Corporation**, Orem, UT (US)

(\*) Notice: Subject to any disclaimer, the term of this patent is extended or adjusted under 35 U.S.C. 154(b) by 1003 days.

(21) Appl. No.: **16/841,339**

(22) Filed: **Apr. 6, 2020**

**Related U.S. Application Data**

(62) Division of application No. 14/879,907, filed on Oct. 9, 2015, now Pat. No. 10,610,999.

(60) Provisional application No. 62/096,315, filed on Dec. 23, 2014, provisional application No. 62/062,553, filed on Oct. 10, 2014.

(51) **Int. Cl.**

**B24D 3/06** (2006.01)

**C25F 1/00** (2006.01)

(52) **U.S. Cl.**

**CPC . B24D 3/06 (2013.01); C25F 1/00 (2013.01)**

(58) **Field of Classification Search**

**CPC ... C25F 1/00; B24D 3/06; E21B 10/00; E31B 10/46**

See application file for complete search history.

(56) **References Cited**

**U.S. PATENT DOCUMENTS**

4,268,276 A ‡ 5/1981 Bovenkerk ..... B01J 3/062  
175/42  
4,410,054 A ‡ 10/1983 Nagel ..... E21B 4/003  
175/10

(Continued)

**FOREIGN PATENT DOCUMENTS**

WO WO-2010135605 A2 \* 11/2010 ..... E21B 10/55

**OTHER PUBLICATIONS**

Percentage by Volume to Percentage by Weight Conversion Calculator for Diamond, Cobalt and Chromium Carbide. <http://www.handymath.com/cgi-bin/dnstyvolwt.cgi> (Mar. 14, 2019) (Year: 2019).\*

(Continued)

*Primary Examiner* — Pegah Parvini

(74) *Attorney, Agent, or Firm* — BKRP LLC

(57) **ABSTRACT**

A method of processing a polycrystalline diamond material includes exposing at least a portion of a polycrystalline diamond material to a processing solution, the polycrystalline diamond material including a metallic material disposed in interstitial spaces defined within the polycrystalline diamond material. The method includes exposing an electrode to the processing solution, applying a positive charge to the polycrystalline diamond material, and applying a negative charge to the electrode. An assembly for processing a polycrystalline diamond body includes a polycrystalline diamond body and an electrode that are in electrical communication with a volume of processing solution, and a power source configured to apply a positive charge to the polycrystalline diamond body and a negative charge to the electrode.

**23 Claims, 40 Drawing Sheets**



| (56)                  | References Cited          |                        |                    |                           |
|-----------------------|---------------------------|------------------------|--------------------|---------------------------|
| U.S. PATENT DOCUMENTS |                           |                        |                    |                           |
| 4,468,138 A ‡         | 8/1984 Nagel .....        | F16C 17/04<br>384/30   | 5,480,233 A ‡      | 1/1996 Cunningham .....   |
| 4,560,014 A ‡         | 12/1985 Geczy .....       | E21B 4/00<br>175/10    | 5,544,713 A ‡      | 8/1996 Dennis .....       |
| 4,738,322 A ‡         | 4/1988 Hall .....         | E21B 10/20<br>175/37   | 6,793,681 B1 ‡     | 9/2004 Pope .....         |
| 4,811,801 A ‡         | 3/1989 Salesky .....      | E21B 10/56<br>175/43   | 7,866,418 B2 ‡     | 1/2011 Bertagnolli .....  |
| 4,913,247 A ‡         | 4/1990 Jones .....        | E21B 10/54<br>175/43   | 8,297,382 B2 ‡     | 10/2012 Bertagnolli ..... |
| 5,016,718 A ‡         | 5/1991 Tandberg .....     | E21B 10/04<br>175/33   | 8,323,367 B1 ‡     | 12/2012 Bertagnolli ..... |
| 5,092,687 A ‡         | 3/1992 Hall .....         | E21B 4/003<br>384/30   | 2008/0115421 A1 *  | 5/2008 Sani .....         |
| 5,120,327 A ‡         | 6/1992 Dennis .....       | B22F 7/06<br>407/11    | 2011/0258936 A1 *  | 10/2011 DiGiovanni .....  |
| 5,135,061 A ‡         | 8/1992 Newton, Jr. .....  | B23B 27/148<br>175/42  | 2012/0261197 A1 *  | 10/2012 Miess .....       |
| 5,154,245 A ‡         | 10/1992 Waldenstrom ..... | E21B 10/5676<br>175/42 | 2013/0291447 A1 *  | 11/2013 Mazyar .....      |
| 5,364,192 A ‡         | 11/1994 Damm .....        | F16C 33/043<br>384/42  | 2017/0282334 A1 *  | 10/2017 Efird .....       |
| 5,368,398 A ‡         | 11/1994 Damm .....        | F16C 33/043<br>384/30  |                    | E21B 10/55                |
| 5,460,233 A ‡         | 10/1995 Meany .....       | E21B 10/5673<br>175/42 | OTHER PUBLICATIONS |                           |

Percentage by Volume to Percentage by Weight Conversion Calculator for Diamond, Cobalt and Tungsten Carbide. <http://www.handymath.com/cgi-bin/dnstyvolwt.cgi> (Nov. 21, 2017).\*

\* cited by examiner

‡ imported from a related application



FIG. 1



FIG. 2



FIG. 3



FIG. 4



FIG. 5A



FIG. 5B



FIG. 5C



FIG. 5D



FIG. 5E



FIG. 6A



FIG. 6B



FIG. 7



FIG. 8





FIG. 9C



FIG. 10A



FIG. 10B



FIG. 10C



FIG. 10D



FIG. 10E



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23A



FIG. 23B



FIG. 24



FIG. 25



FIG. 26



FIG. 27



FIG. 28



FIG. 29



FIG. 30



FIG. 31

FIG. 32



FIG. 33



FIG. 34



FIG. 35



FIG. 36



FIG. 37



FIG. 38



FIG. 39



FIG. 40A



FIG. 40B



FIG. 41A



FIG. 41B



FIG. 42



FIG. 43



FIG. 44



FIG. 45



FIG. 46



FIG. 47



FIG. 48



FIG.49A



FIG.49B



FIG.49C



FIG. 50A 



FIG. 50B 





FIG. 51A



FIG. 51B



FIG. 51C

## LEACHED POLYCRYSTALLINE DIAMOND ELEMENTS

### CROSS-REFERENCE TO RELATED APPLICATIONS

This application is a divisional of U.S. patent application Ser. No. 14/879,907, filed 9 Oct. 2015, which claims priority to U.S. Provisional Application Nos. 62/062,553, filed 10 Oct. 2014, and 62/096,315, filed on 23 Dec. 2014, each of which is hereby incorporated by reference in its entirety.

### BACKGROUND

Wear-resistant, superabrasive materials are traditionally utilized for a variety of mechanical applications. For example, polycrystalline diamond (“PCD”) materials are often used in drilling tools (e.g., cutting elements, gage trimmers, etc.), machining equipment, bearing apparatuses, wire-drawing machinery, and in other mechanical systems. Conventional superabrasive materials have found utility as superabrasive cutting elements in rotary drill bits, such as roller cone drill bits and fixed-cutter drill bits. A conventional cutting element may include a superabrasive layer or table, such as a PCD table. The cutting element may be brazed, press-fit, or otherwise secured into a preformed pocket, socket, or other receptacle formed in the rotary drill bit. In another configuration, the substrate may be brazed or otherwise joined to an attachment member such as a stud or a cylindrical backing. Generally, a rotary drill bit may include one or more PCD cutting elements affixed to a bit body of the rotary drill bit.

As mentioned above, conventional superabrasive materials have found utility as bearing elements, which may include bearing elements utilized in thrust bearing and radial bearing apparatuses. A conventional bearing element typically includes a superabrasive layer or table, such as a PCD table, bonded to a substrate. One or more bearing elements may be mounted to a bearing rotor or stator by press-fitting, brazing, or through other suitable methods of attachment. Typically, bearing elements mounted to a bearing rotor have superabrasive faces configured to contact corresponding superabrasive faces of bearing elements mounted to an adjacent bearing stator.

Cutting elements having a PCD table may be formed and bonded to a substrate using an ultra-high pressure, ultra-high temperature (“HPHT”) sintering process. Often, cutting elements having a PCD table are fabricated by placing a cemented carbide substrate, such as a cobalt-cemented tungsten carbide substrate, into a container or cartridge with a volume of diamond particles positioned on a surface of the cemented carbide substrate. A number of such cartridges may be loaded into a HPHT press. The substrates and diamond particle volumes may then be processed under HPHT conditions in the presence of a catalyst material that causes the diamond particles to bond to one another to form a diamond table having a matrix of bonded diamond crystals. The catalyst material is often a metal-solvent catalyst, such as cobalt, nickel, and/or iron, that facilitates intergrowth and bonding of the diamond crystals.

In one conventional approach, a constituent of the cemented-carbide substrate, such as cobalt from a cobalt-cemented tungsten carbide substrate, liquefies and sweeps from a region adjacent to the volume of diamond particles into interstitial regions between the diamond particles during the HPHT process. The cobalt may act as a catalyst to facilitate the formation of bonded diamond crystals. A

metal-solvent catalyst may also be mixed with a volume of diamond particles prior to subjecting the diamond particles and substrate to the HPHT process.

The metal-solvent catalyst may dissolve carbon from the diamond particles and portions of the diamond particles that graphitize due to the high temperatures used in the HPHT process. The solubility of the stable diamond phase in the metal-solvent catalyst may be lower than that of the metastable graphite phase under HPHT conditions. As a result of the solubility difference, the graphite tends to dissolve into the metal-solvent catalyst and the diamond tends to deposit onto existing diamond particles to form diamond-to-diamond bonds. Accordingly, diamond grains may become mutually bonded to form a matrix of polycrystalline diamond, with interstitial regions defined between the bonded diamond grains being occupied by the metal-solvent catalyst. In addition to dissolving carbon and graphite, the metal-solvent catalyst may also carry tungsten, tungsten carbide, and/or other materials from the substrate into the PCD layer of the cutting element.

The presence of the metal-solvent catalyst and/or other materials in the diamond table may reduce the thermal stability of the diamond table at elevated temperatures. For example, the difference in thermal expansion coefficient between the diamond grains and the solvent catalyst is believed to lead to chipping or cracking in the PCD table of a cutting element during drilling or cutting operations. The chipping or cracking in the PCD table may degrade the mechanical properties of the cutting element or lead to failure of the cutting element. Additionally, at high temperatures, diamond grains may undergo a chemical breakdown or back-conversion with the metal-solvent catalyst. Further, portions of diamond grains may transform to carbon monoxide, carbon dioxide, graphite, or combinations thereof, thereby degrading the mechanical properties of the PCD material.

Accordingly, it is desirable to remove metallic materials, such as metal-solvent catalysts, from a PCD material in situations where the PCD material may be exposed to high temperatures. Chemical leaching is often used to dissolve and remove various materials from the PCD layer. For example, chemical leaching may be used to remove metal-solvent catalysts, such as cobalt, from regions of a PCD layer that may experience elevated temperatures during drilling, such as regions adjacent to the working surfaces of the PCD layer.

During conventional leaching of a PCD table, exposed surface regions of the PCD table are immersed in a leaching solution until interstitial components, such as a metal-solvent catalyst, are removed to a desired depth from the exposed surface regions. The process of chemical leaching often involves the use of highly concentrated and/or corrosive solutions, such as aqua regia and mixtures including hydrofluoric acid (HF), to dissolve and remove metal-solvent catalysts from polycrystalline diamond materials. Moreover, in addition to dissolving metal-solvent catalysts from a PCD material, leaching solutions may be difficult to control, may take a long time, and may dissolve any accessible portions of a substrate to which the PCD material is attached. Therefore, improved methods for leaching PCD materials that reduce or mitigate difficulties with conventional leaching are desired.

### SUMMARY

The instant disclosure is directed to methods and assemblies for processing superabrasive elements. In some

examples, the method may comprise exposing at least a portion of a polycrystalline diamond material to a processing solution, exposing an electrode to the processing solution, applying a positive charge to the polycrystalline diamond material, and applying a negative charge to the electrode. The polycrystalline diamond material may comprise a metallic material (e.g., cobalt, nickel, iron, and/or tungsten) disposed in interstitial spaces defined within the polycrystalline diamond material.

The processing solution may comprise a suitable solution that leaches the metallic material from interstitial spaces within at least a volume of the polycrystalline diamond material. According to at least one embodiment, the rate at which the processing solution leaches the metallic material from the interstitial spaces within at least the volume of the polycrystalline diamond material is increased in the presence of an electrical current between the polycrystalline diamond material and the electrode. According to various embodiments, the electrode may be disposed near at least the portion of the polycrystalline diamond material. The electrode may be disposed such that the electrode does not directly contact the polycrystalline diamond material.

The processing solution may at least partially oxidize the metallic material when the polycrystalline diamond material is processed. According to at least one embodiment, the processing solution may comprise an aqueous solution. According to some embodiments, the processing solution may comprise a buffered or a non-buffered electrolyte solution. In various embodiments, the processing solution may comprise at least one of acetic acid, ammonium chloride, arsenic acid, ascorbic acid, citric acid, formic acid, hydrobromic acid, hydrofluoric acid, hydroiodic acid, lactic acid, malic acid, nitric acid, oxalic acid, phosphoric acid, propionic acid, pyruvic acid, succinic acid, tartaric acid, and/or any suitable carboxylic acid (e.g., monocarboxylic acid, polycarboxylic acid, etc.); the processing solution may additionally or alternatively comprise at least one of an ion, a salt, and an ester of at least one of the foregoing. The electrode may comprise at least one of copper, tungsten carbide, cobalt, zinc, iron, platinum, palladium, niobium, graphite, graphene, nichrome, gold, and silver. According to various embodiments, a masking layer may be disposed over at least a portion of the polycrystalline diamond material.

In some embodiments, a cation of the metallic material may be present in the processing solution following application of the positive charge to the polycrystalline diamond material and application of the negative charge to the electrode. The cation of the metallic material may be reduced and electrodeposited on the electrode. The processing solution may comprise a first processing solution and the method may further comprise exposing at least the portion of the polycrystalline diamond material to a second processing solution (e.g., a more acidic solution than the first processing solution). At least a portion of the polycrystalline diamond material may be exposed to the second processing solution following exposure of at least the portion of the polycrystalline diamond material to the first processing solution. Additionally, at least the portion of the polycrystalline diamond material may be exposed to the second processing solution prior to exposure of at least the portion of the polycrystalline diamond material to the first processing solution. In some embodiments, an electrode for applying the positive charge abuts the polycrystalline diamond material.

According to some embodiments, a method of processing a superabrasive element may include providing a superabrasive element, exposing at least a portion of the superabrasive

element to a processing solution, exposing an electrode to the processing solution, applying a first charge to the polycrystalline diamond table, and applying a second charge to the electrode. The polycrystalline diamond element may comprise a substrate and a polycrystalline diamond table bonded to the substrate, the polycrystalline diamond table comprising a metallic material disposed in interstitial spaces defined within the polycrystalline diamond table. According to various embodiments, the first charge may be applied to the polycrystalline diamond table via the substrate. In some examples, a masking layer may be disposed over at least a portion of the polycrystalline diamond table.

According to at least one embodiment, an assembly for processing a polycrystalline diamond body may include a volume of processing solution, a polycrystalline diamond body, an electrode, and a power source configured to apply a positive charge to the polycrystalline diamond body and a negative charge to the electrode. The polycrystalline diamond body and the electrode may both be in electrical communication with the processing solution. The polycrystalline diamond body may comprise a metallic material disposed in interstitial spaces defined within the polycrystalline diamond body. At least a portion of the polycrystalline diamond body and the electrode may be exposed to the volume of processing solution. The assembly may additionally include a first wire electrically connecting the power source to the polycrystalline diamond body and a second wire electrically connecting the power source to the electrode. The assembly may further include a substrate bonded to the polycrystalline diamond body, the first wire being electrically connected to the substrate by an electrode disposed on a surface portion of the substrate.

In at least one embodiment, a leached polycrystalline diamond element is disclosed. The leached polycrystalline diamond element may be fabricated according to a method. The method includes exposing an electrode and at least a portion of a polycrystalline diamond material to a processing solution. The polycrystalline diamond material includes a plurality of diamond grains defining a plurality of interstitial regions, with at least a portion of the plurality of interstitial regions including a metallic material and at least one tungsten-containing material disposed therein. The method further includes, while the electrode and the at least portion of the polycrystalline diamond material are exposed to the processing solution, applying an electrical potential between the electrode and the polycrystalline diamond material to cause electrochemical and preferential leaching of at least a portion of the metallic material from the polycrystalline diamond material over the at least one tungsten-containing material.

In an embodiment, a polycrystalline diamond compact is disclosed. The polycrystalline diamond compact includes a substrate and a polycrystalline diamond table bonded to the substrate. The polycrystalline diamond table includes a plurality of bonded diamond grains defining a plurality of interstitial regions. The polycrystalline diamond table defines an upper surface spaced from an interfacial surface bonded to the substrate. The polycrystalline diamond table further includes an unleached volume extending inwardly from the interfacial surface, with at least a portion of the plurality of interstitial regions of the unleached volume including a metallic material and at least one tungsten-containing material disposed therein. The polycrystalline diamond table includes a leached volume extending between the unleached volume and the upper surface. The metallic material may be present in the leached volume in a first concentration and the at least one tungsten-containing mate-

rial may be present in the leached volume in a second concentration of greater than 0 to about 4 weight %.

Features from any of the disclosed embodiments may be used in combination with one another in accordance with the general principles described herein. These and other embodiments, features, and advantages will be more fully understood upon reading the following detailed description in conjunction with the accompanying drawings and claims.

#### BRIEF DESCRIPTION OF THE DRAWINGS

The accompanying drawings illustrate a number of embodiments and are a part of the specification. Together with the following description, these drawings demonstrate and explain various principles of the instant disclosure.

FIG. 1 is an isometric view of a superabrasive element according to at least one embodiment.

FIG. 2 is a cross-sectional side view of the superabrasive element of FIG. 1.

FIG. 3 is an isometric view of a superabrasive element according to at least one embodiment.

FIG. 4 is a cross-sectional side view of the superabrasive element of FIG. 3.

FIG. 5A is a cross-sectional side view of a portion of a superabrasive table according to at least one embodiment.

FIGS. 5B-5E are a cross-sectional side view of a portion of a PCD table according to at least one embodiment after a conventional non-electrochemical leaching of the PCD table and electrochemically leaching of the PCD table.

FIG. 6A is a magnified cross-sectional side view of a portion of a superabrasive table according to at least one embodiment.

FIG. 6B is a magnified cross-sectional side view of a portion of a superabrasive table according to at least one embodiment.

FIG. 7 is an isometric view of a superabrasive element disposed near an electrode according to at least one embodiment.

FIG. 8 is a cross-sectional side view of the superabrasive element disposed near the electrode of FIG. 7.

FIG. 9A is a cross-sectional side view of a superabrasive element disposed near an electrode and positioned within a protective leaching cup according to at least one embodiment.

FIG. 9B is a cross-sectional side view of a superabrasive element disposed adjacent to an electrode and positioned within a protective leaching cup according to at least one embodiment.

FIG. 9C is a cross-sectional side view of a leaching assembly according to at least one embodiment.

FIG. 10A is a cross-sectional side view of a leaching assembly according to at least one embodiment.

FIG. 10B is a cross-sectional side view of a leached superabrasive element according to at least one embodiment.

FIG. 10C is a cross-sectional side view of a leached superabrasive element according to at least one embodiment.

FIG. 10D is a cross-sectional side view of a leaching assembly according to at least one embodiment.

FIG. 10E is a cross-sectional side view of a leaching assembly according to at least one embodiment.

FIG. 11 is an isometric view of a superabrasive element and an electrode according to at least one embodiment.

FIG. 12 is a cross-sectional side view of the superabrasive element and the electrode of FIG. 11.

FIG. 13 is an isometric view of a superabrasive element and an electrode according to at least one embodiment.

FIG. 14 is a cross-sectional side view of the superabrasive element and the electrode of FIG. 13.

FIGS. 15-21 are cross-sectional side views of superabrasive elements and electrodes according to various embodiments.

FIG. 22 is a cross-sectional side view of a superabrasive element and electrodes according to at least one embodiment.

FIG. 23A is an isometric view of a superabrasive element coated with a masking layer and disposed near an electrode according to at least one embodiment.

FIG. 23B is a cross-sectional side view of the superabrasive element coated with the masking layer and disposed near the electrode of FIG. 23A.

FIGS. 24-27 are cross-sectional side views of superabrasive elements each coated with a masking layer and disposed near an electrode according to various embodiments.

FIG. 28 is a cross-sectional side view of a superabrasive element coated with a masking layer, positioned within a protective leaching cup, and disposed near an electrode according to at least one embodiment.

FIG. 29 is an isometric view of a leaching assembly according to at least one embodiment.

FIGS. 30-41B are cross-sectional side views of superabrasive elements according to various embodiments.

FIG. 42 is an isometric view of a drill bit according to at least one embodiment.

FIG. 43 is a partial cut-away isometric view of a thrust bearing apparatus according to at least one embodiment.

FIG. 44 is a partial cut-away isometric view of a radial bearing apparatus according to at least one embodiment.

FIG. 45 is a partial cut-away isometric view of a subterranean drilling system according to at least one embodiment.

FIG. 46 is a flow diagram of a method of processing a polycrystalline diamond element according to at least one embodiment.

FIG. 47 is a flow diagram of a method of processing a polycrystalline diamond element according to at least one embodiment.

FIG. 48 is a graph of diamond volume removed (DVR) versus number of passes in an abrasion resistance test for Examples 4 and 5 performed in a wet vertical turret lathe (VTL) test.

FIGS. 49A-49C are photomicrographs of a PCD table of Example 4 at 75x.

FIGS. 50A-50C are photomicrographs of a PCD table of Example 5 at 75x.

FIGS. 51A-51B are plots of the tungsten and cobalt content, respectively, of the leaching solutions of Examples 6 and 7.

FIG. 51C is a plot diagram of the cobalt to tungsten ratios of the leaching solutions of Examples 8 and 9.

Throughout the drawings, identical reference characters and descriptions indicate similar, but not necessarily identical, elements. While the embodiments described herein are susceptible to various modifications and alternative forms, specific embodiments have been shown by way of example in the drawings and will be described in detail herein. However, the embodiments described herein are not intended to be limited to the particular forms disclosed. Rather, the instant disclosure covers all modifications, equivalents, and alternatives falling within the scope of the appended claims.

#### DETAILED DESCRIPTION

The instant disclosure is directed to leached superabrasive elements and leaching systems, methods, and assemblies for

processing superabrasive elements. Such superabrasive elements may be used as cutting elements for use in a variety of applications, such as drilling tools, machining equipment, cutting tools, and other apparatuses, without limitation. Superabrasive elements, as disclosed herein, may also be used as bearing elements in a variety of bearing applications, such as thrust bearings, radial bearings, and other bearing apparatuses, without limitation.

The terms "superabrasive" and "superhard," as used herein, may refer to any material having a hardness that is at least equal to a hardness of tungsten carbide. For example, a superabrasive article may represent an article of manufacture, at least a portion of which may exhibit a hardness that is equal to or greater than the hardness of tungsten carbide. Additionally, the term "solvent," as used herein, may refer to a single solvent compound, a mixture of two or more solvent compounds, and/or a mixture of one or more solvent compounds and one or more dissolved compounds. The term "molar concentration," as used herein, may refer to a concentration in units of mol/L at a temperature of approximately 25° C. For example, a solution comprising solute A at a molar concentration of 1 M may comprise 1 mol of solute A per liter of solution. Moreover, the term "cutting," as used herein, may refer to machining processes, drilling processes, boring processes, and/or any other material removal process utilizing a cutting element and/or other cutting apparatus, without limitation.

FIGS. 1 and 2 illustrate a superabrasive element 10 according to at least one embodiment. As illustrated in FIGS. 1 and 2, superabrasive element 10 may comprise a superabrasive table 14 affixed to or formed upon a substrate 12. Superabrasive table 14 may be affixed to substrate 12 at interface 26, which may be a planar or non-planar interface. Superabrasive element 10 may comprise a rear surface 18, a superabrasive face 20, and an element side surface 15. In some embodiments, element side surface 15 may include a substrate side surface 16 formed by substrate 12 and a superabrasive side surface 22 formed by superabrasive table 14. Rear surface 18 may be formed by substrate 12.

Superabrasive element 10 may also comprise a chamfer 24 (i.e., sloped or angled) formed by superabrasive table 14. Chamfer 24 may comprise an angular and/or rounded edge formed at the intersection of superabrasive side surface 22 and superabrasive face 20. Any other suitable surface shape may also be formed at the intersection of superabrasive side surface 22 and superabrasive face 20, including, without limitation, an arcuate surface (e.g., a radius, an ovoid shape, or any other rounded shape), a sharp edge, multiple chamfers/radii, a honed edge, and/or combinations of the foregoing. At least one edge may be formed at the intersection of chamfer 24 and superabrasive face 20 and/or at the intersection of chamfer 24 and superabrasive side surface 22. For example, cutting element 10 may comprise one or more cutting edges, such as an edge 27 and/or an edge 28. Edge 27 and/or edge 28 may be formed adjacent to chamfer 24 and may be configured to be exposed to and/or in contact with a mining formation during drilling.

In some embodiments, superabrasive element 10 may be utilized as a cutting element for a drill bit, in which chamfer 24 acts as a cutting edge. The phrase "cutting edge" may refer, without limitation, to a portion of a cutting element that is configured to be exposed to and/or in contact with a subterranean formation during drilling. In at least one embodiment, superabrasive element 10 may be utilized as a bearing element (e.g., with superabrasive face 20 acting as a bearing surface) configured to contact oppositely facing bearing elements.

According to various embodiments, superabrasive element 10 may also comprise a substrate chamfer 19 formed by substrate 12. For example, a chamfer comprising an angular and/or rounded edge may be formed by substrate 12 at the intersection of substrate side surface 16 and rear surface 18. Any other suitable surface shape may also be formed at the intersection of substrate side surface 16 and rear surface 18, including, without limitation, an arcuate surface (e.g., a radius, an ovoid shape, or any other rounded shape), a sharp edge, multiple chamfers/radii, a honed edge, and/or combinations of the foregoing.

Superabrasive element 10 may comprise any suitable size, shape, and/or geometry, without limitation. According to at least one embodiment, at least a portion of superabrasive element 10 may have a substantially cylindrical shape. For example, superabrasive element 10 may comprise a substantially cylindrical outer surface surrounding a central axis 29 of superabrasive element 10, as illustrated in FIGS. 1 and 2. Substrate side surface 16 and superabrasive side surface 22 may, for example, be substantially cylindrical and may have any suitable diameters relative to central axis 29, without limitation. According to various embodiments, substrate side surface 16 and superabrasive side surface 22 may have substantially the same outer diameter relative to central axis 29. Superabrasive element 10 may also comprise any other suitable shape, including, for example, an oval, ellipsoid, triangular, pyramidal, square, cubic, rectangular, and/or composite shape, and/or a combination of the foregoing, without limitation.

According to various embodiments, superabrasive element 10 may also comprise a rear chamfer 19. For example, a rear chamfer 19 comprising an angular and/or rounded edge may be formed by superabrasive element 10 at the intersection of substrate side surface 16 and rear surface 18. Any other suitable surface shape may also be formed at the intersection of substrate side surface 16 and rear surface 18, including, without limitation, an arcuate surface (e.g., a radius, an ovoid shape, or any other rounded shape), a sharp edge, multiple chamfers/radii, a honed edge, and/or combinations of the foregoing.

Substrate 12 may comprise any suitable material on which superabrasive table 14 may be formed. In at least one embodiment, substrate 12 may comprise a cemented carbide material, such as a cobalt-cemented tungsten carbide material and/or any other suitable material. In some embodiments, substrate 12 may include a suitable metal-solvent catalyst material, such as, for example, cobalt, nickel, iron, and/or alloys thereof. Substrate 12 may also include any suitable material including, without limitation, cemented carbides such as titanium carbide, niobium carbide, tantalum carbide, vanadium carbide, chromium carbide, and/or combinations of any of the preceding carbides cemented with iron, nickel, cobalt, and/or alloys thereof. Superabrasive table 14 may be formed of any suitable superabrasive and/or superhard material or combination of materials, including, for example PCD. According to additional embodiments, superabrasive table 14 may comprise cubic boron nitride, silicon carbide, polycrystalline diamond, and/or mixtures or composites including one or more of the foregoing materials, without limitation.

Superabrasive table 14 may be formed using any suitable technique. According to some embodiments, superabrasive table 14 may comprise a PCD table fabricated by subjecting a plurality of diamond particles to an HPHT sintering process in the presence of a metal-solvent catalyst (e.g., cobalt, nickel, iron, or alloys thereof) to facilitate intergrowth between the diamond particles and form a PCD body

comprised of bonded diamond grains that exhibit diamond-to-diamond bonding therebetween. For example, the metal-solvent catalyst may be mixed with the diamond particles, infiltrated from a metal-solvent catalyst foil or powder adjacent to the diamond particles, infiltrated from a metal-solvent catalyst present in a cemented carbide substrate, or combinations of the foregoing. The bonded diamond grains (e.g., sp<sub>3</sub>-bonded diamond grains), so-formed by HPHT sintering the diamond particles, define interstitial regions with the metal-solvent catalyst disposed within the interstitial regions of the as-sintered PCD body. The diamond particles may exhibit a selected diamond particle size distribution. Polycrystalline diamond elements, such as those disclosed in U.S. Pat. Nos. 7,866,418 and 8,297,382, the disclosure of each of which is incorporated herein, in its entirety, by this reference, may have magnetic properties in at least some regions as disclosed therein and leached regions in other regions as disclosed herein.

Following sintering, various materials, such as a metal-solvent catalyst, remaining in interstitial regions within the as-sintered PCD body may reduce the thermal stability of superabrasive table 14 at elevated temperatures. In some examples, differences in thermal expansion coefficients between diamond grains in the as-sintered PCD body and a metal-solvent catalyst in interstitial regions between the diamond grains may weaken portions of superabrasive table 14 that are exposed to elevated temperatures, such as temperatures developed during drilling and/or cutting operations. The weakened portions of superabrasive table 14 may be excessively worn and/or damaged during the drilling and/or cutting operations.

Removing the metal-solvent catalyst and/or other materials from the as-sintered PCD body may improve the heat resistance and/or thermal stability of superabrasive table 14, particularly in situations where the PCD material may be exposed to elevated temperatures. A metal-solvent catalyst and/or other materials may be removed from the as-sintered PCD body using any suitable technique, including, for example, electrochemical leaching. In at least one embodiment, a metal-solvent catalyst, such as cobalt, may be removed from regions of the as-sintered PCD body, such as regions adjacent to the working surfaces of superabrasive table 14. Removing a metal-solvent catalyst from the as-sintered PCD body may reduce damage to the PCD material of superabrasive table 14 caused by expansion of the metal-solvent catalyst.

At least a portion of a metal-solvent catalyst, such as cobalt, as well as other materials, may be removed from at least a portion of the as-sintered PCD body using any suitable technique, without limitation. For example, electrochemical, chemical and/or gaseous leaching may be used to remove a metal-solvent catalyst from the as-sintered PCD body up to a desired depth from a surface thereof. The as-sintered PCD body may be electrochemically leached by immersion in an acid or acid solution, such as a solution including acetic acid, ammonium chloride, arsenic acid, ascorbic acid, citric acid, formic acid, hydrobromic acid, hydrofluoric acid, hydroiodic acid, lactic acid, malic acid, nitric acid, oxalic acid, phosphoric acid, propionic acid, pyruvic acid, succinic acid, tartaric acid, and/or any suitable carboxylic acid (e.g., monocarboxylic acid, polycarboxylic acid, etc.), in the presence of an electrode, such as copper, tungsten carbide, cobalt, zinc, iron, platinum, palladium, niobium, graphite, graphene, nichrome, gold, and/or silver electrode, wherein a charge is applied to the as-sintered PCD body and an opposite charge is applied to the electrode or subjected to another suitable process to remove at least a

portion of the metal-solvent catalyst from the interstitial regions of the PCD body and form superabrasive table 14 comprising a PCD table. For example, the as-sintered PCD body may be immersed in an acid solution in the presence of an electrode, a positive charge may be applied to the as-sintered PCD body and a negative charge may be applied to the electrode for a selected amount of time. For example, a PCD body may be positively charged and an electrode may be negatively charged for more than 4 hours, more than 10 hours, between 24 hours to 48 hours, about 2 to about 7 days (e.g., about 3, 5, or 7 days), for a few weeks (e.g., about 4 weeks), or for 1-2 months, depending on the process employed.

Even after leaching, a residual, detectable amount of the metal-solvent catalyst may be present in the at least partially leached superabrasive table 14. It is noted that when the metal-solvent catalyst is infiltrated into the diamond particles from a cemented tungsten carbide substrate including tungsten carbide particles cemented with a metal-solvent catalyst (e.g., cobalt, nickel, iron, or alloys thereof), the infiltrated metal-solvent catalyst may carry tungsten and/or tungsten carbide therewith and the as-sintered PCD body may include such tungsten and/or tungsten carbide therein disposed interstitially between the bonded diamond grains. The tungsten and/or tungsten carbide may be at least partially removed by the selected leaching process or may be relatively unaffected by the selected leaching process. For example, in some embodiments, the electrochemical leaching processes disclosed herein may preferentially remove metal-solvent catalyst or other metallic material (e.g., cobalt or other Group VIII metal) over other materials such as tungsten or carbide material (e.g., tungsten carbide).

In some embodiments, only selected portions of the as-sintered PCD body may be leached, leaving remaining portions of resulting superabrasive table 14 unleached. For example, some portions of one or more surfaces of the as-sintered PCD body may be masked or otherwise protected from exposure to a processing solution and/or gas mixture while other portions of one or more surfaces of the as-sintered PCD body may be exposed to the processing solution and/or gas mixture. Other suitable techniques may be used for removing a metal-solvent catalyst and/or other materials from the as-sintered PCD body or may be used to accelerate an electrochemical leaching process, as will be described in greater detail below. For example, exposing the as-sintered PCD body to heat, pressure, microwave radiation, and/or ultrasound may be employed to leach or to accelerate an electrochemical leaching process, without limitation. Following leaching, superabrasive table 14 may comprise a volume of PCD material that is at least partially free or substantially free of a metal-solvent catalyst.

The plurality of diamond particles used to form superabrasive table 14 comprising the PCD material may exhibit one or more selected sizes. The one or more selected sizes may be determined, for example, by passing the diamond particles through one or more sizing sieves or by any other method. In an embodiment, the plurality of diamond particles may include a relatively larger size and at least one relatively smaller size. As used herein, the phrases "relatively larger" and "relatively smaller" refer to particle sizes determined by any suitable method, which differ by at least a factor of two (e.g., 40  $\mu\text{m}$  and 20  $\mu\text{m}$ ). More particularly, in various embodiments, the plurality of diamond particles may include a portion exhibiting a relatively larger size (e.g., 100  $\mu\text{m}$ , 90  $\mu\text{m}$ , 80  $\mu\text{m}$ , 70  $\mu\text{m}$ , 60  $\mu\text{m}$ , 50  $\mu\text{m}$ , 40  $\mu\text{m}$ , 30  $\mu\text{m}$ , 20  $\mu\text{m}$ , 15  $\mu\text{m}$ , 12  $\mu\text{m}$ , 10  $\mu\text{m}$ , 8  $\mu\text{m}$ ) and another portion exhibiting at least one relatively smaller size (e.g., 30  $\mu\text{m}$ , 20

## 11

μm, 15 μm, 12 μm, 10 μm, 8 μm, 4 μm, 2 μm, 1 μm, 0.5 μm, less than 0.5 μm, 0.1 μm, less than 0.1 μm). In another embodiment, the plurality of diamond particles may include a portion exhibiting a relatively larger size between about 40 μm and about 15 μm and another portion exhibiting a relatively smaller size between about 12 μm and 2 μm. In some embodiments, the plurality of diamond particles may also include three or more different sizes (e.g., one relatively larger size and two or more relatively smaller sizes), without limitation. Different sizes of diamond particle may be disposed in different locations within a polycrystalline diamond volume, without limitation. According to at least one embodiment, disposing different sizes of diamond particles in different locations may facilitate control of a leach depth, as will be described in greater detail below. It should be understood that reference to “particle sizes” herein refers to the average particle size of a plurality of particles, allowing for some slight deviation in individual particle sizes of some of the plurality of particles.

FIGS. 3 and 4 illustrate a superabrasive element 110 according to various embodiments. Superabrasive element 110 may comprise a superabrasive table 114 that is not attached to a substrate. As shown in FIGS. 3 and 4, superabrasive element 110 may include a rear surface 118, a superabrasive face 120, and an element side surface 122 formed by superabrasive table 114. Superabrasive element 110 may also comprise a chamfer 124 (i.e., sloped or angled) and/or any other suitable surface shape at the intersection of element side surface 122 and superabrasive face 120, including, without limitation, an arcuate surface (e.g., a radius, an ovoid shape, or any other rounded shape), a sharp edge, multiple chamfers/radii, a honed edge, and/or combinations of the foregoing. At least one edge, such as an edge 127 and/or an edge 128, may be formed at the intersection of chamfer 124 and each of superabrasive face 120 and element side surface 122, respectively. Element side surface 122 of superabrasive element 110 may radially surround a central axis 129 of superabrasive element 110.

According to various embodiments, superabrasive element 110 may also comprise a rear chamfer 119. For example, a rear chamfer 119 comprising an angular and/or rounded edge may be formed by superabrasive element 110 at the intersection of element side surface 122 and rear surface 118. Any other suitable surface shape may also be formed at the intersection of element side surface 122 and rear surface 118, including, without limitation, an arcuate surface (e.g., a radius, an ovoid shape, or any other rounded shape), a sharp edge, multiple chamfers/radii, a honed edge, and/or combinations of the foregoing.

Superabrasive element 110 may be formed using any suitable technique, including, for example, HPHT sintering, as described above. In some examples, superabrasive element 110 may be created by first forming a superabrasive element 10 that includes a substrate 12 and a superabrasive table 14, as detailed above in reference to FIGS. 1 and 2. Once superabrasive element 10 has been produced, superabrasive table 14 may be separated from substrate 12 to form superabrasive element 110. For example, prior to or following leaching, superabrasive table 14 may be separated from substrate 12 using any suitable process, including a lapping process, a grinding process, a wire-electrical-discharge machining (“wire EDM”) process, or any other suitable material-removal process, without limitation.

According to some embodiments, superabrasive element 110 may be processed and utilized either with or without an attached substrate. For example, following leaching, superabrasive element 110 may be secured directly to a cutting

## 12

tool, such as a drill bit, or to a bearing component, such as a rotor or stator. In various embodiments, following processing, superabrasive element 110 may be attached to a substrate. For example, rear surface 118 of superabrasive element 110 may be brazed, welded, soldered, threadedly coupled, and/or otherwise adhered and/or fastened to a substrate, such as tungsten carbide substrate or any other suitable substrate, without limitation. Polycrystalline diamond elements having pre-sintered polycrystalline diamond bodies including an infiltrant, such as those disclosed in U.S. Pat. No. 8,323,367, the disclosure of which is incorporated herein, in its entirety, by this reference, may be leached a second time according to the processes disclosed herein after reattachment of the pre-sintered polycrystalline diamond bodies.

FIG. 5A is a cross-sectional side view of a portion of a superabrasive table 214, such as the superabrasive tables 14 and 114 illustrated in FIGS. 1-4. Superabrasive table 14 may comprise a composite material, such as a PCD material. A PCD material may include a matrix of bonded diamond grains and interstitial regions defined between the bonded diamond grains. Such interstitial regions may be at least partially filled with various materials. In some embodiments, a metal-solvent catalyst may be disposed in interstitial regions in superabrasive table 14. Tungsten and/or tungsten carbide may also be present in the interstitial regions.

According to various embodiments, materials may be deposited in interstitial regions during processing of superabrasive table 14. For example, material components of substrate 12 may migrate into a mass of diamond particles used to form a superabrasive table 14 during HPHT sintering. As the mass of diamond particles is sintered, a metal-solvent catalyst may melt and flow from substrate 12 into the mass of diamond particles. As the metal-solvent flows into superabrasive table 14, it may dissolve and/or carry additional materials, such as tungsten and/or tungsten carbide, from substrate 12 into the mass of diamond particles. As the metal-solvent catalyst flows into the mass of diamond particles, the metal-solvent catalyst, and any dissolved and/or undissolved materials, may at least partially fill spaces between the diamond particles. The metal-solvent catalyst may facilitate bonding of adjacent diamond particles to form a PCD layer. Following sintering, any materials, such as, for example, the metal-solvent catalyst, tungsten, and/or tungsten carbide, may remain in interstitial regions within superabrasive table 14.

To improve the performance and heat resistance of a surface of superabrasive table 14, at least a portion of a metal-solvent catalyst, such as cobalt, may be removed from at least a portion of superabrasive table 14. Optionally, tungsten and/or tungsten carbide may be removed from at least a portion of superabrasive table 14. A metal-solvent catalyst, as well as other materials, may be removed from superabrasive table 14 using any suitable technique, without limitation.

For example, electrochemical leaching may be used to remove a metal-solvent catalyst from superabrasive table 214 up to a depth D from a surface of superabrasive table 214, as illustrated in FIG. 5A. As shown in FIG. 5A, depth D may be measured relative to an external surface of superabrasive table 214, such as superabrasive face 220, superabrasive side surface 222, and/or chamfer 224. In some examples, a metal-solvent catalyst may be removed from superabrasive table 214 up to a depth D of approximately 2500 μm. In additional examples, a metal-solvent catalyst may be removed from superabrasive table 214 up to a depth D of between approximately 100 and 1000 μm, such as

13

about 100  $\mu\text{m}$  to about 250  $\mu\text{m}$ , about 250  $\mu\text{m}$  to about 500  $\mu\text{m}$ , about 500  $\mu\text{m}$  to about 750  $\mu\text{m}$ , about 750  $\mu\text{m}$  to about 1000  $\mu\text{m}$ , about 100  $\mu\text{m}$  to about 500  $\mu\text{m}$ , or about 500  $\mu\text{m}$  to about 1000  $\mu\text{m}$ .

Following leaching, superabrasive table 214 may comprise a first volume 221 and a second volume 223. Following leaching, superabrasive table 214 may comprise, for example, a first volume 221 that contains a metal-solvent catalyst. An amount of metal-solvent catalyst in first volume 221 may be substantially the same prior to and following leaching. In various embodiments, first volume 221 may be remote from one or more exposed surfaces of superabrasive table 214.

Second volume 223 may comprise a volume of superabrasive table 214 having a lower concentration of the interstitial material than first volume 221. For example, second volume 223 may be substantially free of a metal-solvent catalyst. However, small amounts of catalyst may remain within interstices that are inaccessible to the leaching process. Second volume 223 may extend from one or more surfaces of superabrasive table 214 (e.g., superabrasive face 220, superabrasive side surface 222, and/or chamfer 224) to a depth D from the one or more surfaces. Second volume 223 may be located adjacent to one or more surfaces of superabrasive table 214. An amount of metal-solvent catalyst in first volume 221 and/or second volume 223 may vary at different depths in superabrasive table 214.

In at least one embodiment, superabrasive table 214 may include a transition region 225 between first volume 221 and second volume 223. Transition region 225 may include amounts of metal-solvent catalyst varying between an amount of metal-solvent catalyst in first volume 221 and an amount of metal-solvent catalyst in second volume 223. In various examples, transition region 225 may comprise a relatively narrow region between first volume 221 and second volume 223.

FIGS. 6A and 6B are magnified cross-sectional side views of a portion of the superabrasive table 214 illustrated in FIG. 5A according to various embodiments. As shown in FIGS. 6A and 6B, superabrasive table 214 may comprise grains 234 and interstitial regions 236 between grains 234 defined by grain surfaces 238. Grains 234 may comprise grains formed of any suitable superabrasive material, including, for example, diamond grains. At least some of grains 234 may be bonded to one or more adjacent grains 234, forming a polycrystalline diamond matrix.

Interstitial material 239 may be disposed in at least some of interstitial regions 236. Interstitial material 239 may comprise any suitable material, such as, for example, a metal-solvent catalyst, tungsten, and/or tungsten carbide. As shown in FIG. 6A, interstitial material 239 may not be present in at least some of interstitial regions 236. At least a portion of interstitial material 239 may be removed from at least some of interstitial regions 236 during a leaching procedure. For example, a substantial portion of interstitial material 239 may be removed from second volume 223 during a leaching procedure. In some embodiments, as shown in FIG. 6B, at least some of interstitial regions 236 of second volume 223 may be partially filled with interstitial material 238 that is not removed by leaching. Additionally interstitial material 239 may remain in a first volume 221 following a leaching procedure.

In some examples, interstitial material 239 may be removed from table 214 to a depth that improves the performance and/or heat resistance of a surface of super-abrasive table 214 to a desired degree. In some embodiments, interstitial material 239 may be removed from super-

14

abrasive table 214 to a practical limit. In order to remove interstitial material 239 from superabrasive table 214 to a depth beyond the practical limit, for example, significantly more time, temperature, and/or other process parameter(s) 5 may be required. In some embodiments, interstitial material 239 may be removed from superabrasive table 214 to a practical limit or desired degree where interstitial material remains in at least a portion of superabrasive table 214. In various embodiments, superabrasive table 214 may be fully 10 leached so that interstitial material 239 is substantially removed from a substantial portion of superabrasive table 214.

114. In at least one embodiment, as will be described in greater detail below, interstitial material 239 may be leached from  
15 a superabrasive material, such as a PCD material in superabrasive table 214, by exposing the superabrasive material to a suitable processing solution in the presence of an electrode and applying a charge (e.g., a positive charge) to the superabrasive material and an opposite charge (e.g., a  
20 negative charge) to the electrode. Interstitial material 239 may include a metal-solvent catalyst, such as cobalt, nickel, iron, and/or alloys thereof.

tungsten-containing material may be about greater than 0 to about 1.0 weight %. In a more specific embodiment, the first concentration of the metallic material may be about 0.8 weight % to about 1.0 weight %, and the second concentration of the at least one carbide and/or tungsten-containing material may be about 0.5 weight % to about 1.0 weight % (e.g., about 0.5 weight % to about 0.8 weight %). In an embodiment, the second concentration of the at least one carbide and/or tungsten-containing material is substantially the same in leached volume 223 and unleached volume 221 because the electrochemically leaching process used to form leached volume 223 preferentially removes metallic material and may not cause removal of the at least one carbide material. The concentration of the tungsten-containing material (e.g., tungsten and/or tungsten carbide) and/or the metal-solvent catalyst in leached volume 223 of PCD table 214 may gradually or substantially continuously increase with distance toward to first volume 221.

In a more specific embodiment, diamond may be about 95 weight % to about 99 weight % of leached volume 223, the first concentration of the metallic material may be about 0.3 weight % to about 1.2 weight %, and the second concentration of the at least one carbide and/or tungsten-containing material may be about 1.5 weight % to about 3.0 weight %. In a more specific embodiment, diamond may be about 95 weight % to about 99 weight % of leached volume 223, the first concentration of the metallic material may be about 0.8 weight % to about 1.2 weight %, and the second concentration of the at least one carbide and/or tungsten-containing material may be about 0.6 weight % to about 0.8 weight %. In a more specific embodiment, diamond comprises about 96 weight % to about 98 weight % of leached volume 223, the first concentration of the metallic material may be about 1.0 weight % to about 1.2 weight %, the second concentration of the at least one carbide and/or tungsten-containing material may be about 0.6 weight % to about 0.8 weight %, and the leached volume further includes about 0.15 weight % to about 0.25 weight % of another type of carbide and/or tungsten-containing material such as cobalt tungsten carbide. In any of the foregoing embodiments, in leached volume 223, a tungsten-containing material (e.g., the at least one carbide material) may be disposed interstitially between the bonded diamond grains, but may be unbonded or bonded to adjacent diamond grains. The inventors currently believe that the presence of the carbide and/or tungsten-containing material (e.g., tungsten and/or tungsten carbide) may contribute to enhanced abrasion resistance and/or toughness compared to a conventionally leached PCD table in which the carbide material is removed during the conventional leaching thereof.

In some embodiments, the PCD table may exhibit different layers of different types of leached volumes resulting from leaching using different types of leaching processes. For example, in an embodiment, the PCD table may first be leached to remove metallic material and carbide material in a conventional non-electrochemical leaching process such as exposure to or immersion in an acid solution (e.g., hydrochloric acid, hydrofluoric acid, nitric acid, or mixtures thereof) followed by electrochemically leaching the PCD table according to any of the embodiments disclosed herein. In another embodiment, the PCD table may be electrochemically leached according to any of the embodiments disclosed herein followed by leaching to remove metallic material and/or carbide material in a conventional non-electrochemical leaching process such as exposure to or immersion in the acid solution which may be performed after machining and/or selected masking of the PCD table. Any process

disclosed herein may be used in any order to achieve the PCD structures disclosed herein, without limitation (e.g., electrochemical leaching, non-electrochemical leaching, masking, machining, grinding, combinations thereof, etc.).

For example, FIG. 5B is a cross-sectional side view of a portion of a PCD table according to at least one embodiment after a conventional non-electrochemical leaching process followed by electrochemically leaching the PCD table. PCD table 214 includes a first leached volume 227 that substantially contours superabrasive face 220, superabrasive side surface 222, and chamfer 224. First leached volume 227 extends inwardly from superabrasive face 220, superabrasive side surface 222, and chamfer 224 to a depth D1. First leached volume 227 is formed by at least a conventional non-electrochemical leaching process, such as exposure to or immersion of PCD table 214 in a suitable acid, such as hydrofluoric acid, nitric acid, hydrochloric acid, or combinations thereof. PCD table 214 further includes a second leached volume 229 positioned between first leached volume 227 and an unleached volume 221' that is bonded to the cobalt-cemented tungsten carbide substrate. In some embodiments, second leached volume 229 may substantially contour first leached volume 227. A transition region 231 may be present between first leached volume 227 and second leached volume 229 that has a composition that gradually transitions from the composition of first leached volume 227 to the composition in second leached volume 229. For example, the concentration of carbide material (e.g., tungsten carbide) and/or tungsten-containing material in PCD table 214 may gradually or substantially continuously increase with distance toward to second leached volume 229. The inventors currently believe that gradually or substantially continuously increase in concentration of the carbide material (e.g., tungsten carbide) may help moderate residual stresses in PCD table 214, which may enhance toughness and/or abrasion resistance of PCD table 214. Second leached volume 229 is formed by electrochemically leaching PCD table 214 according to any of the embodiments disclosed herein.

For example, first leached volume 227 may be formed by conventional leaching, which depletes first leached volume 227 of both metal-solvent catalyst or other metallic material (e.g., cobalt or other Group VIII metal) and carbide material (e.g., tungsten carbide and/or other carbides). In an embodiment, first leached volume 227 and PCD table 214 may be further exposed to an electrochemical leaching process, which preferentially removes metal-solvent catalyst or other metallic material from PCD table 214 over carbide material and/or tungsten-containing material (e.g., tungsten carbide and/or tungsten) from first leached volume 227 and further from region(s) of PCD table 214 underlying first leached volume 227 to form second leached volume 229. Second leached volume 229 extends inwardly from superabrasive face 220, superabrasive side surface 222, and chamfer 224 to a depth D2. Depth D2' measured from transition region 231 may be the same, less than, or greater than the depth D1. For example, depths D1 and D2' may each be approximately 2500  $\mu\text{m}$ , such as approximately 100  $\mu\text{m}$  to approximately 1000  $\mu\text{m}$ , approximately 100  $\mu\text{m}$  to approximately 500  $\mu\text{m}$ , or approximately 200  $\mu\text{m}$  to approximately 450  $\mu\text{m}$ . In another embodiment, a precursor to first leached volume 227 and second leached volume 229 may be formed by electrochemically leaching PCD table 214 to the depth D2, followed by exposing the electrochemically leached region in a limited manner to a leaching solution or leaching agent to non-electrochemically leach PCD table 214 to the depth D1 to form first leached volume 227. In such embodiments, the

first leached volume 227 may exhibit a smaller carbide, tungsten-containing, and/or metallic material(s) content than the second leached volume 229, due at least partially to the preferential removal of cobalt over carbide and/or tungsten-containing materials exhibited during electrochemical leaching used to form the second leached volume 229.

Second leached volume 229 may exhibit any of the compositions discussed above with respect to FIG. 5A for the leached volume 223. First leached volume 227 may have less carbide material, less tungsten-containing material, and less metallic material therein than second leached volume 229. For example, first leached volume 227 may be substantially free of carbide material (e.g., tungsten carbide) and/or tungsten-containing material (e.g., tungsten), or may have carbide material and/or tungsten-containing material present in a concentration of less than 0.7 weight %, about 0.2 weight % to about 0.6 weight %, or about 0.1 weight % to about 0.3 weight %; and the metallic material (e.g., cobalt or other Group VIII metal) may be present in first leached volume 227 in a concentration of less than in second leached volume 229, such as about 1.2 weight %, less than 1.0 weight %, or about 0.2 weight % to about 0.6 weight %.

FIG. 5C is an embodiment of polycrystalline diamond compact ("PDC") 10C including PCD table 214C bonded to substrate 12. PCD table 214C includes unleached volume 221C extending inwardly from superabrasive face 220, which may form at least a majority of the volume of PCD table 214C. PCD table 214C further includes first leached volume 227C extending inwardly from chamfer 224, superabrasive side surface 222, and superabrasive face 220 to a selected or a varying leach depth therefrom. First leached volume 227C may exhibit any of the compositions disclosed herein for first leached volume 227 shown in FIG. 5B. PCD table 214C further includes second leached volumes 229C between which first leached volume 227C is disposed. Second leached volumes 229C may exhibit any of the compositions disclosed herein for second leached volume 229 shown in FIG. 5B. A first second leached volume 229C extends from adjacent to first leached volume 227C, along and inwardly from superabrasive side surface 222 and toward substrate 12. A second leached volume 229C extends from adjacent first leached volume 227C inwardly from and along superabrasive face 220. For example, a depth of second leached volume 229C measured inwardly from superabrasive face 220 may decrease with increasing distance away the adjacent first leached volume 227C.

First and second leached volumes 227C and 229C may be formed according to a number of different processes. In an embodiment, PCD table 214C may be appropriately masked with masking layers (e.g., shown in FIG. 26) followed by electrochemically leaching PCD table 214C according to any of the embodiments disclosed herein to form a precursor to second leached volumes 229C. After electrochemical leaching, PCD table 214C may be masked using appropriate masking layers so generally only appropriate portions of superabrasive side surface 222, superabrasive face 220, and chamfer 224 of first leached volume 227C to be formed are exposed to a non-electrochemical leaching process, which removes the tungsten-containing material (e.g., tungsten and/or tungsten carbide) that remained interstitially after electrochemical leaching. In other embodiments, in addition to or as an alternative to masking PCD table 214C, the precursor to second leached volume 229C may be filled with an internal masking material (e.g., a polymeric material such as an epoxy, a carbide, a refractory metal material such as tantalum, molybdenum, alloys thereof, combinations thereof etc.) that at least partially fills interstitial regions thereof and

is resistant to acids used in the non-electrochemical leaching process used to form first leached volume 227C. In another embodiment, the first and second leached volumes 227C and 229C may be separately and selectively formed by appropriately masking PCD table 214C and exposing PCD table 214C to selected electrochemical leaching processes and/or non-electrochemical leaching processes (in any desired order, without limitation). For example, first leached volume 227C may be formed by non-electrochemical leaching, then leached volume 229C may be formed by electrochemical leaching (optionally, via use of masking and/or shaped electrodes).

FIG. 5D is an embodiment of PDC 10D including PCD table 214D bonded to substrate 12. PCD table 214D includes unleached volume 221D extending inwardly from superabrasive face 220 to substrate 12, which may form at least a majority of the volume of PCD table 214D. PCD table 214D further includes first leached volume 227D extending inwardly from chamfer 224, superabrasive side surface 222, and a portion of superabrasive face 220 proximate chamfer 224 to a selected or a varying leach depth therefrom. First leached volume 227D may exhibit any of the compositions disclosed herein for first leached volume 227 shown in FIG. 5B. PCD table 214D further includes second leached volume 229D substantially contouring first leached volume 227D and extending from superabrasive face 220 to superabrasive side surface 222 as it substantially contours first leached volume 227D. In the illustrated embodiment, second leached volume 229D may extend to an interface between PCD table 214D and substrate 12, provided a barrier (e.g., tungsten or binderless chemical vapor deposited tungsten carbide) coats at least a portion of substrate 12 at the interface. The barrier protects the underlying substrate 12 from being affected by the leaching process used to form second leached volume 229D. In other embodiments, second leached volume 229D may be spaced from substrate 12 a standoff distance by a portion of unleached volume 221D. Second leached volume 229D may exhibit any of the compositions disclosed herein for second leached volume 229 shown in FIG. 5B.

First and second leached volumes 227D and 229D may be formed according to a number of different processes. In an embodiment, PCD table 214D may be appropriately masked with masking layers (e.g., shown in FIG. 26) followed by electrochemically leaching PCD table 214D according to any of the embodiments disclosed herein to form a precursor to second leached volume 229D. After electrochemical leaching, PCD table 214D may be masked using appropriate masking layers so generally only appropriate portions of superabrasive side surface 222, superabrasive face 220, and chamfer 224 of first leached volume 227D to be formed are exposed to a non-electrochemical leaching process, which removes the tungsten-containing material (e.g., tungsten and/or tungsten carbide) that remained interstitially after electrochemical leaching. In other embodiments, in addition to or as an alternative to masking PCD table 214D, interstitial regions of second leached volume 229D may be filled with any of the disclosed internal masking materials that are resistant to the acids used in the non-electrochemical leaching process used to form first leached volume 227D. In another embodiment, the first and second leached volumes 227D and 229D may be separately and selectively formed by appropriately masking PCD table 214D and exposing PCD table 214D to selected electrochemical leaching processes and/or non-electrochemical leaching processes (in any desired order, without limitation). Optionally, shaped

electrodes as shown in the embodiments in FIGS. 18-22 may be used to selectively form second leached volume 229D.

FIG. 5E is an embodiment of PDC 10E including PCD table 214E bonded to substrate 12. PCD table 214E includes unleached volume 221E extending inwardly from substrate 12, which may form at least a majority of the volume of PCD table 214E. PCD table 214E further includes first leached volume 227E extending inwardly from chamfer 224, superabrasive side surface 222, and a portion of superabrasive face 220 proximate chamfer 224 to a selected or a varying leach depth therefrom. First leached volume 227E may exhibit any of the compositions disclosed herein for first leached volume 227 shown in FIG. 5B. PCD table 214E further includes second leached volume 229E substantially contouring first leached volume 227E and extending inwardly from superabrasive face 220 located between first leached volume 227E. A portion of second leached volume 229D that substantially contours first leached region 227C is located between unleached volume 221E and first leached region 227C. Second leached volume 229D also extends inwardly from superabrasive side surface 222 at a location adjacent to first leached volume 227D. Second leached volume 229E may exhibit any of the compositions disclosed herein for second leached volume 229 shown in FIG. 5B.

First and second leached volumes 227E and 229E may be formed according to a number of different processes. In an embodiment, PCD table 214E may be appropriately masked with masking layers (e.g., shown in FIG. 26) followed by electrochemically leaching PCD table 214E according to any of the embodiments disclosed herein to form a precursor to second leached volume 229E. After electrochemical leaching, PCD table 214E may be masked using appropriate masking layers so generally only appropriate portions of superabrasive side surface 222, superabrasive face 220, and chamfer 224 of first leached volume 227E to be formed are exposed to a non-electrochemical leaching process, which removes the tungsten-containing material (e.g., tungsten and/or tungsten carbide) that remained after electrochemical leaching. In other embodiments, in addition to or as an alternative to masking PCD table 214E, second leached volume 229E may be filled with any of the disclosed internal masking materials that are resistant to the acids used in the non-electrochemical leaching process used to form first leached volume 227E. In another embodiment, the first and second leached volumes 227E and 229E may be separately and selectively formed by appropriately masking PCD table 214E and exposing PCD table 214E to selected electrochemical leaching processes and/or non-electrochemical leaching processes (in any desired order, without limitation).

FIGS. 7-28 show configurations of superabrasive elements and electrodes for leaching the superabrasive elements according to various embodiments. The configurations illustrated in these figures may enable selective leaching of portions of the superabrasive elements to form desired leach profiles within the superabrasive elements. While certain configurations of superabrasive elements are shown and described herein for purposes of illustration, the apparatuses and methods described herein may be applied to any superabrasive article having any suitable material, shape, and configuration, without limitation.

FIGS. 7 and 8 illustrate a superabrasive element 10 disposed near an electrode 40 according to at least one embodiment. As illustrated in FIGS. 7 and 8, superabrasive element 10 may comprise a superabrasive table 14 affixed to or formed upon a substrate 12. Superabrasive table 14 may be affixed to substrate 12 at interface 26, which may be a planar or non-planar interface. Superabrasive element 10

may comprise a rear surface 18, a superabrasive face 20, and an element side surface 15. In some embodiments, element side surface 15 may include a substrate side surface 16 formed by substrate 12 and a superabrasive side surface 22 formed by superabrasive table 14. Rear surface 18 may be formed by substrate 12.

Superabrasive element 10 may also comprise a chamfer 24 (i.e., sloped or angled) formed by superabrasive table 14. Chamfer 24 may comprise an angular and/or rounded edge 10 formed at the intersection of superabrasive side surface 22 and superabrasive face 20. The chamfer may extend between edge 27 at the superabrasive face 20 and edge 28 at the superabrasive side surface 22. Any other suitable surface shape may also be formed at the intersection of superabrasive side surface 22 and superabrasive face 20, including, without limitation, an arcuate surface (e.g., a radius, an ovoid shape, or any other rounded shape), a sharp edge, multiple chamfers/radii, a honed edge, and/or combinations of the foregoing.

Electrode 40 may comprise any suitable size, shape, and/or geometry, without limitation. According to at least one embodiment, at least a portion of electrode 40 may have a substantially cylindrical shape. For example, electrode 40 may comprise a substantially cylindrical outer surface 25 surrounding a central axis of electrode 40, as illustrated in FIGS. 7 and 8. Electrode 40 may comprise any suitable material that may conduct electricity. Electrode 40 may have an outer diameter that is substantially the same as the outer diameter of element side surface 15 of superabrasive element 10. In at least one embodiment, electrode 40 may comprise copper. Electrode 40 may comprise any suitable electrically conductive material, such as, for example, copper, tungsten carbide, cobalt, zinc, iron, platinum, palladium, niobium, graphite, graphene, nichrome, gold, silver, alloys 30 thereof, any suitable metallic material, and/or any other suitable electrically conductive material, without limitation.

According to various embodiments, a charge may be applied to superabrasive element 10 and electrode 40 through electrical conductors (e.g., wires or any suitable 40 electrical conductor) 44 and 42, respectively. For example, in order to apply a current to a processing solution for processing superabrasive element 10, superabrasive element 10 and electrical conductor 44 may be positioned in the processing solution (e.g., optionally, with a leaching cup 30 or other protective covering). A charge (e.g., a positive charge) may be applied to at least a portion of substrate 12 (e.g., rear surface 18) of superabrasive element 10 through electrical conductor 44 and an opposite charge (e.g., a negative charge) may be applied to electrode 40 through 45 electrical conductor 42. In at least one embodiment, electrical conductor 44 may be electrically connected to substrate 12 by an electrode electrically connected to (e.g., positioned abutting) substrate 12. In some embodiments, electrical conductor 44 may be directly connected to superabrasive table 14 by an electrode electrically connected to (e.g., positioned abutting) superabrasive table 14.

When superabrasive element 10 is disposed in a processing solution such that at least a portion of superabrasive table 14 and electrode 40 are exposed to the processing solution 60 and a voltage is applied to the processing solution via electrode 40 and superabrasive table 14 when superabrasive element 10 is disposed in the processing solution, interstitial materials may be removed from at least a portion of superabrasive table 14 of superabrasive element 10 near electrode 40.

FIGS. 9A and 9B illustrate a superabrasive element 10 disposed near an electrode 40 and positioned within a

protective leaching cup 30 according to at least one embodiment. As illustrated in FIGS. 9A and 9B, superabrasive element 10 may comprise a superabrasive table 14 affixed to or formed upon a substrate 12. Superabrasive table 14 may be affixed to substrate 12 at interface 26, which may be a planar or non-planar interface. Superabrasive element 10 may comprise a rear surface 18, a superabrasive face 20, and an element side surface 15. In some embodiments, element side surface 15 may include a substrate side surface 16 formed by substrate 12 and a superabrasive side surface 22 formed by superabrasive table 14. Rear surface 18 may be formed by substrate 12. Superabrasive element 10 may also comprise a chamfer 24 formed by superabrasive table 14. Chamfer 24 may comprise an angular and/or rounded edge formed between superabrasive side surface 22 and superabrasive face 20.

As shown in FIGS. 9A and 9B, superabrasive element 10 may be positioned within protective leaching cup 30 such that protective leaching cup 30 surrounds at least a portion of superabrasive element 10, including substrate 12. When superabrasive element 10 is positioned within protective leaching cup 30, at least a portion of superabrasive element 10, such as superabrasive table 14 and/or substrate 12, may be positioned adjacent to and/or contacting a portion of protective leaching cup 30. For example, protective leaching cup 30 may be configured to contact at least a portion of element side surface 15 of superabrasive element 10, forming a seal between protective leaching cup 30 and superabrasive element 10, where the leaching cup 30 is partially or fully impermeable to various fluids, such as a leaching material (e.g., a leaching solution).

Protective leaching cup 30 may be formed of any suitable material, without limitation. For example, protective leaching cup 30 may comprise a flexible, elastic, malleable, and/or otherwise deformable material configured to surround and/or contact at least a portion of superabrasive element 10. Protective leaching cup 30 may prevent damage to a portion of superabrasive element 10 when at least another portion of superabrasive element 10 is exposed to various reactive agents. For example, protective leaching cup 30 may prevent a leaching solution from chemically damaging certain portions of superabrasive element 10, such as portions of substrate 12, portions of superabrasive table 14, or both, during leaching. Protective leaching cup 30 may be formed with an opening 32 configured to allow electrical conductor 44 to contract rear surface 18 of superabrasive element 10. Optionally, opening 32 may be sealed with a sealant (e.g., silicone, epoxy, etc.) to prevent the leaching solution from damaging substrate 12, if necessary.

In various embodiments, protective leaching cup (e.g., layer) 30 may comprise one or more materials that are substantially inert and/or otherwise resistant to acids, bases, and/or other reactive components present in a leaching solution used to leach superabrasive element 10. In some embodiments, protective leaching cup 30 may comprise one or more materials exhibiting significant stability at various temperatures and/or pressures, including selected temperatures and/or pressures used in leaching and/or otherwise processing superabrasive element 10. In some embodiments, protective leaching cup 30 may include one or more polymeric materials, such as, for example, nylon, polytetrafluoroethylene (PTFE), polyethylene, polypropylene, rubber, silicone, and/or other polymers, and/or a combination of any of the foregoing, without limitation. For example, protective leaching cup 30 may comprise PTFE blended with one or more other polymeric materials.

Electrode 40 may be disposed near and/or abutting superabrasive element 10. For example, as shown in FIG. 9A, electrode 40 may be disposed near, but separated from, superabrasive table 14 of superabrasive element 10. Electrode 40 may be disposed any suitable distance away from superabrasive element 10. Optionally, as illustrated in FIG. 9B, electrode 40 may be disposed adjacent to at least a portion of superabrasive element 10. For example, electrode 40 may be electrically connected to (e.g., positioned abutting) a portion of superabrasive table 14, such as superabrasive face 20. Although not shown, electrode 40 may be disposed adjacent to any other suitable portion of superabrasive table 14, such as, for example, superabrasive side surface 22 and/or chamfer 24. According to various embodiments, a charge may be applied to superabrasive element 10 and electrode 40 through electrical conductors 44 and 42, respectively.

FIG. 9C is a cross-sectional side view of a leaching assembly according to at least one embodiment. As illustrated in FIG. 9C, superabrasive element 10 (as described with respect to FIGS. 9A and 9B) may be positioned within a protective leaching cup 30 (as described with respect to FIGS. 9A and 9B) and disposed near electrode 40. Superabrasive element 10, electrode 40, and protective leaching cup 30 may further be positioned within a processing vessel 70.

As shown in FIG. 9C, processing vessel 70 may have a rear wall 74 and a side wall 73 defining a cavity 76. Rear wall 74 and side wall 73 may have any suitable shape, without limitation. Processing vessel 70 may include an opening 78 opposite rear wall 74. Cavity 76 may contain a processing solution 72 such that at least a portion of superabrasive element 10 is exposed to processing solution 72. Superabrasive element 10 may be positioned in cavity 76 so that superabrasive element 10 is positioned adjacent to or near rear wall 74 of processing vessel 70. In some embodiments, superabrasive element 10 may be positioned and/or secured within processing vessel 70 using any suitable mechanism, without limitation. Processing vessel 70 may be larger than leaching cup 30, so that there are gaps between leaching cup 30 and processing vessel 70. In other embodiments, more than one superabrasive element 10 and protective leaching cup 30 (e.g., 10 or more, 20 or more, etc.) may be placed within a single processing vessel 70 for loading.

According to some embodiments, processing solution 72 may comprise a conductive solution (e.g., a conductive aqueous solution, a conductive non-aqueous solution, etc.). Solvents in such processing solution 72 may comprise water and/or any other suitable solvent, without limitation. Processing solution 72 may also comprise dissolved electrolytes. Such electrolytes may comprise any suitable electrolyte compounds, including, without limitation, acetic acid; ammonium chloride; arsenic acid; ascorbic acid; citric acid; formic acid; hydrobromic acid; hydrofluoric acid; hydroiodic acid; lactic acid; malic acid; nitric acid; oxalic acid; phosphoric acid; propionic acid; pyruvic acid; succinic acid; tartaric acid; and/or any suitable carboxylic acid (e.g., monocarboxylic acid, polycarboxylic acid, etc.); and/or ions, salts, and/or esters of any of the foregoing; and/or any combination of the foregoing. Such electrolytes may be present in processing solution 72 at any suitable concentration, without limitation. For example, one or more electrolytes may be present in processing solution 72 at a concentration of, for example, less than approximately 5 M. In certain embodiments, one or more electrolytes may be present in processing solution 72 at a concentration of, for example, less than approximately 0.01 M. In at least one

embodiment, one or more electrolytes may be present in processing solution 72 at a concentration of, for example, between approximately 0.01 M and approximately 3 M. In some embodiments, one or more electrolytes may be present in processing solution 72 at a concentration of, for example, between approximately 0.1 M and approximately 1 M. In additional embodiments, one or more electrolytes may be present in processing solution 72 at a concentration of, for example, between approximately 0.2 M and approximately 0.4 M. In at least one embodiment, one or more electrolytes may be present in processing solution 72 at a concentration of, for example, approximately 0.3 M.

Processing solution 72 may have a pH of between approximately 1 and approximately 12. In certain embodiments, processing solution 72 may have a pH below approximately 1. In some embodiments, processing solution 72 may have a pH of between approximately 1 and approximately 7. In at least one embodiment, for example, processing solution 72 may have a pH of approximately 2.0.

In some embodiments, processing solution 72 may include metal salts, such as cobalt salts, iron salts, nickel salts, copper salts, and/or any other suitable transition metal salts, and/or any other suitable metal ion salts, without limitation. Such metal salts may include, for example, cobalt chloride, cobalt nitrate, iron chloride, and/or any other suitable metal salts, without limitation. One or more metal salts may be present in processing solution 72 at any suitable concentration, including, for example, a concentration of less than approximately 2 M. In at least one embodiment, one or more metal salts may be present in processing solution 72 at a concentration of, for example, between approximately 0.01 M and approximately 1 M. In some embodiments, one or more metal salts may be present in processing solution 72 at a concentration of, for example, between approximately 0.03 M and approximately 0.5 M. In additional embodiments, one or more metal salts may be present in processing solution 72 at a concentration of, for example, between approximately 0.05 M and approximately 0.3 M. In at least one embodiment, for example, one or more compounds may be dissolved in processing solution 72 at a concentration of, for example, approximately 0.1 M.

Processing solution 72 may further include any other suitable components, without limitation, including, for example, a buffering agent (e.g., boric acid, an amine compound such as ethylenediamine, triethanolamine, ethanolamine, etc.), a pH control agent (e.g., sodium hydroxide, etc.), and/or a conducting agent (e.g., sodium sulfate, ammonium citrate, etc.). In some examples, processing solution 72 may comprise an acid (e.g., a mineral acid) suitable for increasing the solubility of a metallic material, such as cobalt or any other material, with respect to processing solution 72, including, for example, nitric acid, hydrochloric acid, phosphoric acid, sulfuric acid, boric acid, hydrofluoric acid, and/or any combination of the foregoing mineral acids. The acid may be selected for its ability to attack and/or dissolve a metallic material within superabrasive table 14. Processing solution 72 may then carry the dissolved metallic material out of superabrasive table 14. In some examples, a suitable acid may be configured to increase the solubility of a metallic material, such as cobalt, in the processing mixture, thereby facilitating leaching of the metallic material from superabrasive table 14 using the processing mixture. In additional examples, an acid may be configured to increase the solubility of iron, tungsten, and/or nickel in the processing mixture.

Processing solution 72 may comprise a complexing agent dissolved in the solvent. The complexing agent may com-

prise a compound suitable for forming metal complexes with various interstitial materials, including, for example, tungsten and/or tungsten carbide. The complexing agent may form metal complexes with tungsten and/or tungsten carbide present in a superabrasive material, thereby inhibiting or preventing the formation and/or build-up of tungsten oxides, such as  $WO_2$ ,  $W_2O_5$ , and  $WO_3$ , in the superabrasive material. Metal complexes formed between the complexing agent and tungsten and/or tungsten carbide may be soluble in processing solution 72, thereby enabling the metal complexes to be easily removed from superabrasive table 14. Accordingly, the complexing agent may facilitate the removal of tungsten and/or tungsten carbide from a leached portion of superabrasive table 14, thereby reducing the amount of residual tungsten, tungsten carbide, and/or tungsten oxide present in a leached region of superabrasive table 14. The complexing agent may also facilitate removal of additional metal compounds that may be present in superabrasive table 14. Examples of suitable compounds that may function as complexing agents include, without limitation, phosphoric acid, citric acid, tartaric acid, oxalic acid, ammonium chloride, and/or any combination of the foregoing. Examples of suitable complexing agents include chelators capable of chelating with one or more metal interstitial materials. Suitable chelators may include polycarboxylic acids such as any of those disclosed above (e.g., citric acid), or any other composition capable of chelating with a metal ion.

In various embodiments, processing solution 72 may optionally include one or more of an electrolyte (e.g., acetic acid, ammonium chloride, arsenic acid, ascorbic acid, citric acid, formic acid, hydrobromic acid, hydrofluoric acid, hydroiodic acid, lactic acid, malic acid, nitric acid, oxalic acid, phosphoric acid, propionic acid, pyruvic acid, succinic acid, tartaric acid, carboxylic acid, etc.), an acid (e.g., nitric acid, hydrochloric acid, phosphoric acid, sulfuric acid, boric acid, hydrofluoric acid, etc.), a metal salt (e.g., cobalt salts, iron salts, etc.), a buffering agent (e.g., boric acid, an amine compound such as ethylenediamine, triethanolamine, ethanolamine, etc.), a pH control agent (e.g., sodium hydroxide, etc.), a conducting agent (e.g., sodium sulfate, ammonium citrate, etc.), a complexing agent (e.g., phosphoric acid, citric acid, tartaric acid, oxalic acid, ammonium chloride, etc.), and/or combinations of the foregoing, without limitation.

Electrode 40 may comprise any suitable size, shape, and/or geometry, without limitation. According to at least one embodiment, at least a portion of electrode 40 may be substantially disk shaped. For example, electrode 40 may comprise a disk shape having a circular or non-circular periphery. Electrode 40 may comprise a suitable electrically conductive material, such as, for example, a metallic, semi-metallic, and/or graphitic material. For example electrode 40 may include, without limitation, copper, tungsten carbide, cobalt, zinc, iron, platinum, palladium, niobium, graphite, graphene, nichrome, gold, silver, alloys thereof, any suitable metallic material, and/or any other suitable electrically conductive material, without limitation.

According to various embodiments, a charge may be applied to superabrasive element 10 and electrode 40 through electrical conductors 44 and 42, respectively. For example, in order to apply a current to processing solution 72 for processing superabrasive element 10, at least a portion of superabrasive element 10 may be positioned in processing solution 72 and a charge may be applied to at least a portion of superabrasive element 10 (e.g., rear surface 18 of substrate 12) through electrical conductor 44. For

example, a positive charge may be applied to substrate 12 such that at least a portion of superabrasive element 10 acts as an anode. An opposite charge may be applied to electrode 40 through electrical conductor 42. For example, a negative charge may be applied to electrode 40 such that electrode 40 acts as a cathode. In at least one embodiment, electrical conductor 44 may be electrically connected to substrate 12 by an electrode electrically connected to (e.g., positioned abutting) substrate 12. In some embodiments, electrical conductor 44 may be directly connected to superabrasive table 14 by an electrode electrically connected to (e.g., positioned abutting and/or disposed at least partially within) superabrasive table 14.

According to some embodiments, a voltage of less than approximately 10 V may be applied to processing solution 72 via electrode 40 and superabrasive element 10. In some embodiments, a voltage of approximately 0.01 V to approximately 5 V may be applied to processing solution 72. In some embodiments, a voltage of approximately 0.5 V to approximately 3 V may be applied to processing solution 72. In some embodiments, a voltage of approximately 0.1 V to approximately 3 V may be applied to processing solution 72. In additional embodiments, a voltage of approximately 0.4 V to approximately 2.4 V may be applied to processing solution 72. In some embodiments, a voltage of approximately 0.5 V, 0.6 V, 0.7 V, 0.8 V, 0.9 V, or 1.0 V may be applied to processing solution 72.

In various embodiments, a voltage applied to processing solution 72 may be changed one or more times while superabrasive element 10 is exposed to processing solution 72. For example, the electrical conductivity of processing solution 72 may change during processing of superabrasive element 10 such that different voltages are required over time to maintain a desired current flow between superabrasive element 10 and electrode 40. In at least one embodiment, for example, materials removed from superabrasive element 10 and dissolved in processing solution 72 during processing may cause processing solution 72 to decrease in electrical conductivity and increase in electrical resistance. The voltage between superabrasive element 10 and electrode 40 may be increased in conjunction with the decrease in electrical conductivity/increase in electrical resistance so as to maintain a desired current flow through superabrasive element 10 and/or processing solution 72.

When superabrasive element 10 and electrode 40 are disposed in the processing solution 72 such that at least a portion of superabrasive table 14 and electrode 40 are exposed to processing solution 72 and a voltage is applied to processing solution 72 via electrode 40 and superabrasive table 14, interstitial materials may be removed from at least a portion of superabrasive table 14 and electrodeposited onto a portion of electrode 40 exposed to processing (e.g., electroplating) solution 72. For example, a metallic material, such as cobalt, present in at least a portion of superabrasive table 14 may be electrolytically oxidized in the presence of a current flowing between superabrasive element 10 and electrode 40. The oxidized metallic material may then be leached into processing solution 72 as dissolved metal cations. Dissolved metal cations (e.g., cobalt cations) present in processing solution 72 may then be reduced at electrode 40 to form a metal coating on a surface portion of electrode 40. Accordingly, a metallic material, such as cobalt, may be effectively transferred from at least a portion of superabrasive table 14 of superabrasive element 10 to a surface portion of electrode 40 through electrodeposition of the metallic material onto the surface portion of electrode 40.

In additional embodiments, a negative charge may be applied to superabrasive element 10 such that at least a portion of superabrasive element 10 acts as a cathode and a positive charge may be applied to electrode 40 such that electrode 40 acts as an anode. A metallic material present in superabrasive table 14 may be reduced to form metal anions that are dissolved in processing solution 72 and the dissolved metallic anions may then be electrodeposited through oxidation onto a surface portion of electrode 40.

According to various embodiments, superabrasive table 14 may be exposed to processing solution 72 at a desired temperature and/or pressure prior to and/or during leaching. Exposing superabrasive table 14 to a selected temperature and/or pressure during leaching may increase the depth to which the superabrasive table 14 may be leached. Exposing superabrasive table 14 to a selected temperature and/or pressure during leaching may decrease an amount of time required to leach superabrasive table 14 to a desired degree.

In various examples, at least a portion of superabrasive element 10 and processing solution 72 may be heated to a temperature of approximately 15° C. to approximately 280° C. during leaching. According to additional embodiments, at least a portion of a superabrasive element 10 and processing solution 72 may be heated to a temperature of approximately 20° C. to approximately 95° C. during leaching. For example, at least a portion of a superabrasive element 10 and processing solution 72 may be heated to a temperature of approximately 25° C. According to additional embodiments, at least a portion of a superabrasive element 10 and processing solution 72 may be heated to a temperature of approximately 50° C. or greater during leaching.

In various embodiments, at least a portion of superabrasive element 10 and processing solution 72 may be exposed to a pressure of approximately 0 bar to approximately 100 bar during leaching. In additional embodiments, at least a portion of superabrasive element 10 and processing solution 72 may be exposed to a pressure of approximately 20 bar to approximately 80 bar during leaching. In at least one example, at least a portion of superabrasive element 10 and processing solution 72 may be exposed to a pressure of approximately 50 bar during leaching. In at least one example, at least a portion of superabrasive element 10 and processing solution 72 may be exposed to a pressure of approximately 10 bar or greater during leaching.

According to additional embodiments, at least a portion of superabrasive element 10 and processing solution 72 may be exposed to at least one of microwave radiation, and/or ultrasonic energy. By exposing at least a portion of superabrasive element 10 to microwave radiation, induction heating, and/or ultrasonic energy as superabrasive element 10 is exposed to processing solution 72, the rate at which superabrasive table 14 is leached may be increased.

FIGS. 10A-10E show superabrasive elements 110 and assemblies for leaching superabrasive elements 110. FIG. 10A is a cross-sectional side view of a leaching assembly according to at least one embodiment. As shown in FIG. 10A, superabrasive element 110 may be disposed near an electrode 140. Superabrasive element 110 may comprise a superabrasive table 114 that is not affixed to or formed upon a substrate (see superabrasive element 110 illustrated in FIGS. 3 and 4). Superabrasive element 110 may comprise a rear surface 118, a superabrasive face 120, and an element side surface 122. Superabrasive element 110 may also comprise a chamfer 124 formed by superabrasive table 114. Chamfer 124 may comprise an angular and/or rounded edge formed between superabrasive side surface 122 and superabrasive face 120. Superabrasive element 110 may also

comprise a rear chamfer 119 formed by superabrasive table 114 at the intersection of element side surface 122 and rear surface 118.

In some embodiments, as illustrated in FIG. 10A, superabrasive element 110 may not be surrounded by a protective covering, such as a leaching cup. Optionally, superabrasive element 110 may be at least partially covered by a protective layer, such as a leaching cup and/or a masking layer. Superabrasive element 110 and electrode 140 may be positioned within a processing vessel 170. Processing vessel 170 may have a rear wall 174 and a side wall 173 defining a cavity 176. Rear wall 174 and side wall 173 may have any suitable shape, without limitation. Processing vessel 170 may include an opening 178 opposite rear wall 174. Cavity 176 may contain a suitable processing solution 172 such that at least a portion of superabrasive element 110 is exposed to processing solution 172. Superabrasive element 110 may be positioned in cavity 176 so that superabrasive element 110 is disposed near and/or electrically connected to (e.g., abutting) electrode 140.

Electrode 140 may comprise any suitable size, shape, and/or geometry, without limitation. According to at least one embodiment, at least a portion of electrode 140 may be substantially disk shaped. For example, electrode 140 may comprise a disk shape having a circular or non-circular periphery. Electrode 140 may comprise a suitable electrically conductive material, such as, for example, a metallic, semi-metallic, and/or graphitic material. For example electrode 140 may include, without limitation, copper, tungsten carbide, cobalt, zinc, iron, platinum, palladium, niobium, graphite, graphene, nichrome, gold, silver, alloys thereof, any suitable metallic material, and/or any other suitable electrically conductive material, without limitation.

According to various embodiments, a charge may be applied to superabrasive element 110 and electrode 140 through electrical conductors 144 and 142, respectively. For example, in order to apply a current to processing solution 172 for processing superabrasive element 110, at least a portion of superabrasive element 110 may be positioned in processing solution 172 and a charge may be applied to at least a portion of superabrasive element 110 (e.g., rear surface 118 of substrate 112) through electrical conductor 144 and an opposite charge may be applied to electrode 140 through electrical conductor 142. In some embodiments, as shown in FIG. 10A, superabrasive element 110 may be disposed on an electrode 145, which electrically connects electrical conductor 144 to superabrasive element 110. Electrode 145 may separate superabrasive element 110 from processing vessel 170, thereby facilitating contact between a greater surface area of superabrasive element 110 and processing solution 172. Additionally, electrode 145 may facilitate positioning of superabrasive element 110 near electrode 140. Optionally, superabrasive element 110 may be positioned near rear wall 174 of processing vessel 170 and/or may be connected to electrical conductor 144 without electrode 145.

In some embodiments, superabrasive element 110 may be coupled to electrode 145, or optionally, to electrical conductor 144, through brazing, welding, soldering, adhesive bonding, mechanical fastening, and/or any other suitable bonding technique. For example, superabrasive element 110 may be bonded to electrode 145 or electrical conductor 144 by a braze joint (e.g., a carbide forming braze such as a titanium-based braze, etc.). In at least one embodiment, such a braze joint may be coated with a protective layer (e.g., paint layer, epoxy layer, etc.).

In at least one embodiment, a positive charge may be applied to superabrasive element 110, which acts as an anode, via electrical conductor 144 and electrode 145. An opposite charge may be applied to electrode 140 through electrical conductor 142. For example, a negative charge may be applied to electrode 140 such that electrode 140 acts as a cathode. When superabrasive element 110 and electrode 140 are disposed in the processing solution 172 such that at least a portion of superabrasive table 114 and electrode 140 are exposed to processing solution 172 and a voltage is applied to processing solution 172 via electrode 140 and superabrasive table 114, interstitial materials may be removed from at least a portion of superabrasive table 114 and electrodeposited onto a portion of electrode 140 exposed to processing (e.g., electroplating) solution 172. Superabrasive element 110 may be exposed to processing solution 172 and/or a charge may be applied to processing solution 172 until a desired level of leaching is obtained.

FIGS. 10B and 10C illustrate superabrasive elements 110 of FIG. 10A that have been leached to different extents. FIG. 10B shows superabrasive element 110 that has been leached substantially throughout superabrasive table 114. Accordingly, superabrasive table 114 may have a leached volume 123 that substantially occupies the entire volume of superabrasive table 114. According to various embodiments, at least some of interstitial regions in leached volume 123 may be at least partially filled with interstitial material that is not removed by leaching.

FIG. 10C shows superabrasive element 110 that has been partially leached. Superabrasive table 114 may include a first volume 121 comprising an interstitial material and a second volume 123 having a lower concentration of the interstitial material than first volume 121. As shown in FIG. 10C, first volume 121 may be surrounded by second volume 123 such that substantially all surface portions (i.e., superabrasive face 120, element side surface 122, chamfer 124, and chamfer 119) of superabrasive table 114 are defined by second volume 123, from which the interstitial material has been substantially removed.

FIGS. 10D and 10E show cross-sectional side views of leaching assemblies according to various embodiments. As shown in FIGS. 10D and 10E, superabrasive element 110 may be disposed near a plurality of electrodes, including at least electrodes 140A and 140B. Superabrasive element 110 may comprise a superabrasive table 114 that is not affixed to or formed upon a substrate (see superabrasive element 110 illustrated in FIGS. 3 and 4). Superabrasive element 110 may comprise a rear surface 118, a superabrasive face 120, an element side surface 122, a chamfer 124 between superabrasive side surface 122 and superabrasive face 120, and a rear chamfer 119 between element side surface 122 and rear surface 118.

In some embodiments, as illustrated in FIGS. 10D and 10E, superabrasive element 110 may not be surrounded by a protective covering, such as a leaching cup. Optionally, superabrasive element 110 may be at least partially covered by a protective layer, such as a leaching cup and/or a masking layer. Superabrasive element 110 and electrodes 140A and 140B may be positioned within a processing vessel 170. Processing vessel 170 may have a rear wall 174 and a side wall 173 defining a cavity 176. Rear wall 174 and side wall 173 may have any suitable shape, without limitation. Processing vessel 170 may include an opening 178 opposite rear wall 174. Cavity 176 may contain a suitable processing solution 172 such that at least a portion of superabrasive element 110 is exposed to processing solution 172. Superabrasive element 110 may be positioned in cavity

176 so that superabrasive element 110 is disposed near and/or electrically connected to (e.g., abutting) electrode 140.

Electrodes 140A and 140B may comprise any suitable size, shape, and/or geometry, without limitation. According to at least one embodiment, at least a portion of each of electrode 140A and/or electrode 140B may be substantially disk shaped. For example, electrode 140A and/or electrode 140B may comprise a disk shape having a circular or non-circular periphery. In some embodiments, electrode 140A and/or electrode 140B may have a suitable concave and/or convex surface shape. Electrode 140 may comprise a suitable electrically conductive material, such as, for example, a metallic, semi-metallic, and/or graphitic material.

Electrodes 140A and 140B may be disposed at any suitable locations with respect to superabrasive element 110 and each other. For example, electrode 140A and electrode 140B may be disposed on opposite sides of superabrasive element 110. For example, as illustrated in FIG. 10D, electrode 140A may be positioned near superabrasive face 120 and electrode 140B may be positioned near rear surface 118. As illustrated in FIG. 10E, electrode 140A may be positioned near a portion of element side surface 122 and electrode 140B may be positioned near another portion of the element side surface 122. Optionally, electrodes 140A and 140B may be disposed near the same and/or adjacent sides of superabrasive element 110. In certain embodiments, electrode 140A and/or electrode 140B may be electrically connected to (e.g., positioned abutting) at least a portion of superabrasive element 110.

In some embodiments, electrodes 140A and 140B may represent portions of an annular or ring-shaped electrode peripherally surrounding superabrasive element 110, and electrical conductor 142A and/or electrical conductor 142B may be electrically connected to the annular or ring-shaped electrode at one or more locations. For example, electrodes 140A and 140B may comprise sections or portions of an annular or ring-shaped body, and electrical conductors 142A and 142B may be electrically connected to each section.

According to various embodiments, a charge may be applied to superabrasive element 110 through one or more electrical connections. For example, a charge may be applied to superabrasive element 110 through electrical conductor 144A and/or electrical conductor 144B. A charge may be applied to electrode 140A and/or electrode 140B through electrical conductor 142A and/or electrical conductor 142B, respectively. In order to apply a current to processing solution 172 for processing superabrasive element 110, at least a portion of superabrasive element 110 may be positioned in processing solution 172 and a charge may be applied to at least a portion of superabrasive element 110 through electrical conductor 144A and/or electrical conductor 144B and an opposite charge may be applied to electrode 140A and/or electrode 140B through electrical conductor 142A and/or electrical conductor 142B.

In some embodiments, superabrasive element 110 may be coupled to electrical conductor 144A and/or electrical conductor 144B at any suitable location (e.g., element side surface 122 as shown in FIG. 10D, or superabrasive face 120 and/or rear surface 118 as shown in FIG. 10E) through brazing, welding, soldering, adhesive bonding, mechanical fastening, and/or any other suitable bonding technique. For example, superabrasive element 110 may be bonded to electrode 145 or electrical conductor 144 by a braze joint (e.g., a carbide forming braze such as a titanium-based

braze, etc.). In at least one embodiment, such a braze joint may be coated with a protective layer (e.g., paint layer, epoxy layer, etc.).

As shown in FIGS. 10D and 10E, a positive charge may be applied to superabrasive element 110, which acts as an anode, via electrical conductor 144A and/or electrical conductor 144B. A negative charge may be applied to electrode 140A and/or 140B through electrical conductor 142A and/or electrical conductor 142B, respectively, such that electrode 140A and/or 140B acts as a cathode. When superabrasive element 110 and electrodes 140A and 140B are disposed in the processing solution 172 such that at least a portion of superabrasive table 114 and electrodes 140A and 140B are exposed to processing solution 172 and a voltage is applied to processing solution 172 via superabrasive table 114 and electrode 140A and/or electrode 140B, interstitial materials may be removed from at least a portion of superabrasive table 114 and electrode-deposited onto at least a portion of electrode 140A and/or electrode 140B exposed to processing solution 172. Superabrasive element 110 may be exposed to processing solution 172 and/or a charge may be applied to processing solution 172 until a desired level of leaching is obtained.

According to some embodiments, once interstitial materials have been removed from a substantial portion of superabrasive table or once interstitial materials have been removed from superabrasive element 110 to a selected leach depth, a material coupling electrical conductor 144A and/or electrical conductor 144B to superabrasive element 110 may be at least partially degraded by processing solution 172. For example, a braze joint bonding electrical conductor 144A and/or electrical conductor 144B to superabrasive table 114 may have a more positive reduction potential than an interstitial material (e.g., cobalt) within superabrasive table 114. Accordingly, the interstitial material may be preferentially degraded by processing solution 172 prior to substantial degradation of the braze joint. Once the interstitial material is substantially removed from superabrasive table 114 during leaching, processing solution 172 may more aggressively degrade the braze joint such that electrical conductor 144A and/or electrical conductor 144B are electrically and/or physically disconnected from superabrasive element 110.

FIGS. 11 and 12 illustrate a superabrasive element 310 positioned near an electrode 340 according to at least one embodiment. Electrode 340 may comprise any suitable size, shape and/or geometry, without limitation. As illustrated in FIGS. 11 and 12, superabrasive element 310 may comprise a superabrasive table 314 affixed to or formed upon a substrate 312. Superabrasive table 314 may be affixed to substrate 312 at interface 326, which may be a planar or non-planar interface. Superabrasive element 310 may comprise a rear surface 318, a superabrasive face 320, and an element side surface 315. In some embodiments, element side surface 315 may include a substrate side surface 316 formed by substrate 312 and a superabrasive side surface 322 formed by superabrasive table 314. Rear surface 318 may be formed by substrate 312. Superabrasive element 310 may also comprise a chamfer 324 formed by superabrasive table 314.

According to various embodiments, a charge may be applied to superabrasive element 310 and electrode 340 through electrical conductors (e.g., wires or any suitable electrical conductor) 344 and 342, respectively. For example, in order to apply a current to a processing solution (e.g., processing solution 72 illustrated in FIG. 9C) for processing superabrasive element 310, superabrasive ele-

ment 310 and electrical conductor 344 may be positioned in the processing solution (e.g., optionally, with a leaching cup 30 or other protective covering) and a charge may be applied to at least a portion of substrate 312 (e.g., rear surface 318) of superabrasive element 310 through electrical conductor 344 and an opposite charge may be applied to electrode 340 through electrical conductor 342. In at least one embodiment, electrical conductor 344 may be electrically connected to substrate 312 by an electrode electrically connected to (e.g., positioned abutting) substrate 312. In some embodiments, electrical conductor 344 may be directly connected to superabrasive table 314 by an electrode electrically connected to (e.g., positioned abutting) superabrasive table 314.

According to at least one embodiment, at least a portion of electrode 340 may comprise a substantially annular or ring-shaped body. For example, electrode 340 may comprise a substantially annular ring surrounding a central axis (e.g., central axis 29 shown in FIGS. 1-2), as illustrated in FIGS. 11 and 12. When superabrasive element 310 and electrode 340 are disposed in a processing solution such that at least a portion of superabrasive table 314 and electrode 340 are exposed to the processing solution and a voltage is applied to the processing solution via electrode 340 and superabrasive table 314, interstitial materials may be removed from at least a portion of superabrasive table 314 of superabrasive element 310 exposed to the processing solution. In some embodiments, interstitial materials may be removed to greater depths from surface portions of superabrasive table 314 disposed in relatively closer proximity to electrode 340 than other surface portions of superabrasive table 314. Accordingly, a peripheral region of superabrasive table 314 defining chamfer 324 may be leached to a greater depth than a central region of superabrasive table 314.

FIGS. 13 and 14 illustrate a superabrasive element 410 positioned near an electrode 440 according to at least one embodiment. As illustrated in FIGS. 13 and 14, superabrasive element 410 may comprise a superabrasive table 414 affixed to or formed upon a substrate 412. Superabrasive table 414 may be affixed to substrate 412 at interface 426. Superabrasive element 410 may comprise a rear surface 418, a superabrasive face 420, and an element side surface 415. In some embodiments, element side surface 415 may include a substrate side surface 416 formed by substrate 412 and a superabrasive side surface 422 formed by superabrasive table 414. Rear surface 418 may be formed by substrate 412. Superabrasive element 410 may also comprise a chamfer 424 formed by superabrasive table 414.

According to various embodiments, a charge may be applied to superabrasive element 410 and electrode 440 through electrical conductors (e.g., wires or any suitable electrical conductor) 444 and 442, respectively. For example, in order to apply a current to a processing solution (e.g., processing solution 72 illustrated in FIG. 9C) for processing superabrasive element 410, superabrasive element 410 and electrical conductor 444 may be positioned in the processing solution (e.g., optionally, with a leaching cup 30 or other protective covering) and a charge may be applied to at least a portion of substrate 412 (e.g., rear surface 418) of superabrasive element 410 through electrical conductor 444 and an opposite charge may be applied to electrode 440 through electrical conductor 442. In at least one embodiment, electrical conductor 444 may be electrically connected to substrate 412 by an electrode electrically connected to (e.g., positioned abutting) substrate 412. In some embodiments, electrical conductor 444 may be directly connected to superabrasive table 414 by an electrode electrically connected to (e.g., positioned abutting) superabrasive table 414.

According to at least one embodiment, at least a portion of electrode 440 may comprise a disk shape. For example, electrode 440 may comprise a disk having a substantially circular outer periphery surface surrounding a central axis (e.g., central axis 29 shown in FIGS. 1-2), as illustrated in FIGS. 13 and 14. In some embodiments, electrode 440 may have an outer diameter that is smaller than the outer diameter of element side surface 415 of superabrasive element 410 and/or smaller than an inner diameter of chamfer 424. When superabrasive element 410 and electrode 440 are disposed in a processing solution such that at least a portion of superabrasive table 414 and electrode 440 are exposed to the processing solution and a voltage is applied to the processing solution via electrode 440 and superabrasive table 414, interstitial materials may be removed from at least a portion of superabrasive table 414 of superabrasive element 410 exposed to the processing solution. In some embodiments, interstitial materials may be removed to greater depths from surface portions of superabrasive table 414 disposed in relatively closer proximity to electrode 440 than other surface portions of superabrasive table 414. Accordingly, an axially central region of superabrasive table 414 may be leached to a greater depth than an outer peripheral region.

FIGS. 15-21 illustrate superabrasive elements and electrodes in cross-sectional views. The electrodes illustrated in these figures are intended to be disk-shaped and/or ring-shaped (see, e.g., electrodes 340 and 440 respectively shown in FIGS. 11 and 13).

FIG. 15 shows a cross-sectional side view of a superabrasive element 510 and an electrode 540 according to at least one embodiment. As illustrated in FIG. 15, superabrasive element 510 may comprise a superabrasive table 514 affixed to or formed upon a substrate 512. Superabrasive table 514 may be affixed to substrate 512 at interface 526. Superabrasive element 510 may comprise a rear surface 518, a superabrasive face 520, and an element side surface 515, which may include a substrate side surface 516 formed by substrate 512 and a superabrasive side surface 522 formed by superabrasive table 514. Superabrasive element 510 may also comprise a chamfer 524 formed by superabrasive table 514.

According to various embodiments, a charge may be applied to superabrasive element 510 and electrode 540 through electrical conductors (e.g., wires or any suitable electrical conductor) 544 and 542, respectively. For example, in order to apply a current to a processing solution (e.g., processing solution 72 illustrated in FIG. 9C) for processing superabrasive element 510, superabrasive element 510 and electrical conductor 544 may be positioned in the processing solution (e.g., optionally, with a leaching cup 30 or other protective covering) and a charge may be applied to at least a portion of substrate 512 (e.g., rear surface 518) of superabrasive element 510 through electrical conductor 544 and an opposite charge may be applied to electrode 540 through electrical conductor 542.

According to at least one embodiment, at least a portion of electrode 540 may comprise a substantially cylindrical shape defining a recess 546. For example, electrode 540 may comprise a substantially planar face and a substantially cylindrical outer surface, as illustrated in FIG. 15. Recess 546 may be defined within electrode 540 and may have a diameter that is greater than the outer diameter of element side surface 515 of superabrasive element 510. Electrode 540 may be disposed such that at least a portion of recess 546 surrounds at least a portion of superabrasive table 514 of superabrasive element 510, as shown in FIG. 15. When superabrasive element 510 and electrode 540 are disposed in

the processing solution such that at least a portion of superabrasive table 514 and electrode 540 are exposed to the processing solution and a voltage is applied to the processing solution via electrode 540 and superabrasive table 514, interstitial materials may be removed from at least a portion of superabrasive table 514 exposed to the processing solution.

FIG. 16 shows a cross-sectional side view of a superabrasive element 610 positioned near an electrode 640 according to at least one embodiment. As illustrated in FIG. 16, superabrasive element 610 may comprise a superabrasive table 614 affixed to or formed upon a substrate 612. Superabrasive table 614 may be affixed to substrate 612 at interface 626. Superabrasive element 610 may comprise a rear surface 618, a superabrasive face 620, and an element side surface 615, which may include a substrate side surface 616 formed by substrate 612 and a superabrasive side surface 622 formed by superabrasive table 614. Superabrasive element 610 may also comprise a chamfer 624 formed by superabrasive table 614.

According to various embodiments, a charge may be applied to superabrasive element 610 and electrode 640 through electrical conductors (e.g., wires or any suitable electrical conductor) 644 and 642, respectively. For example, in order to apply a current to a processing solution (e.g., processing solution 72 illustrated in FIG. 9C) for processing superabrasive element 610, superabrasive element 610 and electrical conductor 644 may be positioned in the processing solution (e.g., optionally, with a leaching cup 30 or other protective covering) and a charge may be applied to at least a portion of substrate 612 (e.g., rear surface 618) of superabrasive element 610 through electrical conductor 644 and an opposite charge may be applied to electrode 640 through electrical conductor 642.

According to at least one embodiment, at least a portion of electrode 640 may comprise a substantially cylindrical shape defining a recess 646. For example, electrode 640 may comprise a substantially planar face and a substantially cylindrical outer surface, as illustrated in FIG. 16. Recess 646 may be defined within electrode 640 and may have a diameter that is substantially the same as or smaller than the outer diameter of element side surface 615 of superabrasive element 610. When superabrasive element 610 and electrode 640 are disposed in the processing solution such that at least a portion of superabrasive table 614 and electrode 640 are exposed to the processing solution and a voltage is applied to the processing solution via electrode 640 and superabrasive table 614, interstitial materials may be removed from at least a portion of superabrasive table 614 of superabrasive element 610 exposed to the processing solution.

FIG. 17 shows a cross-sectional side view of a superabrasive element 710 positioned near an electrode 740 according to at least one embodiment. As illustrated in FIG. 17, superabrasive element 710 may comprise a superabrasive table 714 affixed to or formed upon a substrate 712. Superabrasive table 714 may be affixed to substrate 712 at interface 726. Superabrasive element 710 may comprise a rear surface 718, a superabrasive face 720, and an element side surface 715, which may include a substrate side surface 716 formed by substrate 712 and a superabrasive side surface 722 formed by superabrasive table 714. Superabrasive element 710 may also comprise a chamfer 724 formed by superabrasive table 714.

According to various embodiments, a charge may be applied to superabrasive element 710 and electrode 740 through electrical conductors (e.g., wires or any suitable electrical conductor) 744 and 742, respectively. For

example, in order to apply a current to a processing solution (e.g., processing solution 72 illustrated in FIG. 9C) for processing superabrasive element 710, superabrasive element 710 and electrical conductor 744 may be positioned in the processing solution (e.g., optionally, with a leaching cup 30 or other protective covering) and a charge may be applied to at least a portion of substrate 712 (e.g., rear surface 718) of superabrasive element 710 through electrical conductor 744 and an opposite charge may be applied to electrode 740 through electrical conductor 742.

According to at least one embodiment, at least a portion of electrode 740 may comprise a substantially cylindrical shape with a peripheral recess 748 defined therein and extending circumferentially around at least a peripheral portion of electrode 740. For example, peripheral recess 748 may be defined between a face of electrode 740 located nearest superabrasive element 710 and an outer peripheral surface of electrode 740, as illustrated in FIG. 17. When superabrasive element 710 and electrode 740 are disposed in a processing solution such that at least a portion of superabrasive table 714 and electrode 740 are exposed to the processing solution and a voltage is applied to the processing solution via electrode 740 and superabrasive table 714, interstitial materials may be removed from at least a portion of superabrasive table 714 of superabrasive element 710 exposed to the processing solution.

FIG. 18 shows a cross-sectional side view of a superabrasive element 810 and an electrode 840 according to at least one embodiment. As illustrated in FIG. 18, superabrasive element 810 may comprise a superabrasive table 814 affixed to or formed upon a substrate 812. Superabrasive table 814 may be affixed to substrate 812 at interface 826. Superabrasive element 810 may comprise a rear surface 818, a superabrasive face 820, and an element side surface 815, which may include a substrate side surface 816 formed by substrate 812 and a superabrasive side surface 822 formed by superabrasive table 814. Superabrasive element 810 may also comprise a chamfer 824 formed by superabrasive table 814.

According to various embodiments, a charge may be applied to superabrasive element 810 and electrode 840 through electrical conductors (e.g., wires or any suitable electrical conductor) 844 and 842, respectively. For example, in order to apply a current to a processing solution (e.g., processing solution 72 illustrated in FIG. 9C) for processing superabrasive element 810, superabrasive element 810 and electrical conductor 844 may be positioned in the processing solution (e.g., optionally, with a leaching cup 30 or other protective covering) and a charge may be applied to at least a portion of substrate 812 (e.g., rear surface 818) of superabrasive element 810 through electrical conductor 844 and an opposite charge may be applied to electrode 840 through electrical conductor 842.

Electrode 840 may be annular or ring-shaped and electrical conductor 842 may be electrically connected to electrode 840 at one or more locations. For example, electrode 840 may comprise sections or portions of an annular or ring-shaped body, and electrical conductor 842 may be electrically connected to each section. In at least one embodiment, electrical conductor 844 may be electrically connected to substrate 812 by an electrode electrically connected to (e.g., positioned abutting) substrate 812. In some embodiments, electrical conductor 844 may be directly connected to superabrasive table 814 by an electrode electrically connected to (e.g., positioned abutting) superabrasive table 814.

According to at least one embodiment, at least a portion of electrode 840 may comprise a substantially tilted annular or ring-shaped body. For example, electrode 840 may comprise an annular ring surrounding a central axis (e.g., central axis 29 shown in FIGS. 1-2) and tilted at an angle, as illustrated in FIG. 18. Electrode 840 may be disposed in a position such that at least a portion of electrode 840 surrounds at least a portion of superabrasive table 814 of superabrasive element 810, such as chamfer 824, as shown in FIG. 18. In some embodiments, electrode 840 may be tilted at substantially the same angle as chamfer 824. When superabrasive element 810 and electrode 840 are disposed in the processing solution such that at least a portion of superabrasive table 814 and electrode 840 are exposed to the processing solution and a voltage is applied to the processing solution via electrode 840 and superabrasive table 814, interstitial materials may be removed from at least a portion of superabrasive table 814 of superabrasive element 810 exposed to the processing solution. In some embodiments, interstitial materials may be removed to greater depths from surface portions of superabrasive table 814 disposed in relatively closer proximity to electrode 840 than other surface portions of superabrasive table 814. Accordingly, a peripheral region of superabrasive table 814 defining chamfer 824 may be leached to a greater depth than a central region of superabrasive table 814.

FIG. 19 shows a cross-sectional side view of a superabrasive element 910 and an electrode 940 according to at least one embodiment. As illustrated in FIG. 19, superabrasive element 910 may comprise a superabrasive table 914 affixed to or formed upon a substrate 912. Superabrasive table 914 may be affixed to substrate 912 at interface 926. Superabrasive element 910 may comprise a rear surface 918, a superabrasive face 920, and an element side surface 915, which may include a substrate side surface 916 formed by substrate 912 and a superabrasive side surface 922 formed by superabrasive table 914. Superabrasive element 910 may also comprise a chamfer 924 formed by superabrasive table 914.

According to various embodiments, a charge may be applied to superabrasive element 910 and electrode 940 through electrical conductors (e.g., wires or any suitable electrical conductor) 944 and 942, respectively. For example, in order to apply a current to a processing solution (e.g., processing solution 72 illustrated in FIG. 9C) for processing superabrasive element 910, superabrasive element 910 and electrical conductor 944 may be positioned in the processing solution (e.g., optionally, with a leaching cup 30 or other protective covering) and a charge may be applied to at least a portion of substrate 912 (e.g., rear surface 918) of superabrasive element 910 through electrical conductor 944 and an opposite charge may be applied to electrode 940 through electrical conductor 942.

Electrode 940 may be annular or ring-shaped and electrical conductor 942 may be electrically connected to electrode 940 at one or more locations. For example, electrode 940 may comprise sections or portions of an annular or ring-shaped body, and electrical conductor 942 may be electrically connected to each section. In at least one embodiment, electrical conductor 944 may be electrically connected to substrate 912 by an electrode electrically connected to (e.g., positioned abutting) substrate 912. In some embodiments, electrical conductor 944 may be directly connected to superabrasive table 914 by an electrode electrically connected to (e.g., positioned abutting) superabrasive table 914.

According to at least one embodiment, at least a portion of electrode 940 may comprise a substantially annular or ring-shaped body. For example, electrode 940 may comprise a substantially annular ring surrounding a central axis (e.g., central axis 29 shown in FIGS. 1-2), as illustrated in FIG. 19. In at least one embodiment, electrode 940 may have an inner diameter that is greater than the outer diameter of element side surface 915 of superabrasive element 910. Electrode 940 may be disposed in a position such that at least a portion of electrode 940 surrounds at least a portion of superabrasive table 914 of superabrasive element 910, as shown in FIG. 19. When superabrasive element 910 and electrode 940 are disposed in the processing solution such that at least a portion of superabrasive table 914 and electrode 940 are exposed to the processing solution and a voltage is applied to the processing solution via electrode 940 and superabrasive table 914, interstitial materials may be removed from at least a portion of superabrasive table 914 of superabrasive element 910 exposed to the processing solution. In some embodiments, interstitial materials may be removed to greater depths from surface portions of superabrasive table 914 disposed in relatively closer proximity to electrode 940 than other surface portions of superabrasive table 914. Accordingly, a peripheral region of superabrasive table 914 defining chamfer 924 and/or superabrasive side surface 922 may be leached to a greater depth than a central region of superabrasive table 914.

FIG. 20 shows a cross-sectional side view of a superabrasive element 1010 and an electrode 1040 according to at least one embodiment. As illustrated in FIG. 20, superabrasive element 1010 may comprise a superabrasive table 1014 affixed to or formed upon a substrate 1012. Superabrasive table 1014 may be affixed to substrate 1012 at interface 1026. Superabrasive element 1010 may comprise a rear surface 1018, a superabrasive face 1020, and an element side surface 1015, which may include a substrate side surface 1016 formed by substrate 1012 and a superabrasive side surface 1022 formed by superabrasive table 1014. Superabrasive element 1010 may also comprise a chamfer 1024 formed by superabrasive table 1014.

According to various embodiments, a charge may be applied to superabrasive element 1010 and electrode 1040 through electrical conductors (e.g., wires or any suitable electrical conductor) 1044 and 1042, respectively. For example, in order to apply a current to a processing solution (e.g., processing solution 72 illustrated in FIG. 9C) for processing superabrasive element 1010, superabrasive element 1010 and electrical conductor 1044 may be positioned in the processing solution (e.g., optionally, with a leaching cup 30 or other protective covering) and a charge may be applied to at least a portion of substrate 1012 (e.g., rear surface 1018) of superabrasive element 1010 through electrical conductor 1044 and an opposite charge may be applied to electrode 1040 through electrical conductor 1042.

Electrode 1040 may be annular or ring-shaped and electrical conductor 1042 may be electrically connected to electrode 1040 at one or more locations. For example, electrode 1040 may comprise sections or portions of an annular or ring-shaped body, and electrical conductor 1042 may be electrically connected to each section. In at least one embodiment, electrical conductor 1044 may be electrically connected to substrate 1012 by an electrode electrically connected to (e.g., positioned abutting) substrate 1012. In some embodiments, electrical conductor 1044 may be directly connected to superabrasive table 1014 by an electrode electrically connected to (e.g., positioned abutting) superabrasive table 1014.

According to at least one embodiment, at least a portion of electrode **1040** may comprise a substantially annular or ring-shaped body and may define a recess **1046**, as illustrated in FIG. 20. In at least one embodiment, a surface of electrode **1040** defining recess **1046** may have a diameter that is greater than the outer diameter of element side surface **1015** of superabrasive element **1010**. Electrode **1040** may be disposed in a position such that at least a portion of recess **1046** surrounds at least a portion of superabrasive table **1014** of superabrasive element **1010**, as shown in FIG. 20. When superabrasive element **1010** and electrode **1040** are disposed in the processing solution such that at least a portion of superabrasive table **1014** and electrode **1040** are exposed to the processing solution and a voltage is applied to the processing solution via electrode **1040** and superabrasive table **1014**, interstitial materials may be removed from at least a portion of superabrasive table **1014** of superabrasive element **1010** exposed to the processing solution. In some embodiments, interstitial materials may be removed to greater depths from surface portions of superabrasive table **1014** disposed in relatively closer proximity to electrode **1040** than other surface portions of superabrasive table **1014**. Accordingly, a peripheral region of superabrasive table **1014** defining chamfer **1024** and/or superabrasive side surface **1022** may be leached to a greater depth than a central region of superabrasive table **1014**.

FIG. 21 shows a cross-sectional side view of a superabrasive element **1110** and an electrode assembly **1140** comprising a first electrode **1141** and a second electrode **1143** according to at least one embodiment. As illustrated in FIG. 21, superabrasive element **1110** may comprise a superabrasive table **1114** affixed to or formed upon a substrate **1112**. Superabrasive table **1114** may be affixed to substrate **1112** at interface **1126**. Superabrasive element **1110** may comprise a rear surface **1118**, a superabrasive face **1120**, and an element side surface **1115**, which may include a substrate side surface **1116** formed by substrate **1112** and a superabrasive side surface **1122** formed by superabrasive table **1114**. Superabrasive element **1110** may also comprise a chamfer **1124** formed by superabrasive table **1114**.

According to various embodiments, a charge may be applied to superabrasive element **1110** and electrode assembly **1140** through electrical conductors (e.g., wires or any suitable electrical conductor) **1144** and **1142**, respectively. For example, in order to apply a current to a processing solution (e.g., processing solution **72** illustrated in FIG. 9C) for processing superabrasive element **1110**, superabrasive element **1110** and electrical conductor **1144** may be positioned in the processing solution (e.g., optionally, with a leaching cup **30** or other protective covering) and a charge may be applied to at least a portion of substrate **1112** (e.g., rear surface **1118**) of superabrasive element **1110** through electrical conductor **1144** and an opposite charge may be applied to electrode assembly **1140** through electrical conductor **1142**.

At least a portion of electrode assembly **1140** may be annular or ring-shaped and electrical conductor **1142** may be electrically connected to electrode assembly **1140** at one or more locations. For example, second electrode **1143** may comprise sections or portions of an annular or ring-shaped body, and electrical conductor **1142** may be electrically connected to each section. In at least one embodiment, electrical conductor **1144** may be electrically connected to substrate **1112** by an electrode electrically connected to (e.g., positioned abutting) substrate **1112**. In some embodiments, electrical conductor **1144** may be directly connected to

superabrasive table **1114** by an electrode electrically connected to (e.g., positioned abutting) superabrasive table **1114**.

According to at least one embodiment, first electrode **1141** may comprise a disk-shaped electrode positioned near superabrasive face **1120** of superabrasive table **1114**. Second electrode **1143** may comprise a substantially annular or ring-shaped body with an inner diameter that is greater than an outer diameter of element side surface **1115** of superabrasive element **1110**. Second electrode **1143** of electrode assembly **1140** may be disposed in a position such that at least a portion of second electrode **1143** surrounds at least a portion of superabrasive table **1114** of superabrasive element **1110**, as shown in FIG. 21. When superabrasive element **1110** and electrode assembly **1140** are disposed in the processing solution such that at least a portion of superabrasive table **1114**, first electrode **1141**, and second electrode **1143** are exposed to the processing solution and a voltage is applied to the processing solution via electrode assembly **1140** and superabrasive table **1114**, interstitial materials may be removed from at least a portion of superabrasive table **1114** of superabrasive element **1110** exposed to the processing solution. In some embodiments, interstitial materials may be removed to greater depths from surface portions of superabrasive table **1114** disposed in relatively closer proximity to first electrode **1141** and/or second electrode **1143** of electrode assembly **1140** than other surface portions of superabrasive table **1114**.

FIG. 22 shows a cross-sectional side view of a superabrasive element **1210** and electrodes **1240** and **1249** according to at least one embodiment. As illustrated in FIG. 22, superabrasive element **1210** may comprise a superabrasive table **1214** affixed to or formed upon a substrate **1212**. Superabrasive table **1214** may be affixed to substrate **1212** at interface **1226**. Superabrasive element **1210** may comprise a rear surface **1218**, a superabrasive face **1220**, and an element side surface **1215**, which may include a substrate side surface **1216** formed by substrate **1212** and a superabrasive side surface **1222** formed by superabrasive table **1214**. Superabrasive element **1210** may also comprise a chamfer **1224** formed by superabrasive table **1214**.

As shown in FIG. 22, electrode **1249** may be disposed adjacent to at least portion of superabrasive table **1214**. For example, electrode **1249** may be electrically connected to (e.g., positioned abutting) superabrasive face **1220** and/or any other suitable surface of superabrasive table **1214**. According to various embodiments, a charge may be applied to electrode **1240** and electrode **1249**, and likewise to superabrasive table **1214**, through electrical conductors (e.g., wires or any suitable electrical conductor) **1242** and **1244**, respectively. For example, in order to apply a current to a processing solution (e.g., processing solution **72** illustrated in FIG. 9C) for processing superabrasive element **1210**, superabrasive element **1210** and electrode **1249** may be positioned in the processing solution (e.g., optionally, with a leaching cup **30** or other protective covering) and a charge may be applied to at least a portion of superabrasive table **1214** through electrical conductor **1244** and electrode **1249**, and an opposite charge may be applied to electrode **1240** through electrical conductor **1242**.

According to at least one embodiment, electrode **1249** may comprise a disk-shaped electrode. In some embodiments, superabrasive table **1214** may be coupled to electrode **1249** through brazing, welding, soldering, adhesive bonding, mechanical fastening, and/or any other suitable bonding technique. For example, superabrasive table **1214** may be bonded to electrode **1249** by a braze joint (e.g., a carbide

forming braze such as a titanium-based braze, etc.). In at least one embodiment, such a braze joint may be coated with a protective layer (e.g., paint layer, epoxy layer, etc.).

At least a portion of electrode 1240 may be annular or ring-shaped and electrical conductor 1242 may be electrically connected to electrode 1240 at one or more locations. For example, electrode 1240 may comprise sections or portions of an annular or ring-shaped body, and electrical conductor 1242 may be electrically connected to each section. Electrode 1240 may be disposed in a position such that at least a portion of electrode 1240 surrounds at least a portion of superabrasive table 1214 of superabrasive element 1210, as shown in FIG. 22. When superabrasive element 1210 and electrode 1240 are disposed in the processing solution such that at least a portion of superabrasive table 1214 and electrode 1240 are exposed to the processing solution and a voltage is applied to the processing solution via electrode 1240, electrode 1249, and/or superabrasive table 1214, interstitial materials may be removed from at least a portion of superabrasive table 1214 exposed to the processing solution. In some embodiments, interstitial materials may be removed to greater depths from surface portions of superabrasive table 1214 disposed in relatively closer proximity to electrode 1240 than other surface portions of superabrasive table 1214.

FIGS. 23A and 23B show a superabrasive element 1310 coated with masking layers and disposed near an electrode 1340. According to various embodiments, portions of superabrasive element 1310 may be coated or otherwise covered with one or more masking layers that prevent and/or delay a leaching agent from contacting selected regions of superabrasive element 1310 during leaching. For example, a first masking layer 1333 and a second masking layer 1335 may be formed on or disposed abutting at least a portion of superabrasive element 1310.

As illustrated in FIGS. 23A and 23B, superabrasive element 1310 may comprise a superabrasive table 1314 affixed to or formed upon a substrate 1312. Superabrasive table 1314 may be affixed to substrate 1312 at interface 1326. Superabrasive element 1310 may comprise a rear surface 1318, a superabrasive face 1320, and an element side surface 1315, which may include a substrate side surface 1316 formed by substrate 1312 and a superabrasive side surface 1322 formed by superabrasive table 1314. Superabrasive element 1310 may also comprise a chamfer 1324 formed by superabrasive table 1314.

As shown in FIGS. 23A and 23B, first masking layer 1333 may be disposed on at least a portion of superabrasive face 1320, such as a central portion of superabrasive face 1320 surrounding a central axis (e.g., central axis 29 shown in FIGS. 1-2). Second masking layer 1335 may be disposed on at least a portion of element side surface 1315 and rear surface 1318 of superabrasive element 1310 so as to surround at least a portion of superabrasive table 1314 and/or substrate 1312. First masking layer 1333 and second masking layer 1335 may prevent damage to selected portions of superabrasive element 1310 and may provide a desired leach profile when superabrasive element 1310 is exposed to various leaching agents. For example, first masking layer 1333 and/or second masking layer 1335 may prevent or delay a leaching solution from contacting certain portions of superabrasive element 1310, such as portions of substrate 1312, portions of superabrasive table 1314, or both, during leaching.

In various examples, first masking layer 1333 and/or second masking layer 1335 may comprise one or more materials that are substantially inert and/or otherwise resis-

tant and/or impermeable to acids, bases, and/or other reactive compounds present in a leaching solution used to leach superabrasive element 1310. Optionally, first masking layer 1333 and/or second masking layer 1335 may comprise a material that breaks down or degrades in the presence of a leaching agent, such as a material that is at least partially degraded (e.g., at least partially dissolved) at a selected rate during exposure to the leaching agent.

In some embodiments, first masking layer 1333 and/or second masking layer 1335 may comprise one or more materials exhibiting significant stability during exposure to a leaching agent. According to various embodiments, first masking layer 1333 and second masking layer 1335 may comprise any suitable material, including metals, alloys, polymers, carbon allotropes, oxides, carbides, glass materials, ceramics, composites, membrane materials (e.g. permeable or semi-permeable materials), and/or any combination of the foregoing, without limitation. First masking layer 1333 and second masking layer 1335 may be affixed to superabrasive element 1310 through any suitable mechanism, without limitation, including, for example, direct bonding, bonding via an intermediate layer, such as an adhesive or braze joint, mechanical attachment, such as mechanical fastening, frictional attachment, and/or interference fitting. In some embodiments, first masking layer 1333 and/or second masking layer 1335 may comprise a coating or layer of material that is formed on or otherwise adhered to at least a portion of superabrasive element 1310. In additional embodiments, first masking layer 1333 and/or second masking layer 1335 may comprise a material that is temporarily fixed to superabrasive element 1310. For example, first masking layer 1333 may comprise a polymer member (e.g., o-ring, gasket, disk) that is mechanically held in place (e.g., by clamping) during exposure to a leaching agent.

First masking layer 1333 and second masking layer 1335 may be formed over any suitable portions superabrasive element 1310. For example, as illustrated in FIGS. 23A and 23B, first masking layer 1333 may be formed over a central portion of superabrasive face 1320 about a central axis (e.g., central axis 29 shown in FIGS. 1-2). First masking layer 1333 may be separated from chamfer 1324. For example, first masking layer 1333 may not be directly adjacent to and/or in contact with edge 1327 formed at the intersection of superabrasive face 1320 and chamfer 1324. Second masking layer 1335 may be formed over at least a portion of substrate 1312 and superabrasive table 1314. For example, as shown in FIGS. 23A and 23B, second masking layer 1335 may be formed over rear surface 1318 and substrate side surface 1316 of substrate 1312 so as to substantially surround substrate 1312. Optionally, second masking layer 1335 may be formed over a portion of superabrasive side surface 1322. In some embodiments, second masking layer 1335 may also be separated from chamfer 1324. For example, second masking layer 1335 may not be directly adjacent to and/or in contact with edge 1328 formed at the intersection of superabrasive side surface 1322 and chamfer 1324.

According to various embodiments, a charge may be applied to superabrasive element 1310 and electrode 1340 through electrical conductors (e.g., wires or any suitable electrical conductor) 1344 and 1342, respectively. For example, in order to apply a current to a processing solution (e.g., processing solution 72 illustrated in FIG. 9C) for processing superabrasive element 1310, superabrasive element 1310 and electrical conductor 1344 may be positioned in the processing solution (e.g., optionally, with a leaching

cup 30 or other protective covering) and a charge may be applied to at least a portion of substrate 1312 (e.g., rear surface 1318) of superabrasive element 1310 through electrical conductor 1344 and an opposite charge may be applied to electrode 1340 through electrical conductor 1342. In at least one embodiment, electrical conductor 1344 may be electrically connected to substrate 1312 by an electrode electrically connected to (e.g., positioned abutting) substrate 1312. In some embodiments, electrical conductor 1344 may be directly connected to superabrasive table 1314 by an electrode electrically connected to (e.g., positioned abutting) superabrasive table 1314.

Electrode 1340 may comprise any suitable size, shape, and/or geometry, without limitation. In some embodiments, electrode 1340 may comprise a circular or non-circular disk shape. For example, electrode 1340 may have a substantially circular outer periphery surrounding a central axis (e.g., central axis 29 shown in FIGS. 1-2). Electrode 1340 may have an outer diameter that is larger than, the same as, or smaller than the outer diameter of element side surface 1315 of superabrasive element 1310, as shown in FIGS. 23A and 23B. Electrodes and/or combinations of electrodes according to any of the configurations disclosed herein may also be utilized in addition to or in place of electrode 1340 for processing superabrasive element 1310. When superabrasive element 1310 and electrode 1340 are disposed in the processing solution (e.g., processing solution 72 as shown in FIG. 9C) such that at least a portion of superabrasive table 1314 and electrode 1340 are exposed to the processing solution and a voltage is applied to the processing solution via electrode 1340 and superabrasive table 1314, interstitial materials may be removed from at least a portion of superabrasive table 1314 of superabrasive element 1310 exposed to the processing solution and disposed near electrode 1340.

The configuration illustrated in FIGS. 23A and 23B may enable selective leaching of portions of superabrasive element 1310 to form a desired leach profile within superabrasive table 1314. For example, a volume of superabrasive table 1314 adjacent to an uncovered region between first masking layer 1333 and second masking layer 1335 may be leached to a greater depth than surrounding portions of superabrasive table 1314 covered by first masking layer 1333 and second masking layer 1335. The configurations illustrated in FIGS. 23A and 23B may result in the formation of leached volumes in portions of superabrasive table 1314 located near chamfer 1324 during leaching. In some embodiments, the leached volumes may extend from chamfer 1324 to a region adjacent to and/or abutting interface 1326.

Following exposure to a leaching solution, first masking layer 1333 and/or second masking layer 1335 may be substantially removed from superabrasive table 1314 and/or substrate 1312 using any suitable technique, including, for example, lapping, grinding, and/or removal using suitable chemical agents. According to certain embodiments, first masking layer 1333 and/or second masking layer 1335 may be peeled, cut, ground, lapped, and/or otherwise physically, thermally, or chemically removed from superabrasive element 1310. In some embodiments, following or during removal of first masking layer 1333 and/or second masking layer 1335, one or more surfaces of superabrasive table 1314 and/or substrate 1312 may be processed to form a desired surface texture and/or finish using any suitable technique, including, for example, lapping, grinding, and/or otherwise physically and/or chemically treating the one or more surfaces.

FIGS. 24 and 25 illustrate masking layers formed over portions of a superabrasive element 1410 having an edge 1417 formed at the intersection of superabrasive face 1420 and superabrasive side surface 1422. As illustrated, for example, in FIG. 24, first masking layer 1433 may be formed over a central portion of superabrasive face 1420 about a central axis (e.g., central axis 29 shown in FIGS. 1-2). First masking layer 1433 may not be directly adjacent to and/or in contact with edge 1417. In additional embodiments, first masking layer 1433 may be formed adjacent to and/or in contact with edge 1417. Second masking layer 1435 may be formed over at least a portion of substrate 1412 and superabrasive table 1414. For example, as shown in FIG. 24, second masking layer 1435 may be formed over rear surface 1418 and substrate side surface 1416 of substrate 1412 so as to substantially surround substrate 1412. Optionally, second masking layer 1435 may be formed over a portion of superabrasive side surface 1422, such as extending from the substrate longitudinally past interface 1426 between substrate 1412 and superabrasive element 1410. In some embodiments, second masking layer 1435 may not be directly adjacent to and/or in contact with edge 1417, as shown in FIG. 24.

According to various embodiments, a charge may be applied to superabrasive element 1410 and electrode 1440 through electrical conductors (e.g., wires or any suitable electrical conductor) 1444 and 1442, respectively. For example, in order to apply a current to a processing solution (e.g., processing solution 72 illustrated in FIG. 9C) for processing superabrasive element 1410, superabrasive element 1410 and electrical conductor 1444 may be positioned in the processing solution (e.g., optionally, with a leaching cup 30 or other protective covering) and a charge may be applied to at least a portion of substrate 1412 (e.g., rear surface 1418) of superabrasive element 1410 through electrical conductor 1444 and an opposite charge may be applied to electrode 1440 through electrical conductor 1442. In at least one embodiment, electrical conductor 1444 may be electrically connected to substrate 1412 by an electrode electrically connected to (e.g., positioned abutting) substrate 1412. In some embodiments, electrical conductor 1444 may be directly connected to superabrasive table 1414 by an electrode electrically connected to (e.g., positioned abutting) superabrasive table 1414.

Electrode 1440 may comprise any suitable size, shape, and/or geometry, without limitation. In some embodiments, electrode 1440 may comprise a circular or non-circular disk shape. For example, electrode 1440 may have a substantially circular outer periphery surrounding a central axis (e.g., central axis 29 shown in FIGS. 1-2). Electrode 1440 may have an outer diameter that is larger than, the same as, or smaller than the outer diameter of element side surface 1415 of superabrasive element 1410, as shown in FIG. 24. Electrodes according to any of the configurations disclosed herein may also be utilized in addition to or in place of electrode 1440 for processing superabrasive element 1410. When superabrasive element 1410 and electrode 1440 are disposed in the processing solution such that at least a portion of superabrasive table 1414 and electrode 1440 are exposed to the processing solution and a voltage is applied to the processing solution via electrode 1440 and superabrasive table 1414, interstitial materials may be removed from at least a portion of superabrasive table 1414 of superabrasive element 1410 exposed to the processing solution and disposed near electrode 1440.

FIG. 25 illustrates masking layers formed over portions of a superabrasive element 1410 having an edge 1417 formed

at the intersection of superabrasive face 1420 and superabrasive side surface 1422. As illustrated, for example, in FIG. 25, first masking layer 1433 may be formed over a central portion of superabrasive face 1420 about a central axis (e.g., central axis 29 shown in FIGS. 1-2). First masking layer 1433 may not be directly adjacent to and/or in contact with edge 1417. In additional embodiments, first masking layer 1433 may be formed adjacent to and/or in contact with edge 1417. Second masking layer 1435 may be formed over at least a portion of substrate 1412 and superabrasive table 1414. For example, as shown in FIG. 25, second masking layer 1435 may be formed over rear surface 1418 and substrate side surface 1416 of substrate 1412 so as to substantially surround substrate 1412. Optionally, second masking layer 1435 may be formed over at least a portion of superabrasive side surface 1422, such as extending from substrate 1410 longitudinally past interface 1426 between substrate 1412 and superabrasive element 1410. In some embodiments, second masking layer 1435 may be disposed adjacent to and/or in contact with edge 1417, as shown in FIG. 25.

According to various embodiments, a charge may be applied to superabrasive element 1410 and electrode 1440 through electrical conductors (e.g., wires or any suitable electrical conductor) 1444 and 1442, respectively. For example, in order to apply a current to a processing solution (e.g., processing solution 72 illustrated in FIG. 9C) for processing superabrasive element 1410, superabrasive element 1410 and electrical conductor 1444 may be positioned in the processing solution (e.g., optionally, with a leaching cup 30 or other protective covering) and a charge may be applied to at least a portion of substrate 1412 (e.g., rear surface 1418) of superabrasive element 1410 through electrical conductor 1444 and an opposite charge may be applied to electrode 1440 through electrical conductor 1442. In at least one embodiment, electrical conductor 1444 may be electrically connected to substrate 1412 by an electrode electrically connected to (e.g., positioned abutting) substrate 1412. In some embodiments, electrical conductor 1444 may be directly connected to superabrasive table 1414 by an electrode electrically connected to (e.g., positioned abutting) superabrasive table 1414.

Electrode 1440 may comprise any suitable size, shape, and/or geometry, without limitation. In some embodiments, electrode 1440 may comprise a circular or non-circular disk shape. For example, electrode 1440 may have a substantially circular outer periphery surrounding a central axis (e.g., central axis 29 shown in FIGS. 1-2). Electrode 1440 may have an outer diameter that is larger than, the same as, or smaller than the outer diameter of element side surface 1415 of superabrasive element 1410, as shown in FIG. 25. When superabrasive element 1410 and electrode 1440 are disposed in the processing solution such that at least a portion of superabrasive table 1414 and electrode 1440 are exposed to the processing solution and a voltage is applied to the processing solution via electrode 1440 and superabrasive table 1414, interstitial materials may be removed from at least a portion of superabrasive table 1414 of superabrasive element 1410 exposed to the processing solution and disposed near electrode 1440.

FIG. 26 shows a superabrasive element 1510 coated with masking layers and disposed near an electrode 1540. According to various embodiments, portions of superabrasive element 1510 may be coated or otherwise covered with one or more masking layers that prevent and/or delay a leaching agent from contacting selected regions of superabrasive element 1510 during leaching. For example, a first

masking layer 1533 and, optionally, a second masking layer 1535 may be formed on or disposed abutting at least a portion of superabrasive element 1510.

Superabrasive element 1510 may comprise a superabrasive table 1514 affixed to or formed upon a substrate 1512. Superabrasive table 1514 may be affixed to substrate 1512 at interface 1526. Superabrasive element 1510 may comprise a rear surface 1518, a superabrasive face 1520, and an element side surface 1515, which may include a substrate side surface 1516 formed by substrate 1512 and a superabrasive side surface 1522 formed by superabrasive table 1514. Superabrasive element 1510 may also comprise a chamfer 1524 formed by superabrasive table 1514.

According to some embodiments, first masking layer 1533 and/or second masking layer 1535 may be disposed adjacent to and/or in contact with at least a portion of chamfer 1524. For example, as illustrated in FIG. 26, first masking layer 1533 may substantially cover superabrasive face 1520 such that first masking layer 1533 is formed adjacent to edge 1527 of superabrasive table 1514. Optionally, second masking layer 1535 may substantially cover superabrasive side surface 1522 such that second masking layer 1535 is formed adjacent to edge 1528 of superabrasive table 1514. In some embodiments, first masking layer 1533 and/or second masking layer 1535 may be formed over at least a portion of chamfer 1524.

According to various embodiments, a charge may be applied to superabrasive element 1510 and electrode 1540 through electrical conductors (e.g., wires or any suitable electrical conductor) 1544 and 1542, respectively. For example, in order to apply a current to a processing solution (e.g., processing solution 72 illustrated in FIG. 9C) for processing superabrasive element 1510, superabrasive element 1510 and electrical conductor 1544 may be positioned in the processing solution (e.g., optionally, with a leaching cup 30 or other protective covering) and a charge may be applied to at least a portion of substrate 1512 (e.g., rear surface 1518) of superabrasive element 1510 through electrical conductor 1544 and an opposite charge may be applied to electrode 1540 through electrical conductor 1542. In at least one embodiment, electrical conductor 1544 may be electrically connected to substrate 1512 by an electrode electrically connected to (e.g., positioned abutting) substrate 1512. In some embodiments, electrical conductor 1544 may be directly connected to superabrasive table 1514 by an electrode electrically connected to (e.g., positioned abutting) superabrasive table 1514.

Electrode 1540 may comprise any suitable size, shape, and/or geometry, without limitation. In some embodiments, electrode 1540 may comprise a circular or non-circular disk shape. For example, electrode 1540 may have a substantially circular outer periphery surrounding a central axis (e.g., central axis 29 shown in FIGS. 1-2). Electrode 1540 may have an outer diameter that is larger than, the same as, or smaller than the outer diameter of element side surface 1515 of superabrasive element 1510, as shown in FIG. 27. When superabrasive element 1510 and electrode 1540 are disposed in the processing solution such that at least a portion of superabrasive table 1514 and electrode 1540 are exposed to the processing solution and a voltage is applied to the processing solution via electrode 1540 and superabrasive table 1514, interstitial materials may be removed from at least a portion of superabrasive table 1514 of superabrasive element 1510 exposed to the processing solution and disposed near electrode 1540. Accordingly, a peripheral region

of superabrasive table 1514 defining chamfer 1524 may be leached to a greater depth than a central region of superabrasive table 1514.

FIG. 27 is a cross-sectional side view of a superabrasive element 1610 coated with masking layers according to at least one embodiment. As shown in FIG. 27, superabrasive element 1610 may be coated with various masking layers that prevent and/or delay a leaching agent from contacting selected regions of superabrasive element 1610 during leaching. According to some embodiments, a first protective masking layer 1633 and a second protective masking layer 1635 may be formed on at least a portion of superabrasive element 1610. Optionally, a first at-least-partially-degrading masking layer 1637 and a second at-least-partially-degrading masking layer 1647 may be formed on at least a portion of superabrasive element 1610.

As illustrated in FIG. 27, superabrasive element 1610 may comprise a superabrasive table 1614 affixed to or formed upon a substrate 1612. Superabrasive table 1614 may be affixed to substrate 1612 at interface 1626. Superabrasive element 1610 may comprise a rear surface 1618, a superabrasive face 1620, and an element side surface 1615, which may include a substrate side surface 1616 formed by substrate 1612 and a superabrasive side surface 1622 formed by superabrasive table 1614. Superabrasive element 1610 may also comprise a chamfer 1624 formed by superabrasive table 1614.

As shown in FIG. 27, first protective masking layer 1633 may be formed on at least a portion of superabrasive face 1620, such as a central portion of superabrasive face 1620 surrounding a central axis (e.g., central axis 29 shown in FIGS. 1-2). Second protective masking layer 1635 may be formed on at least a portion of element side surface 1615 and rear surface 1618 of superabrasive element 1610 so as to surround at least a portion of superabrasive table 1614 and/or substrate 1612. For example, as illustrated in FIG. 27, first masking layer 1633 may substantially cover at least a portion of superabrasive face 1620 such that first masking layer 1633 is formed adjacent to edge 1627 of superabrasive table 1614. Optionally, second masking layer 1635 may substantially cover at least a portion of superabrasive side surface 1622 such that second masking layer 1635 is formed adjacent to edge 1628 of superabrasive table 1514. First protective masking layer 1633 and second protective masking layer 1635 may prevent damage to selected portions of superabrasive element 1610 and may provide a desired leach profile when superabrasive element 1610 is exposed to various reactive agents. For example, first protective masking layer 1633 and/or second protective masking layer 1635 may prevent or delay a leaching solution from contacting certain portions of superabrasive element 1610, such as portions of substrate 1612, portions of superabrasive table 1614, or both, during leaching. In various examples, first protective masking layer 1633 and/or second protective masking layer 1635 may comprise one or more materials that are substantially inert and/or otherwise resistant and/or impermeable to acids, bases, and/or other reactive compounds present in a leaching solution used to leach superabrasive element 1610.

First at-least-partially-degrading masking layer 1637 may be formed on at least a portion of superabrasive element 1610 adjacent to first protective masking layer 1633. For example, first at-least-partially-degrading masking layer 1637 may be formed on portions of superabrasive face 1620 (e.g., at or adjacent to the edge 1627) and/or chamfer 1624. Second at-least-partially-degrading masking layer 1647 may be formed on at least a portion of superabrasive element

1610 adjacent to second protective masking layer 1635. For example, second at-least-partially-degrading masking layer 1647 may be formed on portions of superabrasive side surface 1622 (e.g., at or adjacent to the edge 1627) and/or chamfer 1624. As shown in FIG. 27, first at-least-partially-degrading masking layer 1637 may be separated from second at-least-partially-degrading masking layer 1647. For example, a space between first at-least-partially-degrading masking layer 1637 and second at-least-partially-degrading masking layer 1647 may be formed over at least a portion of superabrasive table 1614, such as, for example, at least a portion of chamfer 1624. Optionally, a space between first at-least-partially-degrading masking layer 1637 and second at-least-partially-degrading masking layer 1647 may also be formed over a portion of superabrasive face 1620 and/or superabrasive side surface 1622.

According to at least one embodiment, first at-least-partially-degrading masking layer 1637 and/or second at-least-partially-degrading masking layer 1647 may comprise a material that breaks down in the presence of a leaching agent. First at-least-partially-degrading masking layer 1637 and/or second at-least-partially-degrading masking layer 1647 may comprise, for example, a polymeric material that breaks down at a desired rate during exposure to the leaching agent. As first at-least-partially-degrading masking layer 1637 and second at-least-partially-degrading masking layer 1647 disintegrate during leaching, portions of superabrasive element 1610 that were covered by first at-least-partially-degrading masking layer 1637 and second at-least-partially-degrading masking layer 1647 may become exposed to the leaching agent. According to additional embodiments, first at-least-partially-degrading masking layer 1637 and/or second at-least-partially-degrading masking layer 1647 may comprise a material that is more permeable to a leaching agent than first protective masking layer 1633 and/or second protective masking layer 1635. In at least one embodiment, first at-least-partially-degrading masking layer 1637 and/or second at-least-partially-degrading masking layer 1647 may be not substantially degrade when exposed to a leaching agent but may be semi-permeable or permeable to the leaching agent.

First protective masking layer 1633, second protective masking layer 1635, first at-least-partially-degrading masking layer 1637, and second at-least-partially-degrading masking layer 1647 may each comprise any suitable material, including metals, alloys, polymers, carbon allotropes, oxides, carbides, glass materials, ceramics, composites, membrane materials (e.g. permeable or semi-permeable materials), and/or any combination of the foregoing, without limitation. Further, first protective masking layer 1633, second protective masking layer 1635, first at-least-partially-degrading masking layer 1637, and second at-least-partially-degrading masking layer 1647 may be affixed to superabrasive element 1610 through any suitable mechanism, without limitation, including, for example, direct bonding, bonding via an intermediate layer, such as an adhesive or braze joint, mechanical attachment, such as mechanical fastening, frictional attachment, and/or interference fitting.

The configuration illustrated in FIG. 27 may enable selective leaching of portions of superabrasive element 1610 to form a desired leach profile within superabrasive table 1614. For example, a volume of superabrasive table 1614 adjacent to an uncovered region between first at-least-partially-degrading masking layer 1637 and second at-least-partially-degrading masking layer 1647 may be leached to a greater depth than surrounding portions of superabrasive

table 1614. As first at-least-partially-degrading masking layer 1637 and second at-least-partially-degrading masking layer 1647 are degraded during leaching, portions of superabrasive table 1614 that were covered by first at-least-partially-degrading masking layer 1637 and second at-least-partially-degrading masking layer 1647 may subsequently be exposed to the leaching agent. Accordingly, volumes of superabrasive table 1614 adjacent to the regions previously covered by first at-least-partially-degrading masking layer 1637 and second at-least-partially-degrading masking layer 1647 may be exposed to the leaching agent upon degradation of first at-least-partially-degrading masking layer 1637 and second at-least-partially-degrading masking layer 1647.

Accordingly, the regions of superabrasive table 1614 that were originally adjacent to first at-least-partially-degrading masking layer 1637 and second at-least-partially-degrading masking layer 1647 may have a shallower leach depth than regions of superabrasive table 1614 that were adjacent to the uncovered region between first at-least-partially-degrading masking layer 1637 and second at-least-partially-degrading masking layer 1647. For example, the configuration illustrated in FIG. 27 may result in a leach profile having a maximum leach depth in the volume of superabrasive table 1614 adjacent to a central portion of chamfer 1624.

According to various embodiments, a charge may be applied to superabrasive element 1610 and electrode 1640 through electrical conductors (e.g., wires or any suitable electrical conductor) 1644 and 1642, respectively. For example, in order to apply a current to a processing solution (e.g., processing solution 72 illustrated in FIG. 9C) for processing superabrasive element 1610, superabrasive element 1610 and electrical conductor 1644 may be positioned in the processing solution (e.g., optionally, with a leaching cup 30 or other protective covering) and a charge may be applied to at least a portion of substrate 1612 (e.g., rear surface 1618) of superabrasive element 1610 through electrical conductor 1644 and an opposite charge may be applied to electrode 1640 through electrical conductor 1642. In at least one embodiment, electrical conductor 1644 may be electrically connected to substrate 1612 by an electrode electrically connected to (e.g., positioned abutting) substrate 1612. In some embodiments, electrical conductor 1644 may be directly connected to superabrasive table 1614 by an electrode electrically connected to (e.g., positioned abutting) superabrasive table 1614.

Electrode 1640 may comprise any suitable size, shape, and/or geometry, without limitation. In some embodiments, electrode 1640 may comprise a circular or non-circular disk shape. For example, electrode 1640 may have a substantially circular outer periphery surrounding a central axis (e.g., central axis 29 shown in FIGS. 1-2). Electrode 1640 may have an outer diameter that is larger than, the same as, or smaller than the outer diameter of element side surface 1615 of superabrasive element 1610, as shown in FIG. 27. When superabrasive element 1610 and electrode 1640 are disposed in the processing solution such that at least a portion of superabrasive table 1614 and electrode 1640 are exposed to the processing solution and a voltage is applied to the processing solution via electrode 1640 and superabrasive table 1614, interstitial materials may be removed from at least a portion of superabrasive table 1614 of superabrasive element 1610 exposed to the processing solution and disposed near electrode 1640. Accordingly, a peripheral region of superabrasive table 1614 defining chamfer 1624 may be leached to a greater depth than a central region of superabrasive table 1614.

FIG. 28 is a cross-sectional side view of a superabrasive element 1710 coated with a masking layer and positioned within a leaching cup 1730 according to at least one embodiment. As illustrated in FIG. 28, a masking layer 1733 may be formed on or disposed adjacent to at least a portion of superabrasive face 1720, such as a central portion of superabrasive face 1720 surrounding a central axis (e.g., central axis 29 shown in FIGS. 1-2). According to at least one embodiment, masking layer 1733 may comprise one or more materials that are substantially inert and/or otherwise resistant and/or impermeable to acids, bases, and/or other reactive compounds present in a leaching solution used to leach superabrasive element 1710.

As illustrated in FIG. 28, superabrasive element 1710 may comprise a superabrasive table 1714 affixed to or formed upon a substrate 1712. Superabrasive table 1714 may be affixed to substrate 1712 at interface 1726. Superabrasive element 1710 may comprise a rear surface 1718, a superabrasive face 1720, and an element side surface 1715, which may include a substrate side surface 1716 formed by substrate 1712 and a superabrasive side surface 1722 formed by superabrasive table 1714. Superabrasive element 1710 may also comprise a chamfer 1724 formed by superabrasive table 1714.

As shown in FIG. 28, superabrasive element 1710 may be positioned within protective leaching cup 1730 such that protective leaching cup 1730 surrounds at least a portion of superabrasive element 1710, including substrate 1712. For example, a base portion and a lateral (e.g., circumferentially extending) portion of the protective leaching cup 1730 may define a recess 1778 therein. When superabrasive element 1710 is positioned within recess 1778 of protective leaching cup 1730, at least a portion of superabrasive element 1710, such as superabrasive table 1714 and/or substrate 1712, may be positioned adjacent to and/or contacting a portion of protective leaching cup 1730. For example, protective leaching cup 1730 may be configured to contact at least a portion of element side surface 1715 of superabrasive element 1710, forming a seal between protective leaching cup 1730 and superabrasive element 1710 that is partially or fully impermeable to various fluids, such as a leaching material (e.g., a leaching solution). As shown, the portion of the protective leaching cup 1730 in contact with at least a portion of the superabrasive element 1710 may be a circumferentially-extending flange extending inwardly from the inner surface of the leaching cup 1730. The protective leaching cup 1730 may substantially cover at least a portion of superabrasive side surface 1722 such that the superabrasive side surface 1722 is protected therealong, such as at least to the edge 1728.

Protective leaching cup 1730 may be formed of any suitable material, without limitation. For example, protective leaching cup 1730 may comprise a flexible, elastic, malleable, and/or otherwise deformable material configured to surround and/or contact at least a portion of superabrasive element 1710. Protective leaching cup 1730 may prevent damage to superabrasive element 1710 when at least a portion of superabrasive element 1710 is exposed to various leaching agents. For example, protective leaching cup 1730 may prevent a leaching solution from chemically contacting and/or damaging certain portions of superabrasive element 1710, such as portions of substrate 1712, portions of superabrasive table 1714, or both, during leaching.

In various embodiments, protective leaching cup 1730 may comprise one or more materials that are substantially inert and/or otherwise resistant to acids, bases, and/or other reactive components present in a leaching solution used to

leach superabrasive element 1710. In some embodiments, protective leaching cup 1730 may comprise one or more materials exhibiting significant stability at various temperatures and/or pressures. In some embodiments, protective leaching cup 1730 may include one or more polymeric materials, such as, for example, nylon, polytetrafluoroethylene (PTFE), polyethylene, polypropylene, rubber, silicone, and/or other polymers, and/or a combination of any of the foregoing, without limitation. For example, protective leaching cup 1730 may comprise PTFE blended with one or more other polymeric materials. Protective leaching cup 1730 may be formed using any suitable technique. For example, protective leaching cup 1730 may comprise a polymeric material that is shaped through a molding process (e.g., injection molding, blow molding, compression molding, drawing, etc.) and/or a machining process (e.g., grinding, lapping, milling, boring, etc.).

In at least one embodiment, protective leaching cup 1730 may comprise a material that is configured to conform to an exterior portion of superabrasive element 1710. For example, protective leaching cup 1730 may include a malleable and/or elastically deformable material that conforms to an exterior shape of a portion of superabrasive table 1714 abutting protective leaching cup 1730, such as superabrasive side surface 1722. According to some embodiments, protective leaching cup 1730 may comprise a material, such as a polymeric material (e.g., elastomer, rubber, plastic, etc.), that conforms to surface imperfections of superabrasive side surface 1722 and/or substrate side surface 1716. Heat and/or pressure may be applied to protective leaching cup 1730 to cause a portion of protective leaching cup 1730 abutting superabrasive side surface 1722 to more closely conform to superabrasive side surface 1722. Accordingly, a seal between superabrasive side surface 1722 and a portion of protective leaching cup 1730 abutting superabrasive side surface 1722 may be improved, thereby inhibiting passage of a leaching agent between superabrasive element 1710 and protective leaching cup 1730.

When superabrasive element 1710 is positioned within protective leaching cup 1730, at least a portion of superabrasive element 1710, such as superabrasive table 1714 and/or substrate 1712, may be positioned adjacent to and/or contacting a portion of protective leaching cup 1730. For example, at least a portion of a seal region of protective leaching cup 1730 may be configured to contact at least a portion of element side surface 1715 of superabrasive element 1710, forming a seal between protective leaching cup 1730 and superabrasive element 1710 that is partially or fully impermeable to various fluids, such as a leaching agent. As shown in FIG. 28, superabrasive element 1710 may be positioned within protective leaching cup 1730 so that at least a portion of the seal region of protective leaching cup 1730 contacts and forms a seal with at least a portion of element side surface 1715, such as at least a portion of superabrasive side surface 1722 and/or at least a portion of substrate side surface 1716.

According to various embodiments, a charge may be applied to superabrasive element 1710 and electrode 1740 through electrical conductors (e.g., wires or any suitable electrical conductor) 1744 and 1742, respectively. For example, in order to apply a current to a processing solution (e.g., processing solution 72 illustrated in FIG. 9C) for processing superabrasive element 1710, superabrasive element 1710 and electrical conductor 1744 may be positioned in the processing solution (e.g., optionally, with a leaching cup 30 or other protective covering) and a charge may be applied to at least a portion of substrate 1712 (e.g., rear

surface 1718) of superabrasive element 1710 through electrical conductor 1744 and an opposite charge may be applied to electrode 1740 through electrical conductor 1742. In at least one embodiment, electrical conductor 1744 may be electrically connected to substrate 1712 by an electrode electrically connected to (e.g., positioned abutting) substrate 1712. In some embodiments, electrical conductor 1744 may be directly connected to superabrasive table 1714 by an electrode electrically connected to (e.g., positioned abutting) superabrasive table 1714.

Electrode 1740 may comprise any suitable size, shape, and/or geometry, without limitation. In some embodiments, electrode 1740 may comprise a circular or non-circular disk shape. For example, electrode 1740 may have a substantially circular outer periphery surrounding a central axis (e.g., central axis 29 shown in FIGS. 1-2). Superabrasive element 1710 may comprise any suitable size, shape, and/or geometry, without limitation. For example, superabrasive element 1710 may comprise a substantially cylindrical or non-cylindrical outer surface surrounding a central axis (e.g., central axis 29 shown in FIGS. 1-2) of superabrasive element 1710. Electrode 1740 may have an outer diameter that is larger than, the same as, or smaller than the outer diameter of element side surface 1715 of superabrasive element 1710, as shown in FIG. 28. When superabrasive element 1710 and electrode 1740 are disposed in the processing solution such that at least a portion of superabrasive table 1714 and electrode 1740 are exposed to the processing solution and a voltage is applied to the processing solution via electrode 1740 and superabrasive table 1714, interstitial materials may be removed from at least a portion of superabrasive table 1714 of superabrasive element 1710 exposed to the processing solution and disposed near electrode 1740.

The configuration illustrated in FIG. 28 may enable selective leaching of portions of superabrasive element 1710 to form a desired leach profile within superabrasive table 1714. For example, a volume of superabrasive table 1714 adjacent to an uncovered region between masking layer 1733 and the seal region of protective leaching cup 1730, such as at or adjacent to edge 1727, edge 1728, and/or chamfer 1724, may be leached to a greater depth than surrounding portions of superabrasive table 1714 covered by masking layer 1733 or the seal region. Leaching such a configuration may result in the formation of leached volumes in portions of superabrasive table 1714 located near chamfer 1724 during leaching.

FIG. 29 is an isometric view of a leaching assembly 61 according to at least one embodiment. As illustrated in FIG. 29, leaching assembly 61 may comprise a lower tray 60 and an upper tray 62. Lower tray 60 and upper tray 62 may comprise any suitable shape, such as, for example, substantially disk-shaped bodies. According to various embodiments, lower tray 60 and upper tray 62 may be connected by at least one cylindrical shaft 68 supporting lower tray 60 and upper tray 62. At least one of lower tray 60 and upper tray 62 may be movable along shaft 68 such that lower tray 60 and upper tray 62 may be supported adjacent to or separated from each other as desired.

A plurality of holes 64 (not all labeled) may be defined in lower tray 60. In some embodiments, a plurality of holes 66 (not all labeled) may also be defined in upper tray 62. Holes 64 may each be configured to hold a superabrasive element 10. Holes 64 may be configured such that superabrasive elements 10 are recessed in holes 64. Holes 64 may extend partially or fully through lower tray 60. Holes 64 may extend through lower tray 60 such that electrical conductors 44 (not all labeled) may be electrically connected to superabrasive

elements 10. Holes 66 defined in upper tray 62 may each be configured to hold an electrode 40 and/or electrical conductor connected to electrode 40. In some embodiments, holes 66 may be configured such that each electrode 40 (not all labeled) is disposed near, but not contacting, a superabrasive face 20 of a respective superabrasive element 10 when lower tray 60 and upper tray 62 are positioned adjacent to each other. Holes 66 may be configured such that at least a portion of each electrode 40 protrudes from upper tray 62 toward lower tray 60. Holes 66 may extend through upper tray 62 such that electrical conductors 42 (not all labeled) may be electrically connected to electrodes 40.

According to at least one embodiment, leaching assembly 61 may be configured such that a volume of a processing solution (e.g., processing solution 72 illustrated and described with respect to FIG. 9C or processing solution 172 as illustrated and described with respect to FIG. 10A) is disposed in each of holes 64. For example, processing solution may be disposed in each hole 64 such that the processing solution contacts and/or surrounds at least a portion of each superabrasive element 10. Accordingly, at least a portion of each superabrasive element 10, such as at least a portion of superabrasive table 14, may be exposed to the processing solution. Alternatively, lower tray 60 may be at least partially submerged in a processing solution and upper tray 62 may be at least partially submerged in the processing solution.

Upper tray 62 containing electrodes 40 disposed in and/or protruding from holes 66 may be positioned adjacent to lower tray 60 containing superabrasive elements 10 and the processing solution in holes 64. Upper tray 62 and lower tray 60 may be positioned such that at least a portion of each electrode 40 is disposed in holes 64 in contact with the processing solution 72. According to various embodiments, at least a portion of lower tray 60 and upper tray 62 may be sealed together so as to prevent processing solution from leaking from leaching assembly 61 during processing.

According to various embodiments, a charge may be applied to superabrasive element 10 and electrode 40 through electrical conductors 44 and 42, respectively. For example, in order to apply a current to the processing solution for processing superabrasive elements 10, a charge may be applied to at least a portion of each superabrasive element 10 through electrical conductors 44 and an opposite charge may be applied to each electrode 40 through electrical conductors 42.

FIGS. 30-41B show superabrasive elements having leach profiles that may be obtained by leaching apparatuses disclosed herein. The superabrasive elements of FIGS. 30-41B are illustrated with at least one leached region that is referred to below as a second volume. The second volume of any of the embodiments shown in FIGS. 30-41B may exhibit the same or similar compositions due to electrochemical leaching as second volume 223/leached volume of FIG. 5A. In the interest of brevity, the specific compositions are not repeated again for each embodiment in connection with FIGS. 30-41B. Additionally, second volume in any of FIGS. 30-41B may further exhibit a multi-layer leached structure when the superabrasive elements of FIGS. 30-41B are subjected to a conventional leaching process and an electrochemical leaching according to any of the embodiments disclosed herein. In such cases, the each second volume in FIGS. 30-41B should be understood to have a composition and structure the same or similar to first volume 227, second volume 229, and transition region 231 shown in FIG. 5B.

FIG. 30 shows a cross-sectional side view of a superabrasive element 1810 according to at least one embodiment. As

illustrated in FIG. 30, superabrasive element 1810 may comprise a superabrasive table 1814 affixed to or formed upon a substrate 1812. Superabrasive table 1814 may be affixed to substrate 1812 at interface 1826. Superabrasive element 1810 may comprise a rear surface 1818, a superabrasive face 1820, and an element side surface 1815, which may include a substrate side surface formed by substrate 1812 and a superabrasive side surface 1822 formed by superabrasive table 1814. Superabrasive element 1810 may also comprise a chamfer 1824 formed by superabrasive table 1814.

As illustrated in FIG. 30, superabrasive table 1814 may include a first volume 1821 comprising an interstitial material and a second volume 1823 having a lower concentration of the interstitial material than first volume 1821. Portions of superabrasive table 1814, such as second volume 1823 may be leached or otherwise processed to remove interstitial materials, such as a metal-solvent catalyst, from the interstitial regions. Second volume 1823 may be created during leaching of superabrasive table 1814 according to any suitable leaching technique. For example, second volume 1823 may be selectively leached by disposing portions of superabrasive table 1814 of superabrasive element 1810 near an electrode during an electrochemical leaching process (e.g., electrochemical leaching referenced in FIG. 9C). In some embodiments, superabrasive element 1810 may first be leached, after which portions of superabrasive element 1810 may be removed to modify the shape of first volume 1821 and/or second volume 1823 according to one or more methods discussed herein.

A transition region 1825 may extend between first volume 1821 and second volume 1823. Transition region 1825 may include amounts of metal-solvent catalyst varying between an amount of metal-solvent catalyst in first volume 1821 and an amount of metal-solvent catalyst in second volume 1823. As illustrated in FIG. 30, first volume 1821 may be located adjacent to a central portion of superabrasive face 1820. For example, first volume 1821 may be disposed about central axis 1829. First volume 1821 may extend between interface 1826 and superabrasive face 1820 with first volume 1821 forming at least a portion of superabrasive face 1820 such that the central portion of superabrasive face 1820 located about central axis 1829 is defined by first volume 1821, as shown in FIG. 30. In some embodiments, first volume 1821 and superabrasive face 1820 may be separated by a thin layer of leached polycrystalline diamond material located adjacent to a central region of superabrasive face 1820.

Second volume 1823 may be formed around at least a portion of first volume 1821. For example, second volume 1823 may comprise an annular volume surrounding at least a portion of first volume 1821 such that an outer portion of superabrasive face 1820 relative to central axis 1829 is defined by second volume 1823. As shown in FIG. 30, second volume 1823 may be located adjacent to superabrasive face 1820 and/or chamfer 1824 so as to at least partially surround a portion of first volume 1821 that is also adjacent to superabrasive face 1820. Second volume 1823 may be located adjacent to element side surface 1815. Second volume 1823 may be separated from interface 1826 between substrate 1812 and superabrasive table 1814 so as to prevent corrosion of substrate 1812 by a leaching solution used to form second volume 1823.

First volume 1821, second volume 1823, and transition region 1825 may be formed to any suitable size and/or shape within superabrasive table 1814, without limitation. For example, transition region 1825 may extend along a generally straight, angular, curved, and/or variable (e.g., zigzag,

undulating) profile between first volume 1821 and second volume 1823. In various embodiments, transition region 1825 may comprise a relatively narrow region between first volume 1821 and second volume 1823, while transition region 1825 may optionally comprise a relatively wider region between first volume 1821 and second volume 1823.

As shown in FIG. 30, second volume 1823 may have a depth 1836 extending from superabrasive face 1820 in a direction substantially perpendicular to superabrasive face 1820. Second volume 1823 may comprise a generally annular-shaped volume defined between a first diameter 1857 and a second diameter 1858 (e.g., partially defining edge 1828) surrounding central axis 1829. The portion of first volume 1821 surrounded by second volume 1823 may be generally defined by first diameter 1857. Second diameter 1858 may represent a diameter of element side surface 1815. Edge 1827 formed at the intersection of chamfer 1824 and superabrasive face 1820 may be located at a third diameter 1859 relative to central axis 1829.

Second volume 1823 may be leached to any suitable depth from superabrasive face 1820, chamfer 1824, and/or superabrasive side surface 1822, without limitation. According to some embodiments, second volume 1823 may have a leach depth greater than or equal to approximately 200  $\mu\text{m}$  as measured in a substantially perpendicular direction from at least one of superabrasive face 1820, chamfer 1824, and/or superabrasive side surface 1822. In various embodiments, second volume 1823 may have a leach depth between approximately 200  $\mu\text{m}$  and approximately 1200  $\mu\text{m}$  (e.g., approximately 200  $\mu\text{m}$ , 250  $\mu\text{m}$ , 300  $\mu\text{m}$ , 350  $\mu\text{m}$ , 400  $\mu\text{m}$ , 450  $\mu\text{m}$ , 500  $\mu\text{m}$ , 550  $\mu\text{m}$ , 600  $\mu\text{m}$ , 650  $\mu\text{m}$ , 700  $\mu\text{m}$ , 750  $\mu\text{m}$ , 800  $\mu\text{m}$ , 850  $\mu\text{m}$ , 900  $\mu\text{m}$ , 950  $\mu\text{m}$ , 1000  $\mu\text{m}$ , 1050  $\mu\text{m}$ , 1100  $\mu\text{m}$ , 1150  $\mu\text{m}$ , or 1200  $\mu\text{m}$ ) as measured in a substantially perpendicular direction from at least one of superabrasive face 1820, chamfer 1824, and/or superabrasive side surface 1822. According to at least one embodiment, a depth of second volume 1823 as measured from a center portion of chamfer 1824 may be between approximately 200  $\mu\text{m}$  and 700  $\mu\text{m}$ . In an embodiment, a depth of second volume 1823 may extend from the superabrasive face 1820 inward to a depth approximately equal to or greater than the base of the chamfer 1824 at edge 1828.

Superabrasive elements 1810 having superabrasive table 1814 comprising first volume 1821 and second volume 1823 may exhibit properties of increased thermal stability, fatigue resistance, strength, and/or wear resistance. Such properties may be enhanced by the shape, size, and/or locations of first volume 1821, second volume 1823, and/or transition region 1825 of superabrasive table 1814. Accordingly, the superabrasive element configuration illustrated in FIG. 30, as well as other configurations illustrated and described herein, may provide significant resistance to undesired spalling, cracking, and/or thermal damage of superabrasive portions, such as superabrasive table 1814, of the superabrasive elements during drilling.

FIG. 31 shows a cross-sectional side view of a superabrasive element 1910 according to at least one embodiment. As illustrated in FIG. 31, superabrasive element 1910 may comprise a superabrasive table 1914 affixed to or formed upon a substrate 1912. Superabrasive table 1914 may be affixed to substrate 1912 at interface 1926. Superabrasive element 1910 may comprise a rear surface 1918, a superabrasive face 1920, and an element side surface 1915, which may include a substrate side surface formed by substrate 1912 and a superabrasive side surface 1922 formed by

superabrasive table 1914. Superabrasive element 1910 may also comprise a chamfer 1924 formed by superabrasive table 1914.

Superabrasive element 1910 may include a first volume 1921 comprising an interstitial material and a second volume 1923 having a lower concentration of the interstitial material than first volume 1921. Portions of superabrasive table 1914, such as second volume 1923, may be leached or otherwise processed to remove interstitial materials, such as a metal-solvent catalyst, from the interstitial regions. A transition region 1925 may extend between first volume 1921 and second volume 1923 so as to border at least a portion of first volume 1921 and second volume 1923. Transition region 1925 may include amounts of an interstitial material varying between an amount of the interstitial material in first volume 1921 and an amount of the interstitial material in second volume 1923. In other embodiments, the boundary may be well defined (i.e., transition region 1925 may be thin compared to a depth of second volume 1923).

Transition region 1925 located between first volume 1921 and second volume 1923 may extend along any suitable profile within superabrasive table 1914. For example, as illustrated in FIG. 31, sloped boundary portion 1955 of transition region 1925 may extend between chamfer 1924 and central boundary portion 1954 along any suitable profile, including, for example, a generally straight, angular, curved, and/or variable (e.g., zigzag, undulating) profile. In an embodiment, transition region 1925 may extend inwardly from the lateral surface of chamfer 1924 and toward substrate 1912 at central boundary portion 1954, such that transition region 1925 may be located substantially above chamfer 1924. According to at least one embodiment, superabrasive element 1910 may be processed such that transition region 1925 intersects chamfer 1924 and/or a surface region adjacent to chamfer 1924 (e.g., superabrasive side surface 1922). Accordingly, as shown in FIG. 31, second volume 1923 may be located directly adjacent to a central portion of superabrasive face 1920. For example, second volume 1923 may be disposed about central axis 1929. A portion of first volume 1921, such as a portion adjacent to chamfer 1924, may peripherally surround at least a portion of second volume 1923.

FIG. 32 shows a cross-sectional side view of a superabrasive element 2010 according to at least one embodiment. As illustrated in FIG. 32, superabrasive element 2010 may comprise a superabrasive table 2014 affixed to or formed upon a substrate 2012. Superabrasive table 2014 may be affixed to substrate 2012 at interface 2026. Superabrasive element 2010 may comprise a rear surface 2018, a superabrasive face 2020, and an element side surface 2015, which may include a substrate side surface formed by substrate 2012 and a superabrasive side surface 2022 formed by superabrasive table 2014. Superabrasive element 2010 may also comprise a chamfer 2024 formed by superabrasive table 2014.

Superabrasive element 2010 may include a first volume 2021 comprising an interstitial material and a second volume 2023 having a lower concentration of the interstitial material than first volume 2021. Portions of superabrasive table 2014, such as second volume 2023, may be leached or otherwise processed to remove interstitial materials, such as a metal-solvent catalyst, from the interstitial regions. A transition region 2025 may extend between first volume 2021 and second volume 2023 so as to border at least a portion of first volume 2021 and second volume 2023. Transition region 2025 may include amounts of an intersti-

tial material varying between an amount of the interstitial material in first volume **2021** and an amount of the interstitial material in second volume **2023**. In other embodiments, the boundary may be well defined (i.e., transition region **2025** may be thin compared to a depth of second volume **2023**).

In some embodiments, as illustrated in FIG. 32, sloped boundary portion **2055** of transition region **2025** may extend between superabrasive side surface **2022** and central boundary portion **2054** along any suitable profile, including, for example, a generally straight, angular, curved, and/or variable (e.g., zigzag, undulating) profile. In an embodiment, transition region **2025** may extend inwardly from the outermost point of chamfer **2024**, dipping toward the substrate **2012** at central boundary portion **2054**, such that transition region **2025** may be located substantially below the chamfer **2024**. According to at least one embodiment, superabrasive element **2010** may be processed such that transition region **2025** intersects superabrasive side surface **2022** below chamfer **2024**.

FIGS. 33-41B show cross-sectional views of superabrasive elements comprising superabrasive tables having leach profiles that may be obtained by leaching apparatuses disclosed herein. While superabrasive elements illustrated in FIGS. 33-41B shown as superabrasive tables without a substrate, the leach profiles illustrated in these figures may also apply to superabrasive elements (e.g., superabrasive element **10** shown in FIGS. 1-2) comprising a superabrasive element bonded to a substrate. According to some embodiments, the superabrasive elements illustrated in FIGS. 33-41B may be formed by leaching a superabrasive element comprising a substrate and a superabrasive table according to any of the techniques described herein and subsequently separating (e.g., by lapping, grinding, wire EDM, etc.) the superabrasive table from the substrate. Alternatively, a superabrasive element may be formed with a substrate, the substrate may be removed, and then the superabrasive table may be leached.

FIG. 33 shows a superabrasive element **2110** comprising a superabrasive table **2114** having a rear surface **2118**, a superabrasive face **2120**, and an element side surface **2115**. Superabrasive element **2110** may comprise an edge **2117** (i.e., sloped or angled) and/or any other suitable surface shape at the intersection of element side surface **2115** and superabrasive face **2120**, including, without limitation, an arcuate surface (e.g., a radius, an ovoid shape, or any other rounded shape), a sharp edge, multiple chamfers/radii, a honed edge, and/or combinations of the foregoing. Element side surface **2115** of superabrasive element **2110** may radially surround a central axis **2129** of superabrasive element **2110**.

Superabrasive element **2110** may include a first volume **2121** comprising an interstitial material and a second volume **2123** having a lower concentration of the interstitial material than first volume **2121**. Portions of superabrasive table **2114**, such as second volume **2123**, may be leached or otherwise processed to remove interstitial materials, such as a metal-solvent catalyst, from the interstitial regions. A transition region **2125** may extend between first volume **2121** and second volume **2123** so as to border at least a portion of first volume **2121** and second volume **2123**. Transition region **2125** may include amounts of an interstitial material varying between an amount of the interstitial material in first volume **2121** and an amount of the interstitial material in second volume **2123**. In other embodi-

ments, the boundary may be well defined (i.e., transition region **2125** may be thin compared to a depth of second volume **2123**).

As shown in FIG. 33, first volume **2121** may extend between rear surface **2118** and transition region **2125**. Second volume **2123** may be formed adjacent to a substantial portion of superabrasive face **2120**. Transition region **2125** bordering second volume **2123** may extend in a direction generally parallel to superabrasive face **2120**. Optionally, a portion of second volume **2123** may extend along at least a portion of element side surface **2115** so as to radially surround at least a portion of first volume **2121**. A portion of transition region **2125** may extend in a direction generally parallel to element side surface **2115**. According to some embodiments, transition region **2125** may have a substantially consistent thickness along element side surface **2115** and/or along superabrasive face **2120**.

FIG. 34 shows a superabrasive element **2210** comprising a superabrasive table **2214** having a rear surface **2218**, a superabrasive face **2220**, and an element side surface **2215**. Superabrasive table **2214** may also form a chamfer **2224** and one or more cutting edges, such as edge **2227** and edge **2228**, adjacent to chamfer **2224**. Element side surface **2215** of superabrasive element **2210** may radially surround a central axis **2229** of superabrasive element **2210**.

Superabrasive element **2210** may include a first volume **2221** comprising an interstitial material and a second volume **2223** having a lower concentration of the interstitial material than first volume **2221**. Portions of superabrasive table **2214**, such as second volume **2223**, may be leached or otherwise processed to remove interstitial materials, such as a metal-solvent catalyst, from the interstitial regions. A transition region **2225** may extend between first volume **2221** and second volume **2223** so as to border at least a portion of first volume **2221** and second volume **2223**. Transition region **2225** may include amounts of an interstitial material varying between an amount of the interstitial material in first volume **2221** and an amount of the interstitial material in second volume **2223**. In other embodiments, the boundary may be well defined (i.e., transition region **2225** may be thin compared to a depth of second volume **2223**).

As shown in FIG. 34, second volume **2223** may be formed adjacent to chamfer **2224** and superabrasive face **2220**, and transition region **2225** may extend from superabrasive face **2220** to edge **2228** formed at the intersection of chamfer **2224** and element side surface **2215**, with a portion of transition region **2225** extending generally parallel to chamfer **2224**.

FIG. 35 shows a superabrasive element **2310** comprising a superabrasive table **2314** having a rear surface **2318**, a superabrasive face **2320**, and an element side surface **2315**. Superabrasive table **2314** may also form a chamfer **2324** and one or more cutting edges, such as edge **2327** and edge **2328**, adjacent to chamfer **2324**. Element side surface **2315** of superabrasive element **2310** may radially surround a central axis **2329** of superabrasive element **2310**.

Superabrasive element **2310** may include a first volume **2321** comprising an interstitial material and a second volume **2323** having a lower concentration of the interstitial material than first volume **2321**. Portions of superabrasive table **2314**, such as second volume **2323**, may be leached or otherwise processed to remove interstitial materials, such as a metal-solvent catalyst, from the interstitial regions. A transition region **2325** may extend between first volume **2321** and second volume **2323** so as to border at least a portion of first volume **2321** and second volume **2323**.

Transition region 2325 may include amounts of an interstitial material varying between an amount of the interstitial material in first volume 2321 and an amount of the interstitial material in second volume 2323. In other embodiments, the boundary may be well defined (i.e., transition region 2325 may be thin compared to a depth of second volume 2323).

As shown in FIG. 35, second volume 2323 may be formed adjacent to chamfer 2324, superabrasive face 2320, and element side surface 2315, and transition region 2325 may extend generally parallel to chamfer 2324 from superabrasive face 2320 to element side surface 2315.

FIG. 36 shows a superabrasive element 2410 comprising a superabrasive table 2414 having a rear surface 2418, a superabrasive face 2420, and an element side surface 2415. Superabrasive table 2414 may also form a chamfer 2424 and one or more cutting edges, such as edge 2427 and edge 2428, adjacent to chamfer 2424. Element side surface 2415 of superabrasive element 2410 may radially surround a central axis 2429 of superabrasive element 2410.

Superabrasive element 2410 may include a first volume 2421 comprising an interstitial material and a second volume 2423 having a lower concentration of the interstitial material than first volume 2421. Portions of superabrasive table 2414, such as second volume 2423, may be leached or otherwise processed to remove interstitial materials, such as a metal-solvent catalyst, from the interstitial regions. A transition region 2425 may extend between first volume 2421 and second volume 2423 so as to border at least a portion of first volume 2421 and second volume 2423. Transition region 2425 may include amounts of an interstitial material varying between an amount of the interstitial material in first volume 2421 and an amount of the interstitial material in second volume 2423. In other embodiments, the boundary may be well defined (i.e., transition region 2425 may be thin compared to a depth of second volume 2423).

As shown in FIG. 36, second volume 2423 may be formed adjacent to chamfer 2424, superabrasive face 2420, and element side surface 2415, and transition region 2425 may extend from superabrasive face 2420 to element side surface 2415, with a portion of transition region 2425 extending generally parallel to chamfer 2424 and another portion of transition region 2425 extending generally parallel to element side surface 2415.

FIG. 37 shows a superabrasive element 2510 comprising a superabrasive table 2514 having a rear surface 2518, a superabrasive face 2520, and an element side surface 2515. Superabrasive table 2514 may also form a chamfer 2524 and one or more cutting edges, such as edge 2527 and edge 2528, adjacent to chamfer 2524. Element side surface 2515 of superabrasive element 2510 may radially surround a central axis 2529 of superabrasive element 2510.

Superabrasive element 2510 may include a first volume 2521 comprising an interstitial material and a second volume 2523 having a lower concentration of the interstitial material than first volume 2521. Portions of superabrasive table 2514, such as second volume 2523, may be leached or otherwise processed to remove interstitial materials, such as a metal-solvent catalyst, from the interstitial regions. A transition region 2525 may extend between first volume 2521 and second volume 2523 so as to border at least a portion of first volume 2521 and second volume 2523. Transition region 2525 may include amounts of an interstitial material varying between an amount of the interstitial material in first volume 2521 and an amount of the interstitial material in second volume 2523. In other embodiments,

the boundary may be well defined (i.e., transition region 2525 may be thin compared to a depth of second volume 2523).

As shown in FIG. 37, second volume 2523 may be formed adjacent to chamfer 2524 and element side surface 2515, and transition region 2525 may extend from edge 2527 formed at the intersection of chamfer 2524 and superabrasive face 2520 to element side surface 2515, with at least a portion of transition region 2525 extending generally parallel to element side surface 2515. In such embodiments, second volume 2523 and/or transition region 2525 may be substantially annular and extend about at least a portion of first volume 2521.

FIG. 38 shows a superabrasive element 2610 comprising a superabrasive table 2614 having a rear surface 2618, a superabrasive face 2620, and an element side surface 2615. Superabrasive table 2614 may also form a chamfer 2624 and one or more cutting edges, such as edge 2627 and edge 2628, adjacent to chamfer 2624. Element side surface 2615 of superabrasive element 2610 may radially surround a central axis 2629 of superabrasive element 2610.

Superabrasive element 2610 may include a first volume 2621 comprising an interstitial material and a second volume 2623 having a lower concentration of the interstitial material than first volume 2621. Portions of superabrasive table 2614, such as second volume 2623, may be leached or otherwise processed to remove interstitial materials, such as a metal-solvent catalyst, from the interstitial regions. A transition region 2625 may extend between first volume 2621 and second volume 2623 so as to border at least a portion of first volume 2621 and second volume 2623. Transition region 2625 may include amounts of an interstitial material varying between an amount of the interstitial material in first volume 2621 and an amount of the interstitial material in second volume 2623. In other embodiments, the boundary may be well defined (i.e., transition region 2625 may be thin compared to a depth of second volume 2623).

As shown in FIG. 38, second volume 2623 may be formed adjacent to chamfer 2624 and transition region 2625 may extend from edge 2627 to edge 2628, which are each adjacent to chamfer 2624. Transition region 2625 may extend along any suitable profile between edge 2627 and edge 2628, without limitation. According to some embodiments, transition region 2625 may comprise an angular profile, as illustrated in FIG. 38. A thickness or depth of second volume 2623, as measured perpendicular to a surface of chamfer 2624, may be maximum generally near the center of chamfer 2624.

FIG. 39 shows a superabrasive element 2710 comprising a superabrasive table 2714 having a rear surface 2718, a superabrasive face 2720, and an element side surface 2715. Superabrasive table 2714 may also form a chamfer 2724 and one or more cutting edges, such as edge 2727 and edge 2728, adjacent to chamfer 2724. Element side surface 2715 of superabrasive element 2710 may radially surround a central axis 2729 of superabrasive element 2710.

Superabrasive element 2710 may include a first volume 2721 comprising an interstitial material and a second volume 2723 having a lower concentration of the interstitial material than first volume 2721. Portions of superabrasive table 2714, such as second volume 2723, may be leached or otherwise processed to remove interstitial materials, such as a metal-solvent catalyst, from the interstitial regions. A transition region 2725 may extend between first volume 2721 and second volume 2723 so as to border at least a portion of first volume 2721 and second volume 2723.

Transition region 2725 may include amounts of an interstitial material varying between an amount of the interstitial material in first volume 2721 and an amount of the interstitial material in second volume 2723. In other embodiments, the boundary may be well defined (i.e., transition region 2725 may be thin compared to a depth of second volume 2723).

As shown in FIG. 39, second volume 2723 may be formed adjacent to chamfer 2724 and transition region 2725 may extend from edge 2727 to edge 2728, which are each adjacent to chamfer 2724. Transition region 2725 may extend along any suitable profile between edge 2727 and edge 2728, without limitation. According to some embodiments, transition region 2725 may comprise an arcuate profile, as illustrated in FIG. 39. A thickness or depth of second volume 2723, as measured perpendicular to a surface of chamfer 2724, may be maximum generally near the center of chamfer 2724.

FIG. 40A shows a superabrasive element 2810 comprising a superabrasive table 2814 having a rear surface 2818, a superabrasive face 2820, and an element side surface 2815. Superabrasive table 2814 may also form a chamfer 2824 and one or more cutting edges, such as edge 2827 and edge 2828, adjacent to chamfer 2824. Element side surface 2815 of superabrasive element 2810 may radially surround a central axis 2829 of superabrasive element 2810.

Superabrasive element 2810 may include a first volume 2821 comprising an interstitial material and a second volume 2823 having a lower concentration of the interstitial material than first volume 2821. Portions of superabrasive table 2814, such as second volume 2823, may be leached or otherwise processed to remove interstitial materials, such as a metal-solvent catalyst, from the interstitial regions. A transition region 2825 may extend between first volume 2821 and second volume 2823 so as to border at least a portion of first volume 2821 and second volume 2823. Transition region 2825 may include amounts of an interstitial material varying between an amount of the interstitial material in first volume 2821 and an amount of the interstitial material in second volume 2823. In other embodiments, the boundary may be well defined (i.e., transition region 2825 may be thin compared to a depth of second volume 2823).

As shown in FIG. 40A, second volume 2823 may be formed adjacent to chamfer 2824 and transition region 2825 may extend from superabrasive face 2820 to element side surface 2815. Transition region 2825 may extend along any suitable profile between superabrasive face 2820 and element side surface 2815, without limitation. Transition region 2825 may comprise, for example, a profile that generally slopes between superabrasive face 2820 and element side surface 2815. For example, transition region 2825 may extend from a region of element side surface 2815 near edge 2828 to a region of superabrasive face 2820 disposed apart from edge 2827. According to some embodiments, as shown in FIG. 40A, the generally annular-shaped second volume 2823 may comprise a generally ring-shaped volume that is not perfectly symmetric but is irregular in one or more dimensions. For example, second volume 2823 may vary in leach depth and/or profile shape, as defined by transition region 2825, at different peripheral regions about central axis 2829.

FIG. 40B shows a superabrasive element 2910 comprising a superabrasive table 2914 having a rear surface 2918, a superabrasive face 2920, and an element side surface 2915. Superabrasive table 2914 may also form a chamfer 2924 and one or more cutting edges, such as edge 2927 and edge 2928,

adjacent to chamfer 2924. Element side surface 2915 of superabrasive element 2910 may radially surround a central axis 2929 of superabrasive element 2910.

Superabrasive element 2910 may include a first volume 2921 comprising an interstitial material and a second volume 2923 having a lower concentration of the interstitial material than first volume 2921. Portions of superabrasive table 2914, such as second volume 2923, may be leached or otherwise processed to remove interstitial materials, such as a metal-solvent catalyst, from the interstitial regions. A transition region 2925 may extend between first volume 2921 and second volume 2923 so as to border at least a portion of first volume 2921 and second volume 2923. Transition region 2925 may include amounts of an interstitial material varying between an amount of the interstitial material in first volume 2921 and an amount of the interstitial material in second volume 2923. In other embodiments, the boundary may be well defined (i.e., transition region 2925 may be thin compared to a depth of second volume 2923).

As shown in FIG. 40B, second volume 2923 may be formed adjacent to chamfer 2924 and transition region 2925 may extend from superabrasive face 2920 to element side surface 2915. Transition region 2925 may extend along any suitable profile between superabrasive face 2920 and element side surface 2915, without limitation. Transition region 2925 may comprise, for example, a profile that generally slopes between superabrasive face 2920 and element side surface 2915. For example, transition region 2925 may extend from a region of element side surface 2915 near edge 2928 to a region of superabrasive face 2920 disposed apart from edge 2927. According to some embodiments, as shown in FIG. 40B, the generally annular-shaped second volume 2923 may comprise a generally ring-shaped volume that is not perfectly symmetric but is irregular in one or more dimensions. For example, second volume 2923 may vary in leach depth and/or profile shape, as defined by transition region 2925, at different peripheral regions about central axis 2929.

FIG. 41A shows a superabrasive element 3010 comprising a superabrasive table 3014 having a rear surface 3018, a superabrasive face 3020, and an element side surface 3015. Superabrasive table 3014 may also form a chamfer 3024 and one or more cutting edges, such as edge 3027 and edge 3028, adjacent to chamfer 3024. Element side surface 3015 of superabrasive element 3010 may radially surround a central axis 3029 of superabrasive element 3010.

Superabrasive element 3010 may include a first volume 3021 comprising an interstitial material and a second volume 3023 having a lower concentration of the interstitial material than first volume 3021. Portions of superabrasive table 3014, such as second volume 3023, may be leached or otherwise processed to remove interstitial materials, such as a metal-solvent catalyst, from the interstitial regions. A transition region 3025 may extend between first volume 3021 and second volume 3023 so as to border at least a portion of first volume 3021 and second volume 3023. Transition region 3025 may include amounts of an interstitial material varying between an amount of the interstitial material in first volume 3021 and an amount of the interstitial material in second volume 3023. In other embodiments, the boundary may be well defined (i.e., transition region 3025 may be thin compared to a depth of second volume 3023).

As shown in FIG. 41A, second volume 3023 may be formed adjacent to chamfer 3024, superabrasive face 3020, and element side surface 3015, and transition region 3025

may extend from superabrasive face 3020 to rear surface 3018 (or to an interface between superabrasive table 3014 and an adjacent substrate), with transition region 3025 extending generally parallel to element side surface 3015.

FIG. 41B shows a superabrasive element 3110 comprising a superabrasive table 3114 having a rear surface 3118, a superabrasive face 3120, and an element side surface 3115. Superabrasive table 3114 may also form a chamfer 3124 and one or more cutting edges, such as edge 3127 and edge 3128, adjacent to chamfer 3124. Element side surface 3115 of superabrasive element 3110 may radially surround a central axis 3129 of superabrasive element 3110.

Superabrasive element 3110 may include a first volume 3121 comprising an interstitial material and a second volume 3123 having a lower concentration of the interstitial material than first volume 3121. Portions of superabrasive table 3114, such as second volume 3123, may be leached or otherwise processed to remove interstitial materials, such as a metal-solvent catalyst, from the interstitial regions. A transition region 3125 may extend between first volume 3121 and second volume 3123 so as to border at least a portion of first volume 3121 and second volume 3123. Transition region 3125 may include amounts of an interstitial material varying between an amount of the interstitial material in first volume 3121 and an amount of the interstitial material in second volume 3123. In other embodiments, the boundary may be well defined (i.e., transition region 3125 may be thin compared to a depth of second volume 3123).

As shown in FIG. 41B, second volume 3123 may be formed adjacent to superabrasive face 3120, and extend generally parallel to chamfer 3124 and element side surface 3115, and the transition region 3125 may extend from superabrasive face 3120 to rear surface 3118 (or to an interface between superabrasive table 3114 and an adjacent substrate).

Any of the above-described superabrasive elements and first and second regions therein may be formed using one or more corresponding electrodes (e.g., electrodes having complementary positioning and/or geometry) as disclosed above. For example, the first and second volumes 2121 and 2123 of superabrasive element 2110 in FIG. 33 may be formed using the electrode 540 of FIG. 15.

FIG. 42 is an isometric view of a drill bit 80 according to at least one embodiment. Drill bit 80 may represent any type or form of earth-boring or drilling tool, including, for example, a rotary drill bit. As illustrated in FIG. 42, drill bit 80 may comprise a bit body 81 having a longitudinal axis 84. Bit body 81 may define a leading end structure for drilling into a subterranean formation by rotating bit body 81 about longitudinal axis 84 and applying weight to bit body 81. Bit body 81 may include radially and longitudinally extending blades 79 with leading faces 82 and a threaded pin connection 83 for connecting bit body 81 to a drill string.

At least one superabrasive element according to any of the embodiments disclosed herein may be coupled to bit body 81. For example, as shown in FIG. 42, a plurality of superabrasive elements 10 may be coupled to blades 79. Drill bit 80 may utilize any of the disclosed superabrasive elements 10 as cutting elements. Circumferentially adjacent blades 79 may define so-called junk slots 85 therebetween. Junk slots 85 may be configured to channel debris, such as rock or formation cuttings, away from superabrasive elements 10 during drilling. Drill bit 80 may also include a plurality of nozzle cavities 86 for communicating drilling fluid from the interior of drill bit 80 to superabrasive elements 10.

FIG. 42 depicts an example of a drill bit 80 that employs at least one cutting element 10. Drill bit 80 may represent any number of earth-boring tools or drilling tools, including, for example, core bits, roller-cone bits, fixed-cutter bits, eccentric bits, bicenter bits, reamers, reamer wings, and/or any other downhole tools comprising superabrasive cutting elements and/or discs, without limitation. Superabrasive elements 10 disclosed herein may also be utilized in applications other than cutting technology. For example, embodiments of superabrasive elements 10 disclosed herein may also form all or part of heat sinks, wire dies, bearing elements, cutting elements, cutting inserts (e.g., on a roller cone type drill bit), machining inserts, or any other article of manufacture, as known in the art. According to some examples, superabrasive elements 10, as disclosed herein, may be employed in medical device applications, including, without limitation, hip joints, back joints, or any other suitable medical joints. Thus, superabrasive elements 10, as disclosed herein, may be employed in any suitable article of manufacture. Other examples of articles of manufacture that may incorporate superabrasive elements as disclosed herein may be found in U.S. Pat. Nos. 4,811,801; 4,268,276; 4,468,138; 4,738,322; 4,913,247; 5,016,718; 5,092,687; 5,120,327; 5,135,061; 5,154,245; 5,460,233; 5,544,713; and 6,793,681, the disclosure of each of which is incorporated herein, in its entirety, by this reference.

In additional embodiments, a rotor and a stator, such as a rotor and a stator used in a thrust bearing apparatus, may each include at least one superabrasive element according to the embodiments disclosed herein. By way of example, U.S. Pat. Nos. 4,410,054; 4,560,014; 5,364,192; 5,368,398; and 5,480,233, the disclosure of each of which is incorporated herein, in its entirety, by this reference, disclose subterranean drilling systems that include bearing apparatuses utilizing superabrasive elements 10 as disclosed herein.

FIG. 43 is partial cross-sectional isometric view of a thrust-bearing apparatus 87 according to at least one embodiment. Thrust-bearing apparatus 87 may utilize any of the disclosed superabrasive elements 10 as bearing elements. Thrust-bearing apparatus 87 may also include bearing assemblies 88A and 88B. Each of bearing assembly 88A and 88B may include a support ring 89 fabricated from a material, such as steel, stainless steel, or any other suitable material, without limitation.

Each support ring 89 may include a plurality of recesses 90 configured to receive corresponding superabrasive elements 10. Each superabrasive element 10 may be mounted to a corresponding support ring 89 within a corresponding recess 90 by brazing, welding, press-fitting, using fasteners, or any other suitable mounting technique, without limitation. In at least one embodiment, one or more of superabrasive elements 10 may be configured according to any of the superabrasive element embodiments described herein. For example, each superabrasive element 10 may include a substrate 12 and a superabrasive table 14 comprising a PCD material. Each superabrasive table 14 may form a superabrasive face 20 that is utilized as a bearing surface.

Superabrasive faces 20 of bearing assembly 88A may bear against opposing superabrasive faces 20 of bearing assembly 88B in thrust-bearing apparatus 87, as illustrated in FIG. 43. For example, bearing assembly 88A of thrust-bearing apparatus 87 may be termed a "rotor." The rotor may be operably coupled to a rotational shaft. Bearing assembly 88B of thrust-bearing apparatus 87 may be held substantially stationary relative to the bearing assembly 88A and may be termed a "stator."

FIG. 44 is an isometric view of a radial bearing apparatus 91 according to another embodiment. Radial bearing apparatus 91 may utilize any of the disclosed superabrasive element embodiments as bearing elements 10A and 10B. Radial bearing apparatus 91 may include an inner race 92A positioned generally within an outer race 92B. Inner race 92A may include a plurality of bearing elements 10A affixed thereto, and outer race 92B may include a plurality of corresponding bearing elements 10B affixed thereto. One or more of bearing elements 10A and 10B may be configured in accordance with any of the superabrasive element embodiments disclosed herein.

Inner race 92A may be positioned generally within outer race 92B. Thus, inner race 92A and outer race 92B may be configured such that bearing surfaces 20A defined by bearing elements 10A and bearing surfaces 20B defined by bearing elements 10B may at least partially contact one another and move relative to one another as inner race 92A and outer race 92B rotate relative to each other. According to various embodiments, thrust-bearing apparatus 87 and/or radial bearing apparatus 91 may be incorporated into a subterranean drilling system.

FIG. 45 is a partial cross-sectional isometric view of a subterranean drilling system 93 that includes a thrust-bearing apparatus 87, as shown in FIG. 43, according to at least one embodiment. The subterranean drilling system 93 may include a housing 94 enclosing a downhole drilling motor 95 (i.e., a motor, turbine, or any other suitable device capable of rotating an output shaft, without limitation) that is operably connected to an output shaft 96.

The thrust-bearing apparatus 87 shown in FIG. 43 may be operably coupled to downhole drilling motor 95. A rotary drill bit 97, such as a rotary drill bit configured to engage a subterranean formation and drill a borehole, may be connected to output shaft 96. As illustrated in FIG. 45, rotary drill bit 97 may be a roller cone bit comprising a plurality of roller cones 98. According to additional embodiments, rotary drill bit 97 may comprise any suitable type of rotary drill bit, such as, for example, a so-called fixed-cutter drill bit. As a borehole is drilled using rotary drill bit 97, pipe sections may be connected to subterranean drilling system 93 to form a drill string capable of progressively drilling the borehole to a greater depth within a subterranean formation.

A thrust-bearing assembly 88A in thrust-bearing apparatus 87 may be configured as a rotor that is attached to output shaft 96 and a thrust-bearing assembly 88B in thrust-bearing apparatus 87 may be configured as a stator. During a drilling operation using subterranean drilling system 93, the rotor may rotate in conjunction with output shaft 96 and the stator may remain substantially stationary relative to the rotor.

According to various embodiments, drilling fluid may be circulated through downhole drilling motor 95 to generate torque and effect rotation of output shaft 96 and rotary drill bit 97 attached thereto so that a borehole may be drilled. A portion of the drilling fluid may also be used to lubricate opposing bearing surfaces of superabrasive elements 10 on thrust-bearing assemblies 88A and 88B.

FIG. 46 illustrates a method 3200 for processing a polycrystalline diamond element according to at least one embodiment. As shown in FIG. 46, at least a portion of a polycrystalline diamond material may be exposed to a processing solution, the polycrystalline diamond material comprising a metallic material disposed in interstitial spaces defined within the polycrystalline diamond material (act 3202). In some embodiments, for example, a superabrasive element 10 comprising a superabrasive table 14 and a substrate 12 may be disposed in a

protective leaching cup 30 such that the protective leaching cup surrounds substrate 12 and/or at least a portion of superabrasive table 14. Superabrasive element 10 and protective leaching cup 30 may be disposed in a cavity 76 of a processing vessel 70 such that a processing solution 72 contacts at least a portion of superabrasive element 10 as illustrated in FIG. 9C.

An electrode may be exposed to the processing solution (act3204). For example, as shown in FIG. 9C, an electrode 40 may be disposed in processing vessel 70 such that electrode 40 and superabrasive element 10 surrounded by protective leaching cup 30 are at least partially submerged in processing solution 72. Electrode 40 may be exposed to processing solution 72 such that processing solution 72 contacts at least a portion of electrode 40.

A first charge may be applied to the polycrystalline diamond material (act3206). For example, as shown in FIG. 9C, a charge may be applied to superabrasive element 10 through an electrical conductor 44. In some embodiments, a positive charge may be applied to at least a portion of substrate 12 (e.g., rear surface 18) of superabrasive element 10 through electrical conductor 44. In at least one embodiment, electrical conductor 44 may be electrically connected to substrate 12 by an electrode electrically connected to (e.g., positioned abutting) substrate 12. In some embodiments, electrical conductor 44 may be directly connected to superabrasive table 14 by an electrode electrically connected to (e.g., positioned abutting) superabrasive table 14.

A second charge may be applied to the electrode 30 (act3208). For example, as shown in FIG. 9C, a charge may be applied to electrode 40 through an electrical conductor 42. In some embodiments, an opposite charge (e.g., a negative charge) may be applied to electrode 40 through electrical conductor 42.

FIG. 47 illustrates a method 3300 for processing a polycrystalline diamond element according to at least one embodiment. As shown in FIG. 47, a superabrasive element may be provided, the superabrasive element comprising a substrate and a polycrystalline diamond table bonded to the substrate, the polycrystalline diamond table comprising a metallic material disposed in interstitial spaces defined within the polycrystalline diamond table (act3302). For example, as shown in FIGS. 1 and 2, a superabrasive element 10 comprising a substrate 12 bonded to a superabrasive table 14 may be provided. Superabrasive table 14 may comprise a polycrystalline diamond table with metal-solvent catalyst and/or other materials (e.g. interstitial material 239) disposed in interstitial spaces (e.g. interstitial regions 236) defined within the polycrystalline diamond table, as illustrated in FIGS. 6A and 6B.

At least a portion of the polycrystalline diamond table may be exposed to a processing solution (act3304). In some embodiments, for example, a superabrasive element 10 may be disposed in a protective leaching cup 30 such that the protective leaching cup surrounds substrate 12 and/or at least a portion of superabrasive table 14. Superabrasive element 10 and protective leaching cup 30 may be disposed in a cavity 76 of a processing vessel 70 such that a processing solution 72 contacts at least a portion of superabrasive element 10 as illustrated in FIG. 9C.

An electrode may be exposed to the processing solution (act3306). For example, as shown in FIG. 9C, an electrode 40 may be disposed in processing vessel 70 such that electrode 40 and superabrasive element 10 surrounded by protective leaching cup 30 are at least partially submerged in processing solution 72. The electrode 40 may be positioned in contact with, adjacent to, or otherwise proximate to at

least one of superabrasive surface 20, superabrasive side surface 22, or chamfer 24. Electrode 40 may be exposed to processing solution 72 such that processing solution 72 contacts at least a portion of electrode 40.

A first charge may be applied to the metallic material in the superabrasive element 10 (act3308). For example, as shown in FIG. 9C, the first charge may be applied to superabrasive element 10 through an electrical conductor 44. In an embodiment, the first charge may be applied to a PCD table effective to oxidize the metallic material (e.g., interstitial metallic material) therein.

A second charge may be applied to the electrode 40 (act3310). For example, as shown in FIG. 9C, an opposite charge may be applied to electrode 40 through an electrical conductor 42. In an embodiment, the second charge may be applied to the electrode 40 effective to reduce the oxidized metallic material (e.g., cationic interstitial metal) in the processing solution 72, which may plate at least some of the metallic material onto the electrode 40.

The following examples set forth various methods used to form superabrasive elements as disclosed herein. The following examples provide further detail in connection with the specific embodiments described above.

#### Example 1

Cutting elements, each comprising a PCD table attached to a tungsten carbide substrate, were formed by HPHT sintering diamond particles in the presence of cobalt. The sintered-polycrystalline-diamond tables included cobalt and tungsten within the interstitial regions between the bonded diamond grains.

The PCD tables were leached using an aqueous processing solution having a molar concentration of 0.29 M citric acid. The processing solution for processing each cutting element contacted both the PCD table and a corresponding disk-shaped copper electrode disposed near the PCD table. A negative charge was applied to each electrode and a positive charge was applied to the substrate of each cutting element such that a voltage of 0.8 V was generated in the processing solution. The PCD tables were leached at a temperature of approximately 75° C. and atmospheric pressure for between 24 and 168 hours. Following leaching, leach depths of the PCD tables were determined for various portions of the PCD tables, including leach depths measured from the cutting faces, side surfaces, and chamfered cutting edges of the PCD tables, and the leach depths were averaged.

Following 24 hours of leaching, a first PCD table included a leach depth of approximately 167 µm.

Following 72 hours of leaching, a second PCD table included a leach depth of approximately 308 µm.

Following 168 hours of leaching, a third PCD table included a leach depth of approximately 611 µm.

#### Example 2

Cutting elements, each comprising a PCD table attached to a tungsten carbide substrate, were formed by HPHT sintering diamond particles in the presence of cobalt. The sintered-polycrystalline-diamond tables included cobalt and tungsten within the interstitial regions between the bonded diamond grains.

The PCD tables were leached using an aqueous processing solution having a citrate buffer comprising a molar concentration of 0.24 M sodium citrate and 0.05 M citric acid and having a pH of 6.5. The processing solution for

processing each cutting element contacted both the PCD table and a corresponding disk-shaped copper electrode disposed near the PCD table. A negative charge was applied to each electrode and a positive charge was applied to the substrate of each cutting element such that a voltage of 0.8 V was generated in the processing solution. The PCD tables were leached at a temperature of approximately 75° C. and atmospheric pressure for between 24 and 72 hours. Following leaching, leach depths of the PCD tables were determined for various portions of the PCD tables, including leach depths measured from the cutting faces, side surfaces, and chamfered cutting edges of the PCD tables, and the leach depths were averaged.

Following 24 hours of leaching, a first PCD table included a leach depth of approximately 120 µm.

Following 72 hours of leaching, a second PCD table included a leach depth of approximately 250 µm.

#### Example 3

Cutting elements, each comprising a PCD table attached to a tungsten carbide substrate, were formed by HPHT sintering diamond particles in the presence of cobalt. The sintered-polycrystalline-diamond tables included cobalt and tungsten within the interstitial regions between the bonded diamond grains.

The PCD tables were each leached in one of a plurality of aqueous processing solutions having a molar concentration of 0.29 M citric acid and various concentrations of cobalt chloride. The processing solutions for processing each cutting element contacted both the PCD table and a corresponding disk-shaped copper electrode disposed near the PCD table. A negative charge was applied to each electrode and a positive charge was applied to the substrate of each cutting element such that a voltage of 0.8 V was generated in the processing solution. The PCD tables were leached at a temperature of approximately 75° C. and atmospheric pressure for 72 hours. Following leaching, leach depths of the PCD tables were determined for various portions of the PCD tables, including leach depths measured from the cutting faces, side surfaces, and chamfered cutting edges of the PCD tables, and the leach depths were averaged.

Following leaching in a processing solution containing no cobalt chloride, a first PCD table included a leach depth of approximately 188 µm.

Following leaching in a processing solution having a molar concentration of 0.05 M cobalt chloride, a first PCD table included a leach depth of approximately 219 µm.

Following leaching in a processing solution having a molar concentration of 0.1 M cobalt chloride, a first PCD table included a leach depth of approximately 233 µm.

#### Example 4

Cutting elements, each comprising a PCD table attached to a tungsten carbide substrate, were formed by HPHT sintering diamond particles in the presence of cobalt. The sintered-polycrystalline-diamond tables included cobalt and tungsten carbide within the interstitial regions between the bonded diamond grains.

The PCD tables were each leached in an aqueous processing solution of 0.29 M citric acid and 0.1 M cobalt chloride (II). The aqueous processing solution for processing each cutting element contacted both the PCD table and a corresponding disk-shaped copper electrode disposed near the PCD table. A negative charge was applied to the electrode and a positive charge was applied to the substrate of

each cutting element such that a voltage of 0.8 V was generated between the electrode and the substrate. The PCD tables were leached for 168 hours with the aqueous processing solution at a temperature of approximately 90° C. and at atmospheric pressure.

Following leaching, leach depths of the PCD tables were determined for various portions of the PCD tables, including leach depths measured from the cutting faces, side surfaces, and chamfered cutting edges of the PCD tables, and the leach depths were averaged. The leach depth for one of the PCD tables of Example 4 that was electrochemically leached ranged from about 595  $\mu\text{m}$  to about 618  $\mu\text{m}$  measured from the superabrasive face, and about 629  $\mu\text{m}$  to about 686  $\mu\text{m}$  measured inwardly from the chamfer.

The composition of the leached volume of the PCD tables were also determined using x-ray diffraction Rietveld analysis. Table 1 below lists the compositional data by weight % (wt %) obtained by x-ray diffraction Rietveld analysis of a surface of the leached volumes of the PCD tables of Example 4.

#### Comparative Example 5

Cutting elements, each comprising a PCD table attached to a tungsten carbide substrate, were formed by HPHT sintering diamond particles in the presence of cobalt. The sintered-polycrystalline-diamond tables included cobalt and tungsten carbide within the interstitial regions between the bonded diamond grains.

The PCD tables were each leached in a mixture of hydrofluoric and nitric acid. The PCD tables were leached for 192 hours with the mixture at a temperature of approximately 75° C. and atmospheric pressure. Following leaching, leach depths of the PCD tables were determined for various portions of the PCD tables, including leach depths measured from the cutting faces and chamfered cutting edges of the PCD tables. The leach depth for one of the PCD tables that was conventionally leached ranged from about 531  $\mu\text{m}$  to about 546  $\mu\text{m}$  measured from the superabrasive face, and about 616  $\mu\text{m}$  to about 823  $\mu\text{m}$  measured inwardly from the chamfer.

The composition of the leached volume of the PCD tables of Example 5 were also determined using x-ray diffraction Rietveld analysis. Table 2 below lists compositional data (by wt %) obtained by x-ray diffraction Rietveld analysis of a surface of the leached volumes of the PCD tables of Example 5.

TABLE 1

Compositional Data for Leached Volumes of the PCD Tables of Example 4

| Sample No. | Phases Present          |               |                |                                |
|------------|-------------------------|---------------|----------------|--------------------------------|
|            | Tungsten Carbide (wt %) | Cobalt (wt %) | Diamond (wt %) | Cobalt Tungsten Carbide (wt %) |
| Example 4a | 0.788                   | 1.39          | 97.6           | 0.230                          |
| Example 4b | 0.60                    | 1.20          | 97.7           | 0.47                           |
| Example 4c | 0.662                   | 1.15          | 97.9           | 0.27                           |
| Example 4d | 0.769                   | 1.35          | 97.7           | 0.20                           |
| Example 4e | 0.798                   | 1.17          | 97.8           | 0.22                           |

TABLE 2

Compositional Data for Leached Volumes of the PCD Tables That Were Conventionally Leached

| Sample No. | Phases Present                 |               |                |
|------------|--------------------------------|---------------|----------------|
|            | Cobalt Tungsten Carbide (wt %) | Cobalt (wt %) | Diamond (wt %) |
| 1          | 0.33                           | 1.33          | 98.5           |
| 2          | 0.427                          | 1.19          | 98.4           |
| 3          | 0.19                           | 1.29          | 98.5           |
| 4          | 0.48                           | 1.37          | 98.1           |
| 5          | 0.252                          | 1.40          | 98.3           |

Both the cutting elements of Examples 4 and 5 were tested in a vertical turret lathe (VTL) test to evaluate abrasion resistance. The abrasion resistance was evaluated using a VTL test by measuring the volume of cutting element removed or diamond volume removed (DVR) removed versus the volume of Barre granite workpiece removed, while the workpiece was cooled with water. The test parameters used were a depth of cut for the cutting element of about 0.254 mm, a back rake angle for the cutting element of about 20 degrees, an in-feed for the PDC of about 6.35 mm/rev, and a rotary speed of the workpiece to be cut of about 101 RPM. The volume of Barre granite workpiece removed is about 470  $\text{in}^3$  at 50 passes and 2350  $\text{in}^3$  at 250 passes.

FIG. 48 shows the abrasion resistance test data for Examples 4 and 5. The electrochemically leached PCD tables of Example 4 performed statistically better than conventionally leached PCD tables of Example 5 at 100, 150, 200, 250 and 300 passes. At 300 passes, the abrasion resistance of the electrochemical leached PCD tables of Example 4 was about 40% better than the conventionally leached PCD tables of Example 5. The electrochemical leaching process left about 80 times more tungsten carbide in the leached PCD tables of Example 4 than the conventionally leached PCD tables of Example 5.

The leach profiles were also different for the PCD tables of Examples 4 and 5. FIGS. 49A-49C are photomicrographs of different sections of a PCD table of Example 4 at 75 $\times$ .

FIGS. 50A-50C are photomicrographs of different sections of a PCD table of Example 5 at 75 $\times$ . As shown in FIGS. 49A-49C and 50A-50C, the leach profile of the leached volume more closely contours the exterior profile of the PCD table in the electrochemically leached PCD tables of Example 4 than the conventionally leached PCD tables of Example 5. The inventors currently believe that the presence of tungsten and/or tungsten carbide in the leached volume of the PCD tables of Example 4 and the leach profile thereof contributed to the enhanced abrasion resistance compared to the conventionally leached PCD tables of Example 5.

#### Examples 6 and 7

Cutting elements, each comprising a PCD table attached to a cobalt-cemented tungsten carbide substrate, were formed by HPHT sintering diamond particles in the presence of cobalt. The sintered-polycrystalline-diamond tables included cobalt and tungsten-containing material within the interstitial regions between the bonded diamond grains. The PCD tables were subsequently removed from the substrate. The PCD tables were separated into two groups—Example 6 and Example 7—for further processing.

Each of the PCD tables of Example 6 was electrochemically leached in a solution of 0.29 M citric acid and 0.1 M cobalt chloride. After leaching, each PCD table of Example 6 was crushed using repeated blows from a domed PDC. Following crushing, each crushed PCD table was leached a second time in a conventional nonelectrochemical leaching process including immersion in an acidic solution of hydrofluoric and nitric acid to cause chemical digestion.

Each of the PCD tables of Example 7 was conventionally nonelectrochemically leached in the same type of acidic solution of hydrofluoric acid and nitric acid used to cause chemical digestion of Example 6. After leaching, each PCD table of Example 7 was crushed using repeated blows from a domed PDC. Following crushing, each crushed PCD table was conventionally leached a second time in the same type of acidic solution of hydrofluoric and nitric acid used to cause chemical digestion of Example 6.

Following the second leaching process of each of Examples 6 and 7 used to cause chemical digestion, the tungsten and cobalt content of each second leaching solution was analyzed using inductively coupled plasma atomic absorption spectrometry (ICP-AAS) on the respective leaching solutions. The amount of cobalt and tungsten present in the second leaching solution(s) was used to determine the amount of cobalt and tungsten-containing material (e.g., tungsten carbide or tungsten) removed in the second leaching process as units of mg of analyte removed per gram of PCD table (where the PDC table was weighed prior to crushing and digestion). The graphs in FIGS. 51A and 51B demonstrated the relative efficiency of the respective first leaching techniques on cobalt and tungsten-containing material in the PCD tables as a function of the amount of cobalt and tungsten-containing material left in the PCD tables after the first leaching processes.

FIG. 51A is a plot diagram of the amount of cobalt removed from Example 6 and Example 7 after the second leaching process described above. As shown, after the electrochemical leaching associated with Example 6, further leaching of Example 6 removed nearly 8 mg of cobalt per gram of PCD table (average of 7.64 mg Co/g PCD table). After the first conventional leaching associated with Example 7, the second conventional leaching of Example 7 removed nearly 1 mg of cobalt per mg of PCD table (average of 0.66 mg Co/g PCD table).

FIG. 51B is a plot diagram of the amount of tungsten removed from Example 6 and Example 7 after the second leaching process described above. As shown, after the electrochemical leaching associated with Example 6, further leaching of Example 6 removed nearly 24 mg of tungsten per gram of PCD table (average of 23.92 mg W/g PCD table). After the first conventional leaching associated with Example 7, the second conventional leaching of Example 7 removed very little tungsten-containing material per gram of PCD table (average of 0.20 mg W/g PCD table).

As shown, electrochemical leaching preferentially leached cobalt over tungsten-containing material, leaving a relatively larger amount of tungsten-containing material in the interstitial spaces of a PCD table than conventional leaching, while simultaneously removing the cobalt therein.

#### Examples 8 and 9

Cutting elements, each comprising a PCD table attached to a cobalt-cemented tungsten carbide substrate, were formed by HPHT sintering diamond particles in the presence of cobalt. The sintered-polycrystalline diamond tables included cobalt and tungsten-containing material within the

interstitial regions between the bonded diamond grains. The PCD tables were subsequently removed from the substrate. The PCD tables were separated into two groups—Example 8 and Example 9—for further processing.

5 Each of the PCD tables of Example 8 was electrochemically leached in a solution of 0.29 M citric acid and 0.1 M cobalt chloride. Each of the PCD tables of Example 9 was conventionally nonelectrochemically leached in an acidic solution of hydrofluoric acid and nitric acid.

10 Following the respective leaching processes of each of Examples 8 and 9, the tungsten and cobalt content of each leaching solution associated therewith (having the dissolved contents of the PCD tables therein) was analyzed using ICP-AAS. The ratio of amount of cobalt to tungsten in the 15 respective leaching solutions was determined. The ratio of amount of cobalt to tungsten present in the respective leaching solutions showed the preferential nature of electrochemical leaching to cobalt over tungsten-containing material compared to conventional nonelectrochemical leaching.

20 FIG. 51C is a plot diagram of the removed cobalt to tungsten ratios of Examples 8 and 9 after the respective leaching processes. As shown, the electrochemical leaching technique associated with Example 8 resulted in a removed cobalt to tungsten ratio of nearly 8 (7.79) in the citric acid-cobalt chloride leaching solution. The conventional nonelectrochemical leaching technique associated with Example 9 resulted in a removed cobalt to tungsten ratio of nearly 3 (2.90) in the hydrofluoric acid-nitric acid leaching solution. The electrochemical leaching process of Example 8 exhibited a nearly threefold higher cobalt to tungsten ratio than the conventional nonelectrochemical leaching process of Example 8. The ratio of amount of removed cobalt to tungsten present in the respective leaching solutions demonstrated the preferential nature of electrochemical leaching to cobalt over tungsten-containing material compared to conventional nonelectrochemical leaching. Microscopy performed on one of the PCD tables of Example 8 using a scanning electron microscope indicated that there was a 30 compositional gradient in the electrochemically leached region of the PCD table.

35 The preceding description has been provided to enable others skilled in the art to best utilize various aspects of the embodiments described herein. This description is not 40 intended to be exhaustive or to be limited to any precise form disclosed. Many modifications and variations are possible without departing from the spirit and scope of the instant disclosure. It is desired that the embodiments described herein be considered in all respects illustrative and 45 not restrictive and that reference be made to the appended claims and their equivalents for determining the scope of the instant disclosure.

50 Unless otherwise noted, the terms “a” or “an,” as used in the specification and claims, are to be construed as meaning “at least one of.” In addition, for ease of use, the words “including” and “having,” as used in the specification and claims, are interchangeable with and have the same meaning as the word “comprising.”

60 The invention claimed is:

1. A method of making a polycrystalline diamond element, the method comprising:  
55 exposing an electrode and at least a portion of a polycrystalline diamond material to a processing solution, wherein the polycrystalline diamond material includes a plurality of diamond grains defining a plurality of interstitial regions, at least a portion of the plurality of

interstitial regions including a metallic material and at least one tungsten-containing material disposed therein; while the electrode and the at least the portion of the polycrystalline diamond material are exposed to the processing solution, applying an electrical potential between the electrode and the polycrystalline diamond material to cause an electrochemical leaching process; selecting at least one of the processing solution or a characteristic of the electrochemical leaching process to provide a preferential leaching of at least a portion of the metallic material from the polycrystalline diamond material over the at least one tungsten-containing material; and

removing relatively more of a content of the metallic material from the plurality of interstitial regions of the polycrystalline diamond material than a content of the at least one tungsten-containing material during the preferential leaching of the electrochemical leaching process to form a leached volume, wherein the metallic material is present in the leached volume in a first concentration of greater than 0 to about 1.5 weight % and the at least one tungsten-containing material is present in the leached volume in a second concentration of greater than 0 to about 4 weight %.

2. The method of claim 1, wherein the method includes: prior to exposing the electrode and the at least the portion of the polycrystalline diamond material to the processing solution, exposing the at least the portion of the polycrystalline diamond material to an additional processing solution that at least partially non-electrochemically leaches at least a portion of the metallic material from the polycrystalline diamond material; and

wherein applying an electrical potential between the electrode and the polycrystalline diamond material to cause preferential leaching of at least a portion of the metallic material from the polycrystalline diamond material over the at least one tungsten-containing material includes applying the electrical potential between the electrode and the polycrystalline diamond material to cause preferential leaching after exposing the at least the portion of the polycrystalline diamond material to the additional processing solution.

3. The method of claim 1, wherein the processing solution includes at least one of acetic acid, ammonium chloride, arsenic acid, ascorbic acid, carboxylic acid, citric acid, formic acid, hydrobromic acid, hydrofluoric acid, hydroiodic acid, lactic acid, malic acid, nitric acid, oxalic acid, phosphoric acid, propionic acid, pyruvic acid, succinic acid, or tartaric acid.

4. The method of claim 1, wherein the processing solution includes at least one of an ion or a salt, and an ester of at least one of acetic acid, ammonium chloride, arsenic acid, ascorbic acid, carboxylic acid, citric acid, formic acid, hydrobromic acid, hydrofluoric acid, hydroiodic acid, lactic acid, malic acid, nitric acid, oxalic acid, phosphoric acid, propionic acid, pyruvic acid, succinic acid, or tartaric acid.

5. The method of claim 1, wherein the metallic material includes at least one Group VIII metal.

6. The method of claim 5, wherein the at least one Group VIII metal includes at least one of cobalt, iron, or nickel.

7. The method of claim 1, wherein the at least one tungsten-containing material includes one or more of tungsten, tungsten carbide, or cobalt tungsten carbide.

8. The method of claim 1, wherein the at least one tungsten-containing material includes one or more of chro-

mium, niobium, tantalum, titanium, tungsten, vanadium, or a carbide of any of the foregoing.

9. The method of claim 1, wherein the at least one tungsten-containing material includes a cementing constituent having one or more of cobalt, iron, nickel, alloys of any of the foregoing, or combinations of any of the foregoing.

10. The method of claim 1, wherein the first concentration of the metallic material is about 0 weight % to about 1.2 weight %.

11. The method of claim 1, wherein the first concentration of the metallic material is about 0 weight % to about 1 weight %.

12. The method of claim 1, wherein the first concentration of the metallic material is about 0.8 weight % to about 1 weight %.

13. The method of claim 1, wherein the second concentration of the at least one tungsten-containing material is about 0.5 weight % to about 3 weight %.

14. The method of claim 1, wherein the second concentration of the at least one tungsten-containing material is about 0.5 weight % to about 1.5 weight %.

15. The method of claim 1, wherein the second concentration of the at least one tungsten-containing material is about 0.5 weight % to about 1 weight %.

16. The method of claim 1, wherein, after exposing the electrode and at least the portion of the polycrystalline diamond material to the processing solution, the polycrystalline diamond material includes an additional leached volume, the leached volume disposed between the additional leached volume and an unleached volume, wherein the additional leached volume has less of the at least one tungsten-containing material than the leached volume.

17. The method of claim 16, wherein the additional leached volume is substantially free of the at least one tungsten-containing material.

18. The method of claim 16, wherein the concentration of the at least one tungsten-containing material is about the same in the leached volume and the unleached volume.

19. A method of making a polycrystalline diamond element, the method comprising:

exposing an electrode and at least a cutting face portion of a polycrystalline diamond material to a processing solution, wherein the at least the cutting face portion of the polycrystalline diamond material includes a plurality of diamond grains defining a plurality of interstitial regions, at least a portion of the plurality of interstitial regions including a metallic material and at least one tungsten-containing material;

while the electrode and the at least the cutting face portion of the polycrystalline diamond material are exposed to the processing solution in an electrochemical leaching process, applying an electrical potential between the electrode and the polycrystalline diamond material; and removing relatively more of the metallic material from the plurality of interstitial regions of the at least the cutting face portion of the polycrystalline diamond material than the at least one tungsten-containing material during the electrochemical leaching process to form a leached volume.

20. The method of claim 19, further comprising preferentially removing the metallic material while substantially not causing removal of the at least one tungsten-containing material.

21. The method of claim 20, wherein the metallic material is present in the leached volume in the first concentration of greater than 0 to about 1.5 weight %.

**22.** A method of making a polycrystalline diamond element, the method comprising:

exposing an electrode and at least a cutting face portion of a polycrystalline diamond material to a processing solution, wherein the at least the cutting face portion of the polycrystalline diamond material includes a plurality of diamond grains defining a plurality of interstitial regions, at least a portion of the plurality of interstitial regions including a metallic material and at least one tungsten-containing material disposed therein; 5  
while the electrode and the at least the cutting face portion of the polycrystalline diamond material are exposed to the processing solution, applying an electrical potential between the electrode and the polycrystalline diamond material; 10  
removing relatively more of the metallic material from the plurality of interstitial regions of the polycrystalline diamond material than the at least one tungsten-containing material to form a leached volume; and 15  
preferentially removing the metallic material while substantially not causing removal of the at least one tungsten-containing material.

**23.** The method of claim 19, wherein the metallic material is present in the leached volume in a first concentration of greater than 0 to about 1.5 weight % and the at least one tungsten-containing material is present in the leached volume in a second concentration of greater than 0 to about 4 weight %. 25

\* \* \* \* \*